



US011136513B2

(12) **United States Patent**  
Moore et al.

(10) **Patent No.:** US 11,136,513 B2  
(45) **Date of Patent:** \*Oct. 5, 2021

(54) **MULTI-STAGE DEVICE AND PROCESS FOR PRODUCTION OF A LOW SULFUR HEAVY MARINE FUEL OIL FROM DISTRESSED HEAVY FUEL OIL MATERIALS**

(71) Applicant: **Magämä Technology LLC**, Houston, TX (US)

(72) Inventors: **Michael Joseph Moore**, Houston, TX (US); **Bertrand Ray Klussmann**, Houston, TX (US); **Carter James White**, Houston, TX (US)

(73) Assignee: **Magämä Technology LLC**, Houston, TX (US)

(\*) Notice: Subject to any disclaimer, the term of this patent is extended or adjusted under 35 U.S.C. 154(b) by 0 days.

This patent is subject to a terminal disclaimer.

(21) Appl. No.: **16/719,461**

(22) Filed: **Dec. 18, 2019**

(65) **Prior Publication Data**

US 2020/0123458 A1 Apr. 23, 2020

**Related U.S. Application Data**

(63) Continuation of application No. 16/124,884, filed on Sep. 7, 2018, now Pat. No. 10,604,709, which is a (Continued)

(51) **Int. Cl.**

*C10G 69/04* (2006.01)  
*C10G 69/00* (2006.01)  
*C10G 69/02* (2006.01)

(52) **U.S. Cl.**

CPC ..... *C10G 69/04* (2013.01); *C10G 2300/202* (2013.01); *C10G 2300/205* (2013.01); *C10G 2300/302* (2013.01)

(58) **Field of Classification Search**

None

See application file for complete search history.

(56) **References Cited**

U.S. PATENT DOCUMENTS

3,163,593 A 12/1964 Webster et al.  
3,227,645 A 1/1966 Frumkin et al.

(Continued)

FOREIGN PATENT DOCUMENTS

CA 1054130 5/1979  
CA 1060370 8/1979

(Continued)

OTHER PUBLICATIONS

U.S. Appl. No. 16/103,884, Non-Final Office Action dated Mar. 29, 2021.

(Continued)

*Primary Examiner* — Tam M Nguyen

(74) *Attorney, Agent, or Firm* — Carter J. White

(57) **ABSTRACT**

A multi-stage process for reducing the production of a Product Heavy Marine Fuel Oil from Distressed Fuel Oil Materials (DFOM) involving a pre-treatment process that transforms the DFOM into Feedstock HMFO which is subsequently sent to a Core Process for removing the Environmental Contaminates. The Product Heavy Marine Fuel Oil complies with ISO 8217 for residual marine fuel oils and has a sulfur level has a maximum sulfur content (ISO 14596 or ISO 8754) between the range of 0.05 mass % to 1.0 mass. A process plant for conducting the process is also disclosed.

**19 Claims, 13 Drawing Sheets**



**Related U.S. Application Data**

continuation-in-part of application No. PCT/US2018/017863, filed on Feb. 12, 2018, and a continuation-in-part of application No. PCT/US2018/017855, filed on Feb. 12, 2018.

- (60) Provisional application No. 62/589,479, filed on Nov. 21, 2017, provisional application No. 62/458,002, filed on Feb. 12, 2017.

**(56) References Cited****U.S. PATENT DOCUMENTS**

|              |         |                        |              |         |                        |
|--------------|---------|------------------------|--------------|---------|------------------------|
| 3,234,121 A  | 2/1966  | Maclarens              | 6,203,695 B1 | 3/2001  | Harle et al.           |
| 3,287,254 A  | 11/1966 | Paterson               | 6,207,041 B1 | 3/2001  | Morel et al.           |
| 3,306,845 A  | 2/1967  | Poll                   | 6,217,749 B1 | 4/2001  | Espeillac et al.       |
| 3,531,398 A  | 9/1970  | Adams                  | 6,251,262 B1 | 6/2001  | Hatanaka et al.        |
| 3,544,452 A  | 12/1970 | Jaffe                  | 6,251,263 B1 | 6/2001  | Hatanaka et al.        |
| 3,562,800 A  | 2/1971  | Carlson et al.         | 6,265,629 B1 | 7/2001  | Fava et al.            |
| 3,577,353 A  | 5/1971  | White                  | 6,299,759 B1 | 10/2001 | Bradway et al.         |
| 3,658,681 A  | 4/1972  | Wilson et al.          | 6,303,531 B1 | 10/2001 | Lussier et al.         |
| 3,668,116 A  | 6/1972  | Adams et al.           | 6,306,287 B1 | 10/2001 | Billon et al.          |
| 3,684,688 A  | 8/1972  | Roselius               | 6,306,289 B1 | 10/2001 | Hayashi et al.         |
| 3,749,664 A  | 7/1973  | Mickleson              | 6,328,880 B1 | 12/2001 | Yoshita et al.         |
| 3,814,683 A  | 6/1974  | Christman et al.       | 6,344,136 B1 | 2/2002  | Butler et al.          |
| 3,859,199 A  | 1/1975  | Gatsis                 | 6,383,975 B1 | 5/2002  | Rocha et al.           |
| 3,880,598 A  | 4/1975  | Van Der Toorn          | 6,402,940 B1 | 6/2002  | Rappas                 |
| 3,893,909 A  | 7/1975  | Selvidge               | 6,406,615 B1 | 6/2002  | Iwamoto et al.         |
| 3,902,991 A  | 9/1975  | Christensen et al.     | 6,540,904 B1 | 4/2003  | Gun et al.             |
| 4,006,076 A  | 2/1977  | Christensen et al.     | 6,554,994 B1 | 4/2003  | Reynolds et al.        |
| 4,017,382 A  | 4/1977  | Bonnell et al.         | 6,566,296 B2 | 5/2003  | Plantenga et al.       |
| 4,054,508 A  | 10/1977 | Milstein et al.        | 6,576,584 B1 | 6/2003  | Iijima et al.          |
| 4,138,227 A  | 2/1979  | Wilson et al.          | 6,620,313 B1 | 7/2003  | Ginestra et al.        |
| 4,267,033 A  | 5/1981  | Heck et al.            | 6,649,042 B2 | 9/2003  | Soled et al.           |
| 4,306,964 A  | 12/1981 | Angevine               | 6,656,348 B2 | 11/2003 | Dassori et al.         |
| 4,357,263 A  | 11/1982 | Heck et al.            | 6,656,349 B1 | 12/2003 | Fujita et al.          |
| 4,404,097 A  | 9/1983  | Angevine et al.        | 6,673,230 B2 | 1/2004  | Hagen                  |
| 4,420,388 A  | 12/1983 | Bertolacini et al.     | 6,712,955 B1 | 3/2004  | Soled et al.           |
| 4,460,707 A  | 7/1984  | Simpson                | 6,733,659 B1 | 5/2004  | Kure et al.            |
| 4,548,710 A  | 10/1985 | Simpson                | 6,783,661 B1 | 8/2004  | Briot et al.           |
| 4,604,185 A  | 8/1986  | McConaghay, Jr. et al. | 6,797,153 B1 | 9/2004  | Fukuyama et al.        |
| 4,645,584 A  | 2/1987  | Didchenko et al.       | 6,858,132 B2 | 2/2005  | Kumagai et al.         |
| 4,925,554 A  | 5/1990  | Sato et al.            | 6,860,987 B2 | 3/2005  | Plantenga et al.       |
| 5,167,796 A  | 12/1992 | Didchenko et al.       | 6,863,803 B1 | 3/2005  | Riley et al.           |
| 5,306,419 A  | 4/1994  | Harrison et al.        | 6,929,738 B1 | 8/2005  | Riley et al.           |
| 5,342,507 A  | 8/1994  | Dai et al.             | 6,984,310 B2 | 1/2006  | Ginstra et al.         |
| 5,374,350 A  | 12/1994 | Heck et al.            | 7,001,503 B1 | 2/2006  | Hiroki et al.          |
| 5,389,595 A  | 2/1995  | Simpson et al.         | 7,108,779 B1 | 9/2006  | Thakkar                |
| 5,391,304 A  | 2/1995  | Lantos                 | 7,119,045 B2 | 10/2006 | Magna et al.           |
| 5,401,392 A  | 3/1995  | Courty et al.          | 7,166,209 B2 | 1/2007  | Dassori                |
| 5,417,846 A  | 5/1995  | Renard                 | 7,169,294 B2 | 1/2007  | Abe et al.             |
| 5,543,036 A  | 8/1996  | Chang et al.           | 7,232,515 B1 | 6/2007  | Demmin et al.          |
| 5,591,325 A  | 1/1997  | Higashi                | 7,244,350 B2 | 7/2007  | Martin et al.          |
| 5,622,616 A  | 4/1997  | Porter et al.          | 7,265,075 B2 | 9/2007  | Tsukada et al.         |
| 5,686,375 A  | 11/1997 | Iyer et al.            | 7,288,182 B1 | 10/2007 | Soled et al.           |
| 5,759,385 A  | 6/1998  | Aussillous et al.      | 7,384,537 B2 | 6/2008  | Nagamatsu et al.       |
| 5,779,992 A  | 7/1998  | Higashi                | 7,402,547 B2 | 7/2008  | Wellington et al.      |
| 5,837,130 A  | 11/1998 | Crossland              | 7,413,646 B2 | 8/2008  | Wellington et al.      |
| 5,868,923 A  | 2/1999  | Porter et al.          | 7,416,653 B2 | 8/2008  | Wellington             |
| 5,882,364 A  | 3/1999  | Dilworth               | 7,449,102 B2 | 11/2008 | Kalnes                 |
| 5,888,379 A  | 3/1999  | Ushio et al.           | 7,491,313 B2 | 2/2009  | Toshima et al.         |
| 5,897,768 A  | 4/1999  | McVicker et al.        | 7,507,325 B2 | 3/2009  | Gueret et al.          |
| 5,917,101 A  | 6/1999  | Munoz                  | 7,513,989 B1 | 4/2009  | Soled et al.           |
| 5,922,189 A  | 7/1999  | Santos                 | 7,517,446 B2 | 4/2009  | Lott                   |
| 5,928,501 A  | 7/1999  | Sudhakar et al.        | 7,534,342 B2 | 5/2009  | Bhan et al.            |
| 5,948,239 A  | 9/1999  | Virdi et al.           | 7,585,406 B2 | 9/2009  | Khadzhiev et al.       |
| 5,958,816 A  | 9/1999  | Neuman et al.          | 7,588,681 B2 | 9/2009  | Bhan et al.            |
| 5,961,709 A  | 10/1999 | Hayner et al.          | 7,651,604 B2 | 1/2010  | Ancheyta Juarez et al. |
| 5,976,361 A  | 11/1999 | Hood et al.            | 7,651,605 B2 | 1/2010  | Wataru et al.          |
| 5,997,723 A  | 12/1999 | Wiehe et al.           | 7,695,610 B2 | 4/2010  | Bolshakov et al.       |
| 6,017,443 A  | 1/2000  | Buchanan               | 7,713,905 B2 | 5/2010  | Dufresne et al.        |
| 6,117,306 A  | 9/2000  | Morel et al.           | 7,718,050 B2 | 5/2010  | Gueret et al.          |
| 6,160,193 A  | 12/2000 | Gore                   | 7,754,162 B2 | 7/2010  | Dassori                |
| 6,162,350 A  | 12/2000 | Soled et al.           | 7,901,569 B2 | 3/2011  | Farshid et al.         |
| 6,171,477 B1 | 1/2001  | Morel et al.           | 7,938,955 B2 | 5/2011  | Araki et al.           |
| 6,193,766 B1 | 2/2001  | Jordan                 | 7,943,035 B2 | 5/2011  | Chornet et al.         |
|              |         |                        | 8,012,343 B2 | 9/2011  | Plantenga et al.       |
|              |         |                        | 8,021,538 B2 | 9/2011  | Klein                  |
|              |         |                        | 8,114,806 B2 | 2/2012  | Bhan et al.            |
|              |         |                        | 8,163,166 B2 | 4/2012  | Wellington et al.      |
|              |         |                        | 8,173,570 B2 | 5/2012  | Maesen et al.          |
|              |         |                        | 8,241,489 B2 | 8/2012  | Bhan et al.            |
|              |         |                        | 8,268,164 B2 | 9/2012  | Wellington et al.      |
|              |         |                        | 8,318,000 B2 | 11/2012 | Bhan et al.            |
|              |         |                        | 8,318,628 B2 | 11/2012 | Brun et al.            |
|              |         |                        | 8,343,887 B2 | 1/2013  | Maesen et al.          |
|              |         |                        | 8,371,741 B2 | 2/2013  | Hassan                 |
|              |         |                        | 8,372,268 B2 | 2/2013  | Ginestra et al.        |
|              |         |                        | 8,394,254 B2 | 3/2013  | Wellington et al.      |
|              |         |                        | 8,394,262 B2 | 3/2013  | Guichard et al.        |
|              |         |                        | 8,475,651 B2 | 7/2013  | Nemec et al.           |

(56)

## References Cited

## U.S. PATENT DOCUMENTS

|               |         |                        |                 |         |                       |
|---------------|---------|------------------------|-----------------|---------|-----------------------|
| 8,506,794 B2  | 8/2013  | Bhan et al.            | 10,876,053 B2   | 6/2020  | Klussmann et al.      |
| 8,546,626 B2  | 10/2013 | Daudin et al.          | 10,899,983 B1   | 1/2021  | Kar et al.            |
| 8,563,456 B2  | 10/2013 | Dillon et al.          | 10,954,456 B2   | 3/2021  | Moore et al.          |
| 8,608,938 B2  | 12/2013 | Wellington et al.      | 10,995,290 B2   | 5/2021  | Anderson et al.       |
| 8,608,946 B2  | 12/2013 | Bhan et al.            | 2001/0001036 A1 | 5/2001  | Espeillac et al.      |
| 8,613,851 B2  | 12/2013 | Wellington et al.      | 2001/0013484 A1 | 8/2001  | Zeuthen et al.        |
| 8,652,817 B2  | 2/2014  | Wood et al.            | 2002/0037806 A1 | 3/2002  | Dufresne et al.       |
| 8,663,453 B2  | 3/2014  | Wellington et al.      | 2002/0045540 A1 | 4/2002  | Bartholdy             |
| 8,679,319 B2  | 3/2014  | Milam et al.           | 2002/0056664 A1 | 5/2002  | Chabot                |
| 8,679,322 B2  | 3/2014  | Marzin et al.          | 2002/0070147 A1 | 6/2002  | Sonnemans et al.      |
| 8,702,970 B2  | 4/2014  | Maesen et al.          | 2002/0117426 A1 | 8/2002  | Holder                |
| 8,716,164 B2  | 5/2014  | Dillon et al.          | 2002/0144932 A1 | 10/2002 | Gong et al.           |
| 8,721,871 B1  | 5/2014  | Dindi et al.           | 2002/0148757 A1 | 10/2002 | Huff et al.           |
| 8,722,558 B2  | 5/2014  | Konno et al.           | 2002/0157990 A1 | 10/2002 | Feimer et al.         |
| 8,722,563 B2  | 5/2014  | Soled et al.           | 2002/0195375 A1 | 12/2002 | Chapus et al.         |
| 8,722,564 B2  | 5/2014  | Soled et al.           | 2003/0042172 A1 | 3/2003  | Sharivker et al.      |
| 8,741,129 B2  | 6/2014  | Brown et al.           | 2003/0125198 A1 | 7/2003  | Ginestra et al.       |
| 8,747,659 B2  | 6/2014  | Kiss et al.            | 2003/0131526 A1 | 7/2003  | Kresnyak et al.       |
| 8,764,972 B2  | 7/2014  | Bhan et al.            | 2003/0146133 A1 | 8/2003  | Nagamatsu et al.      |
| 8,784,646 B2  | 7/2014  | Sanchez et al.         | 2003/0217951 A1 | 11/2003 | Marchal-George et al. |
| 8,795,514 B2  | 8/2014  | Kimura et al.          | 2004/0007501 A1 | 1/2004  | Sughrue et al.        |
| 8,821,714 B2  | 9/2014  | Chaumonnot et al.      | 2004/0020829 A1 | 2/2004  | Magna et al.          |
| 8,877,040 B2  | 11/2014 | Hoehn et al.           | 2004/0040890 A1 | 3/2004  | Morton et al.         |
| 8,894,838 B2  | 11/2014 | Dindi et al.           | 2004/0055934 A1 | 3/2004  | Tromeur et al.        |
| 8,926,826 B2  | 1/2015  | Dindi et al.           | 2004/0134837 A1 | 7/2004  | Dassori               |
| 8,946,110 B2  | 2/2015  | Toledo Antonio et al.  | 2004/0178117 A1 | 9/2004  | Morton et al.         |
| 8,962,514 B2  | 2/2015  | Seki et al.            | 2004/0186014 A1 | 9/2004  | Tsukada et al.        |
| 8,987,537 B1  | 3/2015  | Droubi et al.          | 2004/0209771 A1 | 10/2004 | Abe et al.            |
| 8,999,011 B2  | 4/2015  | Stern                  | 2004/0232041 A1 | 11/2004 | Kiser et al.          |
| 9,057,035 B1  | 6/2015  | Kraus et al.           | 2004/0256293 A1 | 12/2004 | Abe et al.            |
| 9,102,884 B2  | 8/2015  | Xu et al.              | 2005/0020446 A1 | 1/2005  | Choudhary et al.      |
| 9,109,176 B2  | 8/2015  | Stern et al.           | 2005/0101480 A1 | 5/2005  | Ackerman et al.       |
| 9,127,215 B2  | 9/2015  | Choi et al.            | 2005/0109674 A1 | 5/2005  | Klein                 |
| 9,127,218 B2  | 9/2015  | Banerjee et al.        | 2005/0113250 A1 | 5/2005  | Schleicher et al.     |
| 9,139,782 B2  | 9/2015  | Dindi et al.           | 2005/0133405 A1 | 6/2005  | Wellington et al.     |
| 9,206,363 B2  | 12/2015 | Woo et al.             | 2005/0133406 A1 | 6/2005  | Wellington et al.     |
| 9,212,323 B2  | 12/2015 | Dindi et al.           | 2005/0133411 A1 | 6/2005  | Zeuthen et al.        |
| 9,216,407 B2  | 12/2015 | Duma et al.            | 2005/0133416 A1 | 6/2005  | Bhan et al.           |
| 9,260,671 B2  | 2/2016  | Shafi et al.           | 2005/0133417 A1 | 6/2005  | Bhan et al.           |
| 9,278,339 B2  | 3/2016  | Bellussi et al.        | 2005/0135997 A1 | 6/2005  | Wellington et al.     |
| 9,340,733 B2  | 5/2016  | Marchand et al.        | 2005/0139512 A1 | 6/2005  | Wellington et al.     |
| 9,359,561 B2  | 6/2016  | Bazer-Bachi et al.     | 2005/0139520 A1 | 6/2005  | Bhan et al.           |
| 9,365,781 B2  | 6/2016  | Dindi                  | 2005/0139522 A1 | 6/2005  | Bhan et al.           |
| 9,365,782 B2  | 6/2016  | Dindi                  | 2005/0145537 A1 | 7/2005  | Wellington et al.     |
| 9,387,466 B2  | 7/2016  | Rana et al.            | 2005/0145538 A1 | 7/2005  | Wellington et al.     |
| 9,434,893 B2  | 9/2016  | Dufresne               | 2005/0145543 A1 | 7/2005  | Bhan et al.           |
| 9,458,396 B2  | 10/2016 | Weiss et al.           | 2005/0148487 A1 | 7/2005  | Brownscombe et al.    |
| 9,487,718 B2  | 11/2016 | Kraus et al.           | 2005/0150156 A1 | 7/2005  | Karas et al.          |
| 9,499,758 B2  | 11/2016 | Droubi et al.          | 2005/0150818 A1 | 7/2005  | Bhan et al.           |
| 9,512,319 B2  | 12/2016 | Chatron-Michuad et al. | 2005/0155906 A1 | 7/2005  | Wellington et al.     |
| 9,540,573 B2  | 1/2017  | Bhan                   | 2005/0167321 A1 | 8/2005  | Wellington et al.     |
| 9,546,327 B2  | 1/2017  | Krasu et al.           | 2005/0167327 A1 | 8/2005  | Bhan et al.           |
| 9,605,215 B2  | 3/2017  | Lott et al.            | 2005/0167328 A1 | 8/2005  | Bhan et al.           |
| 9,624,448 B2  | 4/2017  | Joo et al.             | 2005/0167329 A1 | 8/2005  | Bhan et al.           |
| 9,650,312 B2  | 5/2017  | Baldassari et al.      | 2005/0167330 A1 | 8/2005  | Bhan et al.           |
| 9,650,580 B2  | 5/2017  | Merdignac              | 2005/0167331 A1 | 8/2005  | Bhan et al.           |
| 9,657,236 B2  | 5/2017  | Yang et al.            | 2005/0269245 A1 | 12/2005 | Huve                  |
| 9,675,968 B2  | 6/2017  | Alonso Nunez et al.    | 2006/0052235 A1 | 3/2006  | Bai et al.            |
| 9,737,883 B2  | 8/2017  | Yamane et al.          | 2006/0060501 A1 | 3/2006  | Thierry et al.        |
| 9,803,152 B2  | 10/2017 | Kar                    | 2006/0060509 A1 | 3/2006  | Yoshimitsu et al.     |
| 9,896,630 B2  | 2/2018  | Weiss et al.           | 2006/0060510 A1 | 3/2006  | Bhan                  |
| 9,908,105 B2  | 3/2018  | Duma et al.            | 2006/0102522 A1 | 5/2006  | Turaga et al.         |
| 9,908,107 B2  | 3/2018  | Osaki et al.           | 2006/0115392 A1 | 6/2006  | Dassori               |
| 9,919,293 B1  | 3/2018  | Rana et al.            | 2006/0175229 A1 | 8/2006  | Montanari et al.      |
| 9,920,270 B2  | 3/2018  | Robinson               | 2006/0211900 A1 | 9/2006  | Iki et al.            |
| 10,138,438 B2 | 11/2018 | Houten                 | 2006/0231456 A1 | 10/2006 | Bhan                  |
| 10,144,882 B2 | 12/2018 | Dindi et al.           | 2006/0231465 A1 | 10/2006 | Bhan                  |
| 10,150,930 B2 | 12/2018 | Houten                 | 2006/0234876 A1 | 10/2006 | Bhan                  |
| 10,308,884 B2 | 6/2019  | Klussmann et al.       | 2006/0234877 A1 | 10/2006 | Bhan                  |
| 10,443,006 B1 | 10/2019 | Fruchey et al.         | 2006/0249429 A1 | 11/2006 | Iki et al.            |
| 10,533,141 B2 | 1/2020  | Moore et al.           | 2006/0281638 A1 | 12/2006 | Zaid et al.           |
| 10,563,133 B2 | 2/2020  | Moore et al.           | 2006/0289340 A1 | 12/2006 | Brownscombe et al.    |
| 10,584,287 B2 | 3/2020  | Klussmann et al.       | 2007/0000808 A1 | 1/2007  | Bhan et al.           |
| 10,597,594 B1 | 3/2020  | Fruchey et al.         | 2007/0000810 A1 | 1/2007  | Bhan et al.           |
| 10,604,709 B2 | 3/2020  | Moore et al.           | 2007/0105714 A1 | 5/2007  | Turaga et al.         |
|               |         |                        | 2007/0108098 A1 | 5/2007  | Flint et al.          |
|               |         |                        | 2007/0131584 A1 | 6/2007  | Kaines                |

| (56)                  | References Cited |                      |                  |         |                    |            |        |
|-----------------------|------------------|----------------------|------------------|---------|--------------------|------------|--------|
| U.S. PATENT DOCUMENTS |                  |                      |                  |         |                    |            |        |
| 2007/0138055 A1       | 6/2007           | Farshid et al.       | 2012/0181219 A1  | 7/2012  | Seki et al.        |            |        |
| 2007/0170096 A1       | 7/2007           | Shan et al.          | 2013/0037447 A1  | 2/2013  | Zimmerman          |            |        |
| 2007/0175797 A1       | 8/2007           | Iki et al.           | 2013/0081977 A1  | 4/2013  | Woo et al.         |            |        |
| 2007/0284285 A1       | 12/2007          | Stepanik et al.      | 2013/0105357 A1  | 5/2013  | Bhan               |            |        |
| 2008/0017551 A1       | 1/2008           | Kiryama et al.       | 2013/0105364 A1  | 5/2013  | Bhan               |            |        |
| 2008/0047875 A1       | 2/2008           | Karas et al.         | 2013/0126393 A1  | 5/2013  | Ginestra et al.    |            |        |
| 2008/0073247 A1       | 3/2008           | Bolshakov et al.     | 2013/0171039 A1  | 7/2013  | Graham et al.      |            |        |
| 2008/0085225 A1       | 4/2008           | Bhan et al.          | 2013/0186806 A1  | 7/2013  | Diehl et al.       |            |        |
| 2008/0135453 A1       | 6/2008           | Bhan                 | 2013/0225400 A1  | 8/2013  | Liang et al.       |            |        |
| 2008/0149531 A1       | 6/2008           | Roy-Auberger et al.  | 2013/0256190 A1  | 10/2013 | Wees et al.        |            |        |
| 2008/0167180 A1       | 7/2008           | Van Den Brink et al. | 2013/0267409 A1  | 10/2013 | Lee et al.         |            |        |
| 2008/0210595 A1       | 9/2008           | Bolshakov et al.     | 2013/0277273 A1  | 10/2013 | Mazyar             |            |        |
| 2008/0223755 A1       | 9/2008           | Roy-Auberger et al.  | 2013/0288885 A1  | 10/2013 | Domokos et al.     |            |        |
| 2008/0230440 A1       | 9/2008           | Graham et al.        | 2013/0306517 A1  | 11/2013 | Kester et al.      |            |        |
| 2008/0245700 A1       | 10/2008          | Wellington et al.    | 2013/0319910 A1  | 12/2013 | Koseoglu           |            |        |
| 2008/0245702 A1       | 10/2008          | Wellington et al.    | 2014/0001089 A1  | 1/2014  | Bazer-Bachi        |            |        |
| 2008/0262115 A1       | 10/2008          | Calis et al.         | 2014/0027351 A1  | 1/2014  | Bazer-Bachi et al. |            |        |
| 2008/0272027 A1       | 11/2008          | Wellington et al.    | 2014/0061094 A1  | 3/2014  | Ku et al.          |            |        |
| 2008/0272028 A1       | 11/2008          | Wellington et al.    | 2014/0073821 A1  | 3/2014  | Mitsui et al.      |            |        |
| 2008/0308459 A1       | 12/2008          | Hideshi et al.       | 2014/0076783 A1  | 3/2014  | Bhan               |            |        |
| 2009/0048097 A1       | 2/2009           | Jones et al.         | 2014/0097125 A1  | 4/2014  | Bazer-Bachi et al. |            |        |
| 2009/0057194 A1       | 3/2009           | Farshid et al.       | 2014/0166540 A1  | 6/2014  | Guichard et al.    |            |        |
| 2009/0057197 A1       | 3/2009           | Bhan et al.          | 2014/0174980 A1  | 6/2014  | Brown et al.       |            |        |
| 2009/0062590 A1       | 3/2009           | Nadler et al.        | 2014/0174983 A1  | 6/2014  | Klein et al.       |            |        |
| 2009/0114569 A1       | 5/2009           | Osaheni et al.       | 2014/0183098 A1  | 7/2014  | Cooper et al.      |            |        |
| 2009/0134064 A1       | 5/2009           | Reynolds             | 2014/0183099 A1  | 7/2014  | Ginestra et al.    |            |        |
| 2009/0139902 A1       | 6/2009           | Kressmann et al.     | 2014/0291203 A1  | 10/2014 | Molinari et al.    |            |        |
| 2009/0166260 A1       | 7/2009           | Magalie et al.       | 2014/0299515 A1  | 10/2014 | Weiss et al.       |            |        |
| 2009/0178951 A1       | 7/2009           | Balthasar et al.     | 2014/0305843 A1  | 10/2014 | Kraus et al.       |            |        |
| 2009/0230022 A1       | 9/2009           | Gorbaty et al.       | 2014/0315712 A1  | 10/2014 | Smegal             |            |        |
| 2009/0234166 A1       | 9/2009           | Gorbaty et al.       | 2014/0323779 A1  | 10/2014 | Alphazan et al.    |            |        |
| 2009/0255850 A1       | 10/2009          | Bhan et al.          | 2014/0326642 A1  | 11/2014 | Tanaka et al.      |            |        |
| 2009/0255851 A1       | 10/2009          | Bhan et al.          | 2014/0332444 A1  | 11/2014 | Weiss et al.       |            |        |
| 2009/0275788 A1       | 11/2009          | Bedard et al.        | 2014/0353210 A1  | 12/2014 | Graham et al.      |            |        |
| 2009/0283444 A1       | 11/2009          | Bhan et al.          | 2015/0057205 A1  | 2/2015  | Morishima et al.   |            |        |
| 2009/0288987 A1       | 11/2009          | Bhan et al.          | 2015/0108039 A1  | 4/2015  | Bhan               |            |        |
| 2009/0308791 A1       | 12/2009          | Bhan et al.          | 2015/0111726 A1  | 4/2015  | Bhan et al.        |            |        |
| 2009/0308812 A1       | 12/2009          | Osaheni et al.       | 2015/0144531 A1  | 5/2015  | Ginstra et al.     |            |        |
| 2009/0314686 A1       | 12/2009          | Zimmerman            | 2015/0144532 A1  | 5/2015  | He et al.          |            |        |
| 2010/0006475 A1       | 1/2010           | Ginestra             | 2015/0217261 A1  | 8/2015  | Norling            |            |        |
| 2010/0018902 A1       | 1/2010           | Brownscombe et al.   | 2015/0224476 A1  | 8/2015  | Plecha et al.      |            |        |
| 2010/0025291 A1       | 2/2010           | Shafi et al.         | 2015/0240174 A1  | 8/2015  | Kraus et al.       |            |        |
| 2010/0044274 A1       | 2/2010           | Brun et al.          | 2015/0315480 A1  | 11/2015 | Hanks et al.       |            |        |
| 2010/0055005 A1       | 3/2010           | Bhan et al.          | 2015/0321177 A1  | 11/2015 | Rana et al.        |            |        |
| 2010/0098602 A1       | 4/2010           | Bhan et al.          | 2015/0337225 A1  | 11/2015 | Droubi et al.      |            |        |
| 2010/0155301 A1       | 6/2010           | Guichard et al.      | 2015/0353848 A1  | 12/2015 | Patron             |            |        |
| 2010/0200463 A1       | 8/2010           | Patron et al.        | 2015/0353851 A1  | 12/2015 | Buchanan           |            |        |
| 2010/0213103 A1       | 8/2010           | Patron et al.        | 2016/0001272 A1  | 1/2016  | Daudin             |            |        |
| 2010/0243526 A1       | 9/2010           | Ginestra et al.      | 2016/0017240 A1  | 1/2016  | Duma et al.        |            |        |
| 2010/0243532 A1       | 9/2010           | Myers et al.         | 2016/0024396 A1  | 1/2016  | Zink et al.        |            |        |
| 2010/0264067 A1       | 10/2010          | Osaheni et al.       | 2016/0060549 A1  | 3/2016  | Juarez et al.      |            |        |
| 2010/0294698 A1       | 11/2010          | e Mello et al.       | 2016/0074840 A1  | 3/2016  | Duma et al.        |            |        |
| 2010/0326890 A1       | 12/2010          | Bhan                 | 2016/0075954 A1  | 3/2016  | Monson et al.      |            |        |
| 2011/0017637 A1       | 1/2011           | Reynolds et al.      | 2016/0122665 A1* | 5/2016  | Weiss .....        | C10G 65/12 | 208/57 |
| 2011/0079542 A1       | 4/2011           | Ellis et al.         |                  |         |                    |            |        |
| 2011/0083997 A1       | 4/2011           | Silva et al.         |                  |         |                    |            |        |
| 2011/0094938 A1       | 4/2011           | Morel                |                  |         |                    |            |        |
| 2011/0108461 A1       | 5/2011           | Gabrielov et al.     |                  |         |                    |            |        |
| 2011/0127194 A1       | 6/2011           | Zhang et al.         |                  |         |                    |            |        |
| 2011/0155558 A1       | 6/2011           | Cardoso et al.       |                  |         |                    |            |        |
| 2011/0155644 A1       | 6/2011           | Bhattacharyya et al. |                  |         |                    |            |        |
| 2011/0174681 A1       | 7/2011           | Milam et al.         |                  |         |                    |            |        |
| 2011/0178346 A1       | 7/2011           | Milam et al.         |                  |         |                    |            |        |
| 2011/0186477 A1       | 8/2011           | Milam et al.         |                  |         |                    |            |        |
| 2011/0186480 A1       | 8/2011           | Milam et al.         |                  |         |                    |            |        |
| 2011/0203971 A1       | 8/2011           | Kiss et al.          |                  |         |                    |            |        |
| 2011/0218097 A1       | 9/2011           | Rayo Mayoral et al.  |                  |         |                    |            |        |
| 2011/0240517 A1       | 10/2011          | Chornet et al.       |                  |         |                    |            |        |
| 2011/0277377 A1       | 11/2011          | Novak et al.         |                  |         |                    |            |        |
| 2012/0018352 A1       | 1/2012           | Seki et al.          |                  |         |                    |            |        |
| 2012/0103868 A1       | 5/2012           | Dindi et al.         |                  |         |                    |            |        |
| 2012/0116145 A1       | 5/2012           | Bhan et al.          |                  |         |                    |            |        |
| 2012/0145528 A1       | 6/2012           | Myers et al.         |                  |         |                    |            |        |
| 2012/0175285 A1       | 7/2012           | Bhan et al.          |                  |         |                    |            |        |
| 2012/0175286 A1       | 7/2012           | Bhan et al.          |                  |         |                    |            |        |

| (56)                     | References Cited |                        |    |               |         |  |
|--------------------------|------------------|------------------------|----|---------------|---------|--|
| U.S. PATENT DOCUMENTS    |                  |                        |    |               |         |  |
| 2017/0009163 A1          | 1/2017           | Kraus et al.           | EP | 1567262 A1    | 8/2005  |  |
| 2017/0022433 A1          | 1/2017           | Brown et al.           | EP | 1709141 A2    | 10/2006 |  |
| 2017/0029723 A1          | 2/2017           | Bazer-Bachi et al.     | EP | 1894625 A2    | 3/2008  |  |
| 2017/0044451 A1          | 2/2017           | Kar et al.             | EP | 2130895 A1    | 12/2009 |  |
| 2017/0058205 A1          | 3/2017           | Ho et al.              | EP | 2167616 A1    | 3/2010  |  |
| 2017/0058223 A1          | 3/2017           | Droubi et al.          | EP | 2510076 A2    | 10/2012 |  |
| 2017/0066979 A1          | 3/2017           | Lei et al.             | EP | 2907867 A1    | 8/2015  |  |
| 2017/0073592 A1          | 3/2017           | Nonaka et al.          | EP | 2947133 A1    | 11/2015 |  |
| 2017/0120224 A1          | 5/2017           | Boualleg et al.        | EP | 3041608 A1    | 7/2016  |  |
| 2017/0120228 A1          | 5/2017           | Boualleg et al.        | EP | 3074485 A0    | 10/2016 |  |
| 2017/0120229 A1          | 5/2017           | Boualleg et al.        | EP | 2990465 A1    | 3/2019  |  |
| 2017/0121612 A1          | 5/2017           | Boualleg et al.        | FR | 2681871       | 4/1993  |  |
| 2017/0128912 A1          | 5/2017           | Boualleg et al.        | FR | 3011004 A     | 3/2015  |  |
| 2017/0136446 A1          | 5/2017           | Carati et al.          | FR | 3011004 A1    | 3/2015  |  |
| 2017/0137725 A1          | 5/2017           | Boualleg et al.        | FR | 3013723 A     | 5/2015  |  |
| 2017/0165639 A1          | 6/2017           | Klein et al.           | FR | 3013723 A1    | 5/2015  |  |
| 2017/0175012 A1          | 6/2017           | Schleiffer et al.      | FR | 3053356       | 1/2018  |  |
| 2017/0183575 A1          | 6/2017           | Rubin-Pitel et al.     | GB | 1324167       | 7/1973  |  |
| 2017/0183582 A1          | 6/2017           | Hoehn et al.           | GB | 1502915       | 3/1978  |  |
| 2017/0192126 A1          | 7/2017           | Koseoglu               | GB | 1504586       | 3/1978  |  |
| 2017/0232414 A1          | 8/2017           | Hassan                 | GB | 1505886       | 3/1978  |  |
| 2017/0260463 A1          | 9/2017           | Schleiffer et al.      | GB | 2124252       | 2/1984  |  |
| 2017/0267937 A1          | 9/2017           | Schleiffer et al.      | JP | 2015059220 A  | 3/2015  |  |
| 2017/0306250 A1          | 10/2017          | Ginestra               | JP | 20200122450   | 8/2020  |  |
| 2017/0306252 A1          | 10/2017          | Malek Abbaslou et al.  | RU | 2700705       | 9/2019  |  |
| 2017/0335206 A1          | 11/2017          | Mukherjee et al.       | WO | 9113951 A1    | 9/1991  |  |
| 2017/0349846 A1          | 12/2017          | Ding et al.            | WO | 9820969       | 5/1998  |  |
| 2017/0355913 A1          | 12/2017          | Mountainland et al.    | WO | 9919061 A1    | 4/1999  |  |
| 2017/0355914 A1          | 12/2017          | Weiss et al.           | WO | 200145839 A1  | 6/2001  |  |
| 2017/0362514 A1          | 12/2017          | Hanks et al.           | WO | 9197971 A1    | 12/2001 |  |
| 2018/0016505 A1          | 1/2018           | Matsushita             | WO | 3209870 A2    | 2/2002  |  |
| 2018/0104676 A1          | 4/2018           | Yamane et al.          | WO | 02062926 A2   | 8/2002  |  |
| 2018/0134965 A1          | 5/2018           | Brown et al.           | WO | 2004052534 A1 | 6/2004  |  |
| 2018/0134972 A1          | 5/2018           | Brown et al.           | WO | 2004053028 A1 | 6/2004  |  |
| 2018/0134974 A1          | 5/2018           | Weiss et al.           | WO | 2005028596 A1 | 3/2005  |  |
| 2018/0147567 A1          | 5/2018           | Matsushita et al.      | WO | 2005063933 A2 | 7/2005  |  |
| 2018/0154340 A1          | 6/2018           | Boualleg et al.        | WO | 2009001314 A1 | 12/2008 |  |
| 2018/0230388 A1          | 8/2018           | Li et al.              | WO | 2011071705 A2 | 6/2011  |  |
| 2018/0251690 A1          | 9/2018           | Mountainland et al.    | WO | 2013083662    | 6/2013  |  |
| 2018/0291291 A1          | 10/2018          | Brown et al.           | WO | 2014096703 A  | 6/2014  |  |
| 2018/0371343 A1          | 12/2018          | Rubin-Patel et al.     | WO | 2014096703 A1 | 6/2014  |  |
| 2019/0002772 A1          | 1/2019           | Moore et al.           | WO | 2014096704 A  | 6/2014  |  |
| 2019/0010405 A1          | 1/2019           | Moore et al.           | WO | 2014160603 A1 | 10/2014 |  |
| 2019/0040329 A1*         | 2/2019           | Moore ..... C10G 69/04 | WO | 2014177424 A2 | 11/2014 |  |
| 2019/0078027 A1          | 3/2019           | Deimund et al.         | WO | 2015134521 A1 | 3/2015  |  |
| 2019/0093026 A1          | 3/2019           | Wohaibi et al.         | WO | 2015078674 A1 | 6/2015  |  |
| 2019/0136144 A1          | 5/2019           | Wohaibi et al.         | WO | 2015097199 A1 | 7/2015  |  |
| 2019/0185772 A1          | 6/2019           | Berkhous et al.        | WO | 2015122931 A1 | 8/2015  |  |
| 2019/0203130 A1          | 7/2019           | Mukherjee              | WO | 2015147222 A1 | 10/2015 |  |
| 2019/0233732 A1          | 8/2019           | Sun                    | WO | 2015147223 A1 | 10/2015 |  |
| 2019/0338203 A1          | 11/2019          | Umansky et al.         | WO | 2015178941 A1 | 11/2015 |  |
| 2019/0338205 A1          | 11/2019          | Ackerson et al.        | WO | 2015179017 A2 | 11/2015 |  |
| 2019/0382668 A1          | 12/2019          | Klussmann et al.       | WO | 2015189190 A1 | 12/2015 |  |
| 2020/0123458 A1          | 4/2020           | Moore et al.           | WO | 2016089590 A1 | 6/2016  |  |
| 2020/0199462 A1          | 6/2020           | Klussmann et al.       | WO | 2016146326 A1 | 9/2016  |  |
| 2020/0231886 A1          | 7/2020           | Kraus et al.           | WO | 2016195973 A1 | 12/2016 |  |
| 2020/0248080 A1          | 8/2020           | Peer et al.            | WO | 201780387 A1  | 5/2017  |  |
| 2020/0385644 A1          | 12/2020          | Rogel et al.           | WO | 2017168312 A1 | 10/2017 |  |
| 2021/0024842 A1          | 1/2021           | Fruchey et al.         | WO | 2017186484 A1 | 11/2017 |  |
| 2021/0062096 A1          | 3/2021           | Hodgkins et al.        | WO | 2018073018 A1 | 4/2018  |  |
| 2021/0102130 A1          | 4/2021           | Marques et al.         | WO | 2018075015 A1 | 4/2018  |  |
| 2021/0155858 A1          | 5/2021           | Koseoglu et al.        | WO | 2018075016 A1 | 4/2018  |  |
| FOREIGN PATENT DOCUMENTS |                  |                        |    |               |         |  |
| CA                       | 1248513          | 1/1989                 | WO | 2018075017    | 4/2018  |  |
| EP                       | 804288 A1        | 11/1997                | WO | 2018075017    | 4/2018  |  |
| EP                       | 870817 A1        | 10/1998                | WO | 2018075017 A1 | 4/2018  |  |
| EP                       | 876443 A1        | 11/1998                | WO | 2018093535 A1 | 5/2018  |  |
| EP                       | 952888 A1        | 11/1999                | WO | 2018101244 A1 | 6/2018  |  |
| EP                       | 1041133 A1       | 10/2000                | WO | 2018053323 A1 | 3/2019  |  |
| EP                       | 1052015 A1       | 11/2000                | WO | 2019104243 A1 | 5/2019  |  |
| EP                       | 1299192 A1       | 4/2003                 | WO | 2019125674 A1 | 6/2019  |  |
| EP                       | 1358302 A0       | 11/2003                | WO | 2019133880 A1 | 7/2019  |  |
| EP                       | 1352946 A4       | 12/2004                |    |               |         |  |

| (56)                                                                                                                                                                                                                                                                                                                                                                                                                                                                                                       | References Cited |        |  |
|------------------------------------------------------------------------------------------------------------------------------------------------------------------------------------------------------------------------------------------------------------------------------------------------------------------------------------------------------------------------------------------------------------------------------------------------------------------------------------------------------------|------------------|--------|--|
| FOREIGN PATENT DOCUMENTS                                                                                                                                                                                                                                                                                                                                                                                                                                                                                   |                  |        |  |
| WO                                                                                                                                                                                                                                                                                                                                                                                                                                                                                                         | 2019178701 A1    | 9/2019 |  |
| WO                                                                                                                                                                                                                                                                                                                                                                                                                                                                                                         | 2021066265 A1    | 4/2021 |  |
| OTHER PUBLICATIONS                                                                                                                                                                                                                                                                                                                                                                                                                                                                                         |                  |        |  |
| U.S. Appl. No. 16/103,884, Request for Continued Prosecution and Response to Final Office Action Dated, filed by Applicant dated Nov. 24, 2020.                                                                                                                                                                                                                                                                                                                                                            |                  |        |  |
| U.S. Appl. No. 16/103,884, Final Office Action dated Jun. 24, 2020.                                                                                                                                                                                                                                                                                                                                                                                                                                        |                  |        |  |
| U.S. Appl. No. 16/103,884, Response to Non-Final Office Action dated Mar. 10, 2020 filed by Applicant dated Jun. 10, 2020.                                                                                                                                                                                                                                                                                                                                                                                 |                  |        |  |
| U.S. Appl. No. 16/103,884, Non-Final Office Action dated Mar. 10, 2020.                                                                                                                                                                                                                                                                                                                                                                                                                                    |                  |        |  |
| Phillips 66, <i>Phillips 66, Petitioner v Magemā Technology LLC, Patent Owner, Petition for Inter Parties Review, Case IPR2021-01168, U.S. Pat. No. 10,308,884 B2, Dated Jul. 7, 2021, All pages.</i>                                                                                                                                                                                                                                                                                                      |                  |        |  |
| Phillips 66, <i>Phillips 66, Petitioner v Magemā Technology LLC, Patent Owner, Petition for Inter Parties Review, Case IPR2021-01173, U.S. Pat. No. 10,584,287 B2, Dated Jul. 12, 2021, All pages.</i>                                                                                                                                                                                                                                                                                                     |                  |        |  |
| Phillips 66, <i>Phillips 66, Petitioner v Magema Technology LLC, Patent Owner, Petition for Inter Parties Review, Case PR2021-01174, U.S. Pat. No. 10,604,709 B2, dated Jul. 13, 2021, All pages.</i>                                                                                                                                                                                                                                                                                                      |                  |        |  |
| Phillips 66, <i>Phillips 66, Petitioner v Magema Technology LLC, Patent Owner, Petition for Inter Parties Review, Case PR2021-01175, U.S. Pat. No. 10,533,141 B2, dated Jul. 14, 2021, All pages.</i>                                                                                                                                                                                                                                                                                                      |                  |        |  |
| International Organization for Standardization. Petroleum products—Fuels (class F)—Specifications of marine fuels (ISO Standard No. 8217:2017(E)), 2017, pp. 1-30 as presented in Petitioner's Exhibit 1003 in PR2021-01168; IPR2021-01173; IPR2021-01174; IPR2021-01175.                                                                                                                                                                                                                                  |                  |        |  |
| PHILLIPS 66, Petitioner's Exhibit 1015 Defendants Supplemental Preliminary Invalidity Contentions pp. 1-50, as presented in IPR2021-01168; IPR2021-01173; IPR2021-01174; IPR2021-01175.                                                                                                                                                                                                                                                                                                                    |                  |        |  |
| Mafalda Silva, Life Cycle Assessment of Marine Fuel Production, Jul. 2017, Norwegian University of Science and Technology, pp. 16-18, 32-35, 66 as presented Petitioner's Exhibit 1055 in IPR2021-01168; IPR2021-01173; IPR2021-01174; IPR2021-01175 and cited in Petitioner's Exhibit 1015 in IPR2021-01168; IPR2021-01173; IPR2021-01174; IPR2021-01175.                                                                                                                                                 |                  |        |  |
| Cambiasso Risso Group, Challenges of IMO's 0.5% Global Bunker Sulfur Cap, Dec. 12, 2016, p. 9, as presented in Petitioner's Exhibit 1057 in IPR2021-01168; IPR2021-01173; IPR2021-01174; IPR2021-01175 and cited in Petitioner's Exhibit 1015 in IPR2021-01168; IPR2021-01173; IPR2021-01174; IPR2021-01175.                                                                                                                                                                                               |                  |        |  |
| Phillips 66, Petitioner's Exhibit 1082 Declaration of Edward L. Sughrue II, pp. 1-84 as presented in IPR2021-01168; IPR2021-01173; IPR2021-01174; IPR2021-01175.                                                                                                                                                                                                                                                                                                                                           |                  |        |  |
| Surinder Parkash, Petroleum Fuels Manufacturing Handbook, 2010, R.R Donnelley, Publisher, pp. 82, 83, 84, 94, 95, 96 as presented in Petitioner's Exhibit 1102 in IPR2021-01174.                                                                                                                                                                                                                                                                                                                           |                  |        |  |
| International Search Report issued in corresponding International Application No. PCT/US2018/017855 dated Apr. 27, 2018 (3 pages).                                                                                                                                                                                                                                                                                                                                                                         |                  |        |  |
| International Search Report issued in corresponding International Application No. PCT/US2018/017863 dated Apr. 27, 2018 (3 pages).                                                                                                                                                                                                                                                                                                                                                                         |                  |        |  |
| Tesoro Refining & Marketing Co. Material Safety Data Sheet—Fuel Oil, pp. 1-10, Jul. 26, 2012, San Antonio, Texas, US.                                                                                                                                                                                                                                                                                                                                                                                      |                  |        |  |
| Tesoro Refining & Marketing Co. Material Safety Data Sheet—Marine Gas Oil, pp. 1-11, Nov. 17, 2012, San Antonio, Texas, US.                                                                                                                                                                                                                                                                                                                                                                                |                  |        |  |
| Tesoro Refining & Marketing Co. Material Safety Data Sheet—Resid pp. 1-10, Apr. 6, 2015, San Antonio, Texas, US.                                                                                                                                                                                                                                                                                                                                                                                           |                  |        |  |
| Courtmark Refining and Logistics, LLC, Material Safety Data Sheet—No. 6 Fuel Oil, Dec. 2012, pp. 1-4, Mt. Vernon, Indiana US.                                                                                                                                                                                                                                                                                                                                                                              |                  |        |  |
| Valero Marekting & Supply Company, Material Safety Data Sheet—Residual Fuel Oil, Dec. 4, 2010, pp. 1-14, San Antonio, Texas US.                                                                                                                                                                                                                                                                                                                                                                            |                  |        |  |
| Oceanbat SA. Material Safety Data Sheet—Marine Fuel Oil, Jul. 2013, pp. 1-7, Guayaquil Ecuador.                                                                                                                                                                                                                                                                                                                                                                                                            |                  |        |  |
| Exxonmobilcorporation, Material Safety Data Sheet—Marine Fuel Oil, pp. 1-12, Sep. 18, 2013, Fairfax Virginis US.                                                                                                                                                                                                                                                                                                                                                                                           |                  |        |  |
| Shell Trading (US) Company, Material Safety Data Sheet—Ultra Low Sulfur Fuel Oil, pp. 1-21, Jun. 19, 2018, Houston, Texas US.                                                                                                                                                                                                                                                                                                                                                                              |                  |        |  |
| Suncor Energy Inc., Material Safety Data Sheet—Heating Fuel Oil Type 6/Residual Marine Fuel, pp. 1-11, Jul. 6, 2018, Calgary Alberta Canada.                                                                                                                                                                                                                                                                                                                                                               |                  |        |  |
| Marathon Petroleum Company LP, Material Safety Data Sheet—Marathon No. 6 Fuel Oil, Dec. 7, 2010, pp. 1-14., Findlay, Ohio US.                                                                                                                                                                                                                                                                                                                                                                              |                  |        |  |
| BP Australia Pty Ltd., Material Safety Data Sheet—BP380 Marine Fuel, Oct. 27, 2011. pp. 1-6, Docklands, Victoria Australia.                                                                                                                                                                                                                                                                                                                                                                                |                  |        |  |
| U.S. Oil & Refining Co., Material Safety Data Sheet—Residual Fuel Oil, Dec. 18, 2008, pp. 1-11. Tacoma, Washington US.                                                                                                                                                                                                                                                                                                                                                                                     |                  |        |  |
| American Bureau of Shipping, Publication 31 Notes On Heavy Fuel Oil, 1984, pp. 1-68, Houston Texas US.                                                                                                                                                                                                                                                                                                                                                                                                     |                  |        |  |
| American Bureau of Shipping, Notes Use of Low Sulphur Marine Fuel for Main and Auxiliary Diesel Engines, Jan. 1, 2010, pp. 1-68, Houston Texas US ( <a href="https://www.eagle.org/eagleExternalPortalWEB&gt;ShowProperty/BEA%20Repository/pdfs/Regulatory/Docs/LowSulphurNote_Engine">https://www.eagle.org/eagleExternalPortalWEB&gt;ShowProperty/BEA%20Repository/pdfs/Regulatory/Docs/LowSulphurNote_Engine</a> ).                                                                                     |                  |        |  |
| Shuvi Zhang, Dong Liu, Wenan Deng, Guohe Que, A Review of Slurry-Phase Hydrocracking Heavy Oil Technology, Energy & Fuels, vol. 21, No. 6, Nov. 2007, pp. 3057-3062, American Chemical Society, Washington DC US.                                                                                                                                                                                                                                                                                          |                  |        |  |
| Peiman Pourmoghadam, Susan Davari, Zahra Delavar Moghaddam, A Technical And Economic Assessment of Fuel Oil Hydrotreating Technology For Steam Power Plant SO <sub>2</sub> and NO <sub>x</sub> Emissions Control, Advances in Environmental Technology vol. 2, Issue 1, Accepted Oct. 3, 2016, pp. 45-54, Iranian Research Organization For Science and Technology, Tehran Islamic Republic of Iran.                                                                                                       |                  |        |  |
| Dawoud Bahzad, Jamal Al-Fadhl, Ayyad Al-Dhafeeri, Aliabdal, Assessment of Selected Apparent Kinetic Parameters of the HDM and HDS reactions of Two Kuwaiti Residual Oils, Using Two Types of Commercial ARDS Catalysts, Energy & Fuels, vol. 24, Jan. 8, 2010, pp. 1495-1501, American Chemical Society, Washington DC US.                                                                                                                                                                                 |                  |        |  |
| X. Marafi, A. Hauser, a Stanislaus, Atmospheric Residual Desulfurization Process for Residual Oil Upgrading: An Investigation of the Effect of Catalyst Type and Operation Severity on Product Oil Quality, Energy & Fuels, vol. 20, Apr. 4, 2006, pp. 1145-1149, American Chemical Society, Washington DC US.                                                                                                                                                                                             |                  |        |  |
| M.M. Boduszynki, C.E. Rechsteiner, A.S.G. Shafzadeh, R.M.K. Carlson, Composition and Properties of Heavy Crudes, No. 1998 202 UNITAR Centre for Heavy Crude and Tar Sands, 1998, pp. 1-12, Canada.                                                                                                                                                                                                                                                                                                         |                  |        |  |
| Gard AS, Bunkers and Bunkering—A selection of articles previously published by Gard AS, Jan. 2014, pp. 1-53, Arendal Norway.                                                                                                                                                                                                                                                                                                                                                                               |                  |        |  |
| Monique B. Vermeire Everything You Need to Know About Marine Fuels, Jun. 2012, pp. 1-32, Ghent Belgium.                                                                                                                                                                                                                                                                                                                                                                                                    |                  |        |  |
| Chevron Lummus Group, Product web page—RDS/VRDS, 2013-2018, pp. 1-2, <a href="http://www.chevrontechnologymarketing.com/CLGtech/rds_vrds.aspx">http://www.chevrontechnologymarketing.com/CLGtech/rds_vrds.aspx</a> .                                                                                                                                                                                                                                                                                       |                  |        |  |
| T.M. Saleh, H. Ismail, J.E.Corbett, R.S. Bali, Commercial Experience in the Operation of Atmospheric Residue Desulfurization Unit in Kuwait national Petroleum Company At Mina Al-Ahmadi Refinery, Catalyst in Petroleum Refining, 1989, pp. 175-189, Elsevier Science Publishers B.V., Amsterdam The Netherlands.                                                                                                                                                                                         |                  |        |  |
| Victor S. Semeykina, Ekaterina V. Parkhomchuk, Alexander V. Polukhin, Pavel D. Parunin, Anton I. Lysikov, Artem B. Ayupov, Svetlana V. Cherepanova, Vladislav V. Kanazhevskiy, Vasil V. Kaichev, Tatyana S. Glazneva, Valentina V. Zvereva, CoMoNi Catalyst Texture and Surface Properties in Heavy Oil Processing. Part I: Hierarchical Macro/Mesoporous Alumina Support, Industrial & Engineering Chemistry Research, vol. 55, Feb. 29, 2016, pp. 3535-3545 American Chemical Society, Washington DC US. |                  |        |  |
| Victor S. Semeykina, Ekaterina V. Parkhomchuk, Alexander V. Polukhin, Pavel D. Parunin, Anton I. Lysikov, Artem B. Ayupov, Svetlana V. Cherepanova, Vladislav V. Kanazhevskiy, Vasil V. Kaichev, Tatyana S. Glazneva, Valentina V. Zvereva, CoMoNi Catalyst Texture and Surface Properties in Heavy Oil Processing. Part II: Macroporous Sepiolite-Like Mineral, Industrial & Engineering Chemistry Research, Vol 55,Aug. 1, 2016, pp. 9129-9139 American Chemical Society, Washington DC US.              |                  |        |  |
| Andre Hauser, Abdulaziz Marafi, Adel Almutairi, Anthony Stanislaus, Comparative Study of Hydrodemetallization (HDM) Catalyst Aging                                                                                                                                                                                                                                                                                                                                                                         |                  |        |  |

(56)

## References Cited

## OTHER PUBLICATIONS

- by Boscan Feed and Kuwait Atmospheric Residue, Energy & Fuels, vol. 22 Aug. 27, 2008, pp. 2952-2932, American Chemical Society, Washington DC US.
- Criterion Catalysts & Technologies LP, Residue Upgrading using Fixed-bed Hydroconversion Product Brochure , pp. 1 & 2, downloaded Jan. 9, 2018, web page [https://www.criterioncatalysts.com/products/product-applications/residue-upgrading/jcr\\_content/par/expandablelist/expandablesection\\_854912165.stream/1519837987339/9483494a3cf09f165f81](https://www.criterioncatalysts.com/products/product-applications/residue-upgrading/jcr_content/par/expandablelist/expandablesection_854912165.stream/1519837987339/9483494a3cf09f165f81)
- bab4f7a2e855ea62aa53f4885b9e56c0e9e0787e5939/criterion-fixed-. Criterion Catalysts & Technologies LP, Residue Upgrading Product Information Sheet, pp. 1 & 2, Aug. 2008, Houston Texas US.
- John-Lauren Tronche, Jelena Grigorjeva, Annie Siebert (editor), How Are Refiners Preparing For 2015 Marine Fuel Spec Changes?, pp. 1-2, Jun. 6, 2014, S&P. Global Platts. Houston Texas US.
- DNV GL Maritime, Hong Kong Requires Ocean-Going Vessels to Comply with 0.50% M/M Sulphur Limit While at Berth, Statutory Update No. 1, Mar. 2015, p. 1, DNV GL Maritime, Hamburg Germany.
- Mike Stockle, Tina Knight, Impact of Low-Sulphur Bunkers on Refineries, Catalysis 2009, pp. 1-7, [www.digitalrefining.com/article/1000090](http://www.digitalrefining.com/article/1000090), article based on presentation from the Nov. 2008 ERC Annual Meeting, Vienna Austria.
- Ekaterina V. Parkhomchuk, Anton I. Lysikov, Alexey G. Okunev, Pavel D. Parunin, Victoria S. Semeikina, Artem B. Ayupov, Valentina A. Trunova, Valentin N. Parmon, Meso/Macroporous CoMo Alumina Pellets for Hydrotreating of Heavy Oil, Industrial & Engineering Chemistry Research, vol. 15 Nov. 13, 2013, pp. 17117-17125 American Chemical Society, Washington DC US.
- Cristian J. Calderon Jorge Ancheyta, Modeling of Slurry-Phase Reactors for Hydrocracking of Heavy Oils, Energy & Fuels, vol. 30 Jan. 28, 2016, pp. 2525-2543, American Chemical Society, Washington DC US.
- DNV GL Maritime, Notice for Low Sulphur "Hybrid" Fuel Operation, Technical Update No. 3, Mar. 2015, pp. 1&2, DNV GL Maritime, Hamburg Germany.
- Abdul Waheed Bhutto, Rashid Abro, Shurong Goa, Tauqeer Abbas, Xiaochun Chen, Guangren Yu, Oxidative Desulfurization of Fuel Oils Using Ionic Liquids: A Review, Journal of the Taiwan Institute of Chemical Engineers, vol. 62, Feb. 28, 2016, pp. 84-97, Elsevier B.V. Amsterdam The Netherlands.
- I.V. Babich, J.A. Moulijn, Science and Technology of Novel Processes for Deep Desulfurization of Oil Refinery Streams: A Review, Fuel, vol. 82 ,Nov. 14, 2002, pp. 607-631 Elsevier B.V. Amsterdam The Netherlands Published first on the web via [fuelfirst.com](http://www.fuelfirst.com).
- A. Hauser, A. Marafi, A. Stanislaus, A. Al-Adwani, Relation Between Feed Quality and Coke Formation in a Three Stage Atmospheric Residue Desulfurization (ARDS) Process, Energy & Fuels, vol. 19 Feb. 8, 2005, pp. 544-553, American Chemical Society, Washington DC US.
- A Marafi, H. Al-Bazzaz, M. Al-Marri, F. Maruyama, M. Absi-Halbi, A. Stanislaus, Residual-Oil Hydrotreating Kinetics for graded Catalyst Systems: Effect of Original and Treated Feedstocks, Energy Fuels, vol. 17 (5), Jul. 2, 2003 pp. 1191-1197 American Chemical Society, Washington DC US.
- Hmaza Al-Bazza, Jia-Lin Kang, Dduha Chehadeh, Dawoud Bahzad, David Shan-Hill Wong, Shi-Shang Jang, Robust Predictions of Catalyst Deactivation of Atmospheric Residual Desulfurization, Energy Fuels, vol. 29, Oct. 21, 2015 pp. 7089-7100 American Chemical Society, Washington DC US.
- A.G. Okunev, E.V. Parkhomchuk, A.I Lysikov, P. D. Parunin, V.S. Semeykina, V.N. Parmon, Catalytic Hydroprocessing of Heavy Oil Feedstocks, Russian Chemical Reviews, vol. 84, Sep. 2015, pp. 981-999, Russian Academy of Sciences and Turpion Ltd. Moscow, Russia.
- Ernest Czermanski, Slawomir Drozdziecki, Maciej Matczak, Eugen Spangenberg, Bogusz Nisnicki, Sulphur Regulation—Technology Solutions and Economic Consequences, Institute of Maritime trans-
- port and Seaborne Trade, University of Gdansk, 2014, pp. 1-76, University of Gdansk, Gdansk Poland.
- Charles Olsen, Brian Watkins, Greg Rosinski, The Challenges of Processing FCC LCO, Catalogram 110 Special Edition, Fall 2011, pp. 6-8, W.R. Grace & Co Advanced Refining Technologies, Columbus Maryland, US.
- Yanzi Jia, Qinghe Yang, Shuling Sun, Hong Nie, Dadong Li, The Influence of Metal Deposits on Residue Hydrodemetallization Catalyst in the Absence and Presence of Coke, Energy Fuels, vol. 30 Feb. 22, 2016 pp. 2544-2554 American Chemical Society, Washington DC US.
- James G. Speight, Upgrading Heavy Oils and Residua: The Nature of the Problem, Catalysis on the Energy Scene, 1984, pp. 515-527, Elsevier Science Publishers B.V. Amsterdam, The Netherlands.
- Blessing Umana, Nan Zhang, Robin Smith, Development of Vacuum Residue Hydrodesulphurization—Hydrocracking Models and Their Integration with Refinery Hydrogen Networks, Industrial & Engineering Chemistry Research, vol. 55, Jan. 27, 2016, pp. 2391-2406, American Chemical Society, Washington DC US.
- Miike Stockle, Tina Knight, Impact of Low Sulphur Bunkers on Refineries, Catalysis, 2009, pp. 1-7, downloaded from website: [www.digitalrefining.com/article/1000090](http://www.digitalrefining.com/article/1000090).
- James G. Speight, The Desulfurization of Heavy Oils and Residua, 2nd Ed. 1999, Chapter 5, pp. 168-205, Marcel Dekker Inc. New York NY US.
- James G. Speight, The Desulfurization of Heavy Oils and Residua, 2nd Ed. 1999, Chapter 6, pp. 206-253, Marcel Dekker Inc. New York NY US.
- James G. Speight, The Desulfurization of Heavy Oils and Residua, 2nd Ed. 1999, Chapter 8, pp. 302-334, Marcel Dekker Inc. New York NY US.
- James G. Speight, The Desulfurization of Heavy Oils and Residua, 2nd Ed. 1999, Chapter 9, pp. 335-385, Marcel Dekker Inc. New York NY US.
- Mohammad Farhat Ali, et al. A review of methods for the demetallization of residual fuel oils, Fuel Processing Technology, Mar. 8, 2006, pp. 573-584, vol. 87, Elsevier B.V..
- Mohan S. Rana, et al., A review of recent advances on process technologies for upgrading of heavy oils and Residua, Fuel, Available online Sep. 7, 2006, pp. 1216-1231, vol. 86, Elsevier B.V..
- Carolina Leyva, et al., Activity and surface properties of NiMo/SiO<sub>2</sub>-Al<sub>2</sub>O<sub>3</sub> catalysts for hydroprocessing of heavy oils, Applied Catalysis A: General, Available online Feb. 28, 2012, pp. 1-12, vol. 425-426, Elsevier B.V..
- Oliver C. Mullins et al., Asphaltenes Explained for the Nonchemist, Petrophysics, Jun. 2015, pp. 266-275, vol. 56, No. 3.
- M. Ghasemi, et al., Phase Behavior and Viscosity Modeling of Athabasca Bitumen and Light Solvent Mixtures, SPE165416, Jun. 2013, pp. 1-26, Society of Petroleum Engineers.
- Marten Ternan, Catalytic Hydrogenation and Asphaltene Conversion of Athabasca Bitumen, The Canadian Journal of Chemical Engineering, Oct. 1983, pp. 689-696, vol. 61.
- Jeremi'as Marti'nez, et al.,Comparison of correlations to predict hydrotreating product properties during hydrotreating of heavy oils, Catalysis Today, Available online Dec. 5, 2009, pp. 300-307, vol. 150, Elsevier B.V..
- Luis C. Castneda, et al., Current situation of emerging technologies for upgrading of heavy oils, Catalysis Today, Available online Jul. 4, 2013, pp. 248-273, vol. 220-222, Elsevier B.V..
- C. Ferreira, et al., Hydrodesulfurization and hydrodemetallization of different origin vacuum residues: Characterization and reactivity, FUEL, Available online Apr. 14, 2012, pp. 1-11, <http://dx.doi.org/10.1016/j.fuel.2012.03.054>, Elsevier B.V..
- C.V. Philip, et al. GPC Characterization for Assessing Compatibility Problems with Heavy Fuel Oils, Fuel Processing Technology 1984: pp. 189-201., Elsevier B.V..
- Muhammad A. Altajam & Marten Ternan, Hydrocracking of Athabasca bitumen using Co-Mo catalysts supported on wide pore carbon extrudates, FUEL, Aug. 1989, pp. 955-960, Butterworth & Co. Publishers Ltd..
- J.W. Holmes & J.A. Bullin, Fuel Oil Compatibility Probed, Hydrocarbon Processing, Sep. 1983: pp. 101-103.

(56)

**References Cited**

OTHER PUBLICATIONS

- Charles J. Glover, & Jerry A. Bullin, Identification of Heavy Residual Oils by GC and GCMS, Journal of Environmental Science and Health A24(1), 1989: pp. 57-75.
- H. Puron, et al., Kinetic analysis of vacuum residue hydrocracking in early reaction stages, FUEL, Available online Sep. 27, 2013, pp. 408-414, vol. 117, Elsevier B.V.
- Yanet Villasna, et al. Upgrading and Hydrotreating of Heavy Oils and Residua, Energy Science and Technology, vol. 3, Oil and Natural Gas, 2015, pp. 304-328, Stadium Press LLC, Houston TX USA.

\* cited by examiner



FIG. 1



EIG. 2



FIG. 3



FIG. 4



FIG. 5



FIG. 6



FIG. 7



FIG. 8



FIG. 9





FIG. 12



FIG. 13



FIG. 14



FIG. 15



FIG. 16

**MULTI-STAGE DEVICE AND PROCESS FOR  
PRODUCTION OF A LOW SULFUR HEAVY  
MARINE FUEL OIL FROM DISTRESSED  
HEAVY FUEL OIL MATERIALS**

**BACKGROUND**

There are two basic marine fuel types: distillate based marine fuel, also known as Marine Gas Oil (MGO) or Marine Diesel Oil (MDO); and residual based marine fuel, also known as heavy marine fuel oil (HMFO). Distillate based marine fuel both MGO and MDO, comprises petroleum middle distillate fractions separated from crude oil in a refinery via a distillation process. Gasoil (also known as medium diesel) is a petroleum middle distillate in boiling range and viscosity between kerosene (light distillate) and lubricating oil (heavy distillate) containing a mixture of C<sub>10</sub> to C<sub>19</sub> hydrocarbons. Gasoil (a heavy distillate) is used to heat homes and is used blending with lighter middle distillates as a fuel for heavy equipment such as cranes, bulldozers, generators, bobcats, tractors and combine harvesters. Generally maximizing middle distillate recovery from heavy distillates mixed with petroleum residues is the most economic use of these materials by refiners because they can crack gas oils into valuable gasoline and distillates in a fluid catalytic cracking (FCC) unit. Diesel oils for road use are very similar to gas oils with road use diesel containing predominantly contain a middle distillate mixture of C<sub>10</sub> through C<sub>19</sub> hydrocarbons, which include approximately 64% aliphatic hydrocarbons, 1-2% olefinic hydrocarbons, and 35% aromatic hydrocarbons. Distillate based marine fuels (MDO and MGO) are essentially road diesel or gas oil fractions blended with up to 15% residual process streams, and optionally up to 5% volume of polycyclic aromatic hydrocarbons (asphaltenes). The residual and asphaltene materials are blended into the middle distillate to form MDO and MGO as a way to both swell volume and productively use these low value materials.

Asphaltenes are large and complex polycyclic hydrocarbons with a propensity to form complex and waxy precipitates, especially in the presence of aliphatic (paraffinic) hydrocarbons that are the primary component of Marine Diesel. Once asphaltenes have precipitated out, they are notoriously difficult to re-dissolve and are described as fuel tank sludge in the marine shipping industry and marine bunker fueling industry. One of skill in the art will appreciate that mixing Marine Diesel with asphaltenes and process residues is limited by the compatibility of the materials and formation of asphaltene precipitates and the minimum Cetane number required for such fuels.

Residual based fuels or Heavy Marine Fuel Oil (HMFO) are used by large ocean-going ships as fuel for large two stroke diesel engines for over 50 years. HMFO is a blend of the residues generated throughout the crude oil refinery process. Typical refinery streams combined to from HMFO may include, but are not limited to: atmospheric tower bottoms (i.e. atmospheric residues), vacuum tower bottoms (i.e. vacuum residues) visbreaker residue, FCC Light Cycle Oil (LCO), FCC Heavy Cycle Oil (HCO) also known as FCC bottoms, FCC Slurry Oil, heavy gas oils and delayed cracker oil (DCO), deasphalted oils (DAO); heavy aromatic residues and mixtures of polycyclic aromatic hydrocarbons, reclaimed land transport motor oils; pyrolysis oils and tars; asphaltene solids and tars; and minor portions (often less than 20% vol.) of middle distillate materials such as cutter oil, kerosene or diesel to achieve a desired viscosity. HMFO has a higher aromatic content (especially polynuclear aro-

matics and asphaltenes) than the marine distillate fuels noted above. The HMFO component mixture varies widely depending upon the crude slate (i.e. source of crude oil) processed by a refinery and the processes utilized within that refinery to extract the most value out of a barrel of crude oil. The HMFO is generally characterized as being highly viscous, high in sulfur and metal content (up to 5 wt %), and high in asphaltenes making HMFO the one product of the refining process that has historically had a per barrel value less than feedstock crude oil.

Industry statistics indicate that about 90% of the HMFO sold contains 3.5 weight % sulfur. With an estimated total worldwide consumption of HMFO of approximately 300 million tons per year, the annual production of sulfur dioxide by the shipping industry is estimated to be over 21 million tons per year. Emissions from HMFO burning in ships contribute significantly to both global marine air pollution and local marine air pollution levels.

The International Convention for the Prevention of Pollution from Ships, also known as the MARPOL convention or just MARPOL, as administered by the International Maritime Organization (IMO) was enacted to prevent marine pollution (i.e. marpol) from ships. In 1997, a new annex was added to the MARPOL convention; the Regulations for the Prevention of Air Pollution from Ships—Annex VI to minimize airborne emissions from ships (SO<sub>x</sub>, NO<sub>x</sub>, ODS, VOC) and their contribution to global air pollution. A revised Annex VI with tightened emissions limits was adopted in October 2008 and effective 1 Jul. 2010 (hereafter called Annex VI (revised) or simply Annex VI).

MARPOL Annex VI (revised) adopted in 2008 established a set of stringent air emissions limits for all vessel and designated Emission Control Areas (ECAs). The ECAs under MARPOL Annex VI are: i) Baltic Sea area—as defined in Annex I of MARPOL—SO<sub>x</sub> only; ii) North Sea area—as defined in Annex V of MARPOL—SO<sub>x</sub> only; iii) North American—as defined in Appendix VII of Annex VI of MARPOL—SO<sub>x</sub>, NO<sub>x</sub> and PM; and, iv) United States Caribbean Sea area—as defined in Appendix VII of Annex VI of MARPOL—SO<sub>x</sub>, NO<sub>x</sub> and PM.

Annex VI (revised) was codified in the United States by the Act to Prevent Pollution from Ships (APPS). Under the authority of APPS, the U.S. Environmental Protection Agency (the EPA), in consultation with the United States Coast Guard (USCG), promulgated regulations which incorporate by reference the full text of Annex VI. See 40 C.F.R. § 1043.100(a)(1). On Aug. 1, 2012 the maximum sulfur content of all marine fuel oils used onboard ships operating in US waters/ECA was reduced from 3.5% wt. to 1.00% wt. (10,000 ppm) and on Jan. 1, 2015 the maximum sulfur content of all marine fuel oils used in the North American ECA was lowered to 0.10% wt. (1,000 ppm). At the time of implementation, the United States government indicated that vessel operators must vigorously prepare to comply with the 0.10% wt. (1,000 ppm) US ECA marine fuel oil sulfur standard. To encourage compliance, the EPA and USCG refused to consider the cost of compliant low sulfur fuel oil to be a valid basis for claiming that compliant fuel oil was not available for purchase. For over five years there has been a very strong economic incentive to meet the marine industry demands for low sulfur HMFO, however technically viable solutions have not been realized and a premium price has been commanded by refiners to supply a low sulfur HMFO compliant with Annex VI sulfur emissions requirements in the ECA areas.

Since enactment in 2010, the global sulfur cap for HMFO outside of the ECA areas was set by Annex VI at 3.50% wt.

effective 1 Jan. 2012; with a further reduction to 0.50% wt, effective 1 Jan. 2020. The global cap on sulfur content in HMFO has been the subject of much discussion in both the marine shipping and marine fuel bunkering industry. There has been and continues to be a very strong economic incentive to meet the international marine industry demands for low sulfur HMFO (i.e. HMFO with a sulfur content less than 0.50 wt. %). Notwithstanding this global demand, solutions for transforming high sulfur HMFO into low sulfur HMFO have not been realized or brought to market. There is an on-going and urgent demand for processes and methods for making a low sulfur HMFO compliant with MARPOL Annex VI emissions requirements.

Replacement of Heavy Marine Fuel Oil with Marine Gas Oil or Marine Diesel:

One primary solution to the demand for low sulfur HMFO to simply replace high sulfur HMFO with marine gas oil (MGO) or marine diesel (MDO). The first major difficulty is the constraint in global supply of middle distillate materials that make up 85-90% vol of MGO and MDO. It is reported that the effective spare capacity to produce MGO is less than 100 million metric tons per year resulting in an annual shortfall in marine fuel of over 200 million metric tons per year. Refiners not only lack the capacity to increase the production of MGO, but they have no economic motivation because higher value and higher margins can be obtained from using middle distillate fractions for low sulfur diesel fuel for land-based transportation systems (i.e. trucks, trains, mass transit systems, heavy construction equipment, etc.).

Blending:

Another primary solution is the blending of high sulfur HMFO with lower sulfur containing fuels such as MGO or MDO low sulfur marine diesel (0.1% wt. sulfur) to achieve a Product HMFO with a sulfur content of 0.5% wt. In a straight blending approach (based on linear blending) every 1 ton of high sulfur HSFO (3.5% sulfur) requires 7.5 tons of MGO or MDO material with 0.1% wt. S to achieve a sulfur level of 0.5% wt. HMFO. One of skill in the art of fuel blending will immediately understand that blending hurts key properties of the HMFO, specifically lubricity, fuel density, CCAI, viscosity, flash point and other important physical bulk properties. Blending a mostly paraffinic-type distillate fuel (MGO or MDO) with a HMFO having a high poly aromatic content often correlates with poor solubility of asphaltenes. A blended fuel is likely to result in the precipitation of asphaltenes and/or waxing out of highly paraffinic materials from the distillate material forming an intractable fuel tank sludge. Fuel tank sludge causes clogging of filters and separators, transfer pumps and lines, build-up of sludge in storage tanks, sticking of fuel injection pumps, and plugged fuel nozzles. Such a risk to the primary propulsion system is not acceptable for a ship in the open ocean.

It should further be noted that blending of HMFO with marine distillate products (MGO or MDO) is not economically viable. A blender will be taking a high value product (0.1% S marine gas oil (MGO) or marine diesel (MDO)) and blending it 7.5 to 1 with a low value high sulfur HMFO to create a final IMO/MARPOL compliant HMFO (i.e. 0.5% wt. S Low Sulfur Heavy Marine Fuel Oil—LSHMF) which will sell at a discount to the value of the principle ingredient (i.e. MGO or MDO).

Processing of Residual Oils.

For the past several decades, the focus of refining industry research efforts related to the processing of heavy oils (crude oils, distressed oils, or residual oils) has been on upgrading the properties of these low value refinery process oils to create middle distillate and lighter oils with greater value.

The challenge has been that crude oil, distressed oil and residues contain high levels of sulfur, nitrogen, phosphorous, metals (especially vanadium and nickel); asphaltenes and exhibit a propensity to form carbon or coke on the catalyst. The sulfur and nitrogen molecules are highly refractory and aromatically stable and difficult and expensive to crack or remove. Vanadium and nickel porphyrins and other metal organic compounds are responsible for catalyst contamination and corrosion problems in the refinery. The sulfur, nitrogen, and phosphorous, must be removed because they are well-known poisons for the precious metal (platinum and palladium) catalysts utilized in the processes downstream of the atmospheric or vacuum distillation towers.

The difficulties treating atmospheric or vacuum residual streams has been known for many years and has been the subject of considerable research and investigation. Numerous residue-oil conversion processes have been developed in which the goals are same: 1) create a more valuable, preferably middle distillate range hydrocarbons; and 2) concentrate the contaminates such as sulfur, nitrogen, phosphorous, metals and asphaltenes into a form (coke, heavy coker residue, FCC slurry oil) for removal from the refinery stream. Well known and accepted practice in the refining industry is to increase the reaction severity (elevated temperature and pressure) to produce hydrocarbon products that are lighter and more purified, increase catalyst life times and remove sulfur, nitrogen, phosphorous, metals and asphaltenes from the refinery stream.

In summary, since the announcement of the MARPOL Annex VI standards reducing the global levels of sulfur in HMFO, refiners of crude oil have had modest success in their technical efforts to create a process for the production of a low sulfur substitute for high sulfur HMFO. Despite the strong governmental and economic incentives and needs of the international marine shipping industry, refiners have little economic reason to address the removal of environmental contaminates from high sulfur HMFOs. The global refining industry has been focused upon generating greater value from each barrel of oil by creating middle distillate hydrocarbons (i.e. diesel) and concentrating the environmental contaminates into increasingly lower value streams (i.e. residues) and products (petroleum coke, HMFO). Shipping companies have focused on short term solutions, such as the installation of scrubbing units, or adopting the limited use of more expensive low sulfur marine diesel and marine gas oils as a substitute for HMFO. On the open seas, most if not all major shipping companies continue to utilize the most economically viable fuel, that is HMFO. There remains a long standing and unmet need for processes and devices that remove the environmental contaminants (i.e. sulfur, nitrogen, phosphorous, metals especially vanadium and nickel) from HMFO without altering the qualities and properties that make HMFO the most economic and practical means of powering ocean going vessels.

## SUMMARY

It is a general objective to reduce the environmental contaminates from Distressed Fuel Oil Materials (DFOM) in a multi stage device implementing a pre-treatment stage that transforms the DFOM into a Feedstock Heavy Marine Fuel Oil (Feedstock HMFO) and a Core Process that removes the environmental contaminants from the Feedstock HMFO, minimizes the changes in the desirable properties of the

Feedstock HMFO and minimizes the production of by-product hydrocarbons (i.e. light hydrocarbons having C<sub>1</sub>-C<sub>4</sub> and wild naphtha (C<sub>4</sub>-C<sub>20</sub>)).

A first aspect and illustrative embodiment encompasses a multi-stage device for the production of a Product Heavy Marine Fuel Oil from Distressed Fuel Oil Materials, the device comprising: means for pre-treating the Distressed Fuel Oil Materials into a Feedstock HMFO, said means for pre-treating being selected from the group consisting of a stripper column; a distillation column; a divided wall distillation column; a reactive distillation column; a counter-current extraction unit; a fixed bed absorption unit, a solids separation unit, a blending unit; and combinations thereof. The illustrative device further includes a means for mixing a quantity of Feedstock Heavy Marine Fuel Oil with a quantity of Activating Gas mixture to give a Feedstock Mixture; means for heating the Feedstock mixture, wherein the means for mixing and means for heating communicate with each other; a Reaction System in fluid communication with the means for heating, wherein the Reaction System comprises one or more reactor vessels selected from the group consisting of: dense packed fixed bed trickle reactor; dense packed fixed bed up-flow reactor; ebulliated bed three phase up-flow reactor; fixed bed divided wall reactor; fixed bed three phase bubble reactor; fixed bed liquid full reactor, fixed bed high flux reactor; fixed bed structured catalyst bed reactor; fixed bed reactive distillation reactor and combinations thereof, and wherein the one or more reactor vessels contains one or more reaction sections configured to promote the transformation of the Feedstock Mixture to a Process Mixture. Also included in the illustrative embodiment is means for receiving said Process Mixture and separating the liquid components of the Process Mixture from the bulk gaseous components of the Process Mixture, said means for receiving in fluid communication with the reaction System; and means for separating any residual gaseous components and by-product hydrocarbon components from the Process Mixture to form a Product Heavy Marine Fuel Oil. In a preferred embodiment, the Reaction System comprises two or more reactor vessel wherein the reactor vessels are configured in a matrix of at least 2 reactors by 2 reactors. Another alternative and preferred embodiment of the Reactor System comprises at least six reactor vessels wherein the reactor vessels are configured in a matrix of at least 3 reactors arranged in series to form two reactor trains and wherein the 2 reactor trains arranged in parallel and configured so Process Mixture can be distributed across the matrix. In an illustrative embodiment, the Pre-Treatment Unit is a divided wall distillation column, preferably comprising one or more structured beds, wherein the one or more structured beds comprises a plurality of catalyst retention structures, each catalyst retentions structure comprising at least two coplanar fluid permeable metal sheets, wherein at least one of the fluid permeable sheets is corrugated and wherein the two coplanar fluid permeable metal sheets define one or more catalyst rich spaces and one or more catalyst lean spaces, wherein within the catalyst rich space there is one or more catalyst materials and optionally inert packing materials and wherein the catalyst lean spaces optionally contain an inert packing material. In another illustrative embodiment, the Pre-Treatment Unit is a reactive distillation column, wherein the reactive distillation column comprises one or more structured beds, wherein the one or more structured beds comprises a plurality of catalyst retention structures, each catalyst retentions structure comprising at least two coplanar fluid permeable metal sheets, wherein at least one of the fluid permeable sheets is corrugated and wherein the two coplanar fluid permeable metal sheets define one or more catalyst rich spaces and one or more catalyst lean spaces, wherein within the catalyst rich space there is one or more catalyst materials and optionally inert

packing materials and wherein the catalyst lean spaces optionally contain an inert packing material. It is envisioned that the Pre-Treatment Unit may be composed of more than one Pre-Treatment Unit, for example a blending unit, followed by a stripper column, wherein the stripper column separates the non-residual volatile components of the Distressed Fuel Oil Materials having a boiling temperature of less than 400° F. (205° C.) from the residual components of the Distressed Fuel Oil Materials and producing a distillate stream composed of at least a middle and heavy distillate and a residual stream composed of a Feedstock Heavy Marine Fuel Oil. In a preferred illustrative embodiment, the Pre-Treatment Unit comprises a blending unit, followed by a reactive distillation column, wherein the reactive distillation column comprises one or more structured beds, wherein the one or more structured beds comprises a plurality of catalyst retention structures, each catalyst retentions structure comprising at least two coplanar fluid permeable metal sheets, wherein at least one of the fluid permeable sheets is corrugated and wherein the two coplanar fluid permeable metal sheets define one or more catalyst rich spaces and one or more catalyst lean spaces, wherein within the catalyst rich space there is one or more catalyst materials and optionally inert packing materials and wherein the catalyst lean spaces optionally contain an inert packing material and wherein the reactive distillation column separates the non-residual volatile components of the Distressed Fuel Oil Materials having a boiling temperature of less than 400° F. (205° C.) from the residual components of the Distressed Fuel Oil Materials and producing a distillate stream composed of a middle and heavy distillate and a residual stream composed of a Feedstock Heavy Marine Fuel Oil.

A second aspect and illustrative embodiment encompasses a multi-stage process for the production of a Product Heavy Marine Fuel Oil that is ISO 8217:2017 and has a sulfur content (ISO 14596 or ISO 8754) between the range of 0.50 mass % to 0.05 mass % from DFOM that contain Environmental Contaminates. The illustrative process comprises of at least a pre-treatment process and the Core Process. The illustrative pre-treatment process involves the processing of the DFOM in a Pre-Treatment Unit under operative conditions to give a Feedstock Heavy Marine Fuel Oil that is ISO 8217 except for the environmental contaminates including a sulfur content (ISO 14596 or ISO 8754) between the range of 5.0 wt % to 0.50 wt %. The exemplary Core Process includes: mixing a quantity of the Feedstock Heavy Marine Fuel Oil with a quantity of Activating Gas mixture to give a Feedstock Mixture; contacting the Feedstock Mixture with one or more catalysts under reactive conditions in a Reaction System to form a Process Mixture from the Feedstock Mixture; receiving said Process Mixture and separating the liquid components of the Process Mixture from the bulk gaseous components of the Process Mixture; subsequently separating any residual gaseous components and by-product hydrocarbon components from the Product Heavy Marine Fuel Oil; and, discharging the Product Heavy Marine Fuel Oil.

#### DESCRIPTION OF DRAWINGS

FIG. 1 is a process block flow diagram of an illustrative Core Process to produce Product HMFO.

FIG. 2 is a process flow diagram of a multistage process for transforming the Feedstock HMFO and a subsequent Core Process to produce Product HMFO.

FIG. 3 is a process flow diagram of a first alternative configuration for the Reactor System (11) in FIG. 2.

FIG. 4 is a process flow diagram of a first alternative configuration for the Reactor System (11) in FIG. 2.

FIG. 5 is a process flow diagram of a multi-reactor configuration for the Reactor System (11) in FIG. 2.

FIG. 6 is a process flow diagram of a multi-reactor matrix configuration for the Reactor System (11) in FIG. 2.

FIG. 7 is a schematic illustration of a blending based Pre-Treatment Unit.

FIG. 8 is a schematic illustration of a stripper based Pre-Treatment Unit.

FIG. 9 is a schematic illustration of a distillation based Pre-Treatment Unit.

FIG. 10 is a side view of a catalyst retention structure of a first illustrative embodiment of a structured catalyst bed.

FIG. 11 is a side view of a first illustrative embodiment of a structured catalyst bed.

FIG. 12 is a side view of a catalyst retention structure of a second illustrative embodiment of a structured catalyst bed.

FIG. 13 is a side view of a first illustrative embodiment of a structured catalyst bed.

FIG. 14 is a schematic illustration of a Pre-Treatment Unit configured to operate under reactive distillation conditions.

FIG. 15 is a schematic illustration of a Pre-Treatment Unit configured to operate as a divide wall, fixed bed reactor with an internal reflux.

FIG. 16 is a schematic illustration of a Pre-Treatment Unit configured to operate as a divide wall, fixed bed reactor with an internal reflux integrated with the Core Process.

#### DETAILED DESCRIPTION

The inventive concepts as described herein utilize terms that should be well known to one of skill in the art, however certain terms are utilized having a specific intended meaning and these terms are defined below:

ISO 8217 is the international standard for the bulk physical properties and chemical characteristics for marine fuel products, as used herein the term specifically refers to the ISO 8217:2017; ISO 8217:2012; ISO 8217:2010 and ISO 8217: 2005 for residual based marine fuel grades with ISO 8217:2017 being preferred. One of skill in the art will appreciate that over 99% of the ISO 8217:2005 deliveries have bulk physical properties that comply with other three standards (except for sulfur levels and other Environmental Contaminates).

Distressed Fuel Oil Material (DFOM) is a residual petroleum material or blend of components that is not compliant with the ISO 8217 standards for residual marine fuels, examples include heavy hydrocarbons such as atmospheric residue; vacuum residue; FCC slurry oil; black oil; FCC cycle oil; vacuum gas oil; gas oil; distillates; coker gas oil; de-asphalted heavy oil; synthetic oils; viscbreaker residue; crude oils such as heavy crude oil; distressed crude oil; and the like or residual marine fuel or distillate and residual blends that have a 4 or 5 rating on ASTM D4740 compatibility tests, DFOM are not merchantable as Heavy Marine Fuel Oil.

Environmental Contaminates are organic and inorganic components of HMFO that result in the formation of  $\text{SO}_x$ ,  $\text{NO}_x$  and particulate materials upon combustion. More specifically: sulfur (ISO 14596 or ISO 8754); aluminum plus silicon (ISO 10478); Total Nitrogen (ASTM D5762) and vanadium content (ISO 14597).

Feedstock Heavy Marine Fuel Oil is a residual petroleum product compliant with the ISO 8217 standards for the physical properties or characteristics of a merchantable HMFO except for the concentration of Environmental

Contaminates, more specifically a Feedstock HMFO has a sulfur content greater than the global MARPOL Annex VI standard of 0.5% wt. sulfur (ISO 14596 or ISO 8754), and preferably and has a sulfur content (ISO 14596 or ISO 8754) between the range of 5.0% wt. to 1.0% wt.

Product HMFO is a residual petroleum product based fuel compliant with the ISO 8217 standards for the properties or characteristics of a merchantable HMFO and has a sulfur content lower than the global MARPOL Annex VI standard of 0.5% wt. sulfur (ISO 14596 or ISO 8754), and preferably a maximum sulfur content (ISO 14596 or ISO 8754) between the range of 0.05% wt. to 1.0% wt.

Activating Gas: is a mixture of gases utilized in the process combined with the catalyst to remove the environmental contaminates from the Feedstock HMFO.

Fluid communication: is the capability to transfer fluids (either liquid, gas or combinations thereof, which might have suspended solids) from a first vessel or location to a second vessel or location, this may encompass connections made by pipes (also called a line), spools, valves, intermediate holding tanks or surge tanks (also called a drum).

Merchantable quality: is a level of quality for a residual marine fuel oil so the fuel is fit for the ordinary purpose it should serve (i.e. serve as a residual fuel source for a marine ship) and can be commercially sold as and is fungible and compatible with other heavy or residual marine bunker fuels.

Bbl or bbl: is a standard volumetric measure for oil; 1 bbl=0.1589873 m<sup>3</sup>; or 1 bbl=158.9873 liters; or 1 bbl=42.00 US liquid gallons.

Bpd or bpd: is an abbreviation for Bbl per day. SCF: is an abbreviation for standard cubic foot of a gas; a standard cubic foot (at 14.73 psi and 60° F.) equals 0.0283058557 standard cubic meters (at 101.325 kPa and 15° C.).

Bulk Properties: are broadly defined as the physical properties or characteristics of a merchantable HMFO as required by ISO 8217; and the measurements include: kinematic viscosity at 50° C. as determined by ISO 3104; density at 15° C. as determined by ISO 3675; CCAI value as determined by ISO 8217, ANNEX B; flash point as determined by ISO 2719; total sediment—aged as determined by ISO 10307-2; and carbon residue—micro method as determined by ISO 10370.

Core Process:

The inventive concepts are illustrated in more detail in this description referring to the drawings. FIG. 1 shows the generalized block process flows for a Core Process of reducing the environmental contaminates in a Feedstock HMFO and producing a Product HMFO. A predetermined volume of Feedstock HMFO (2) is mixed with a predetermined quantity of Activating Gas (4) to give a Feedstock Mixture. The Feedstock HMFO utilized generally complies with the bulk physical and certain key chemical properties for a residual marine fuel oil otherwise compliant with ISO 8217 exclusive of the Environmental Contaminates. More particularly, when the Environmental Contaminant is sulfur, the concentration of sulfur in the Feedstock HMFO may be between the range of 5.0% wt. to 1.0% wt. The Feedstock HMFO should have bulk physical properties required of an ISO 8217 compliant HMFO. The Feedstock HMFO should exhibit the Bulk Properties of: a maximum of kinematic

viscosity at 50° C. (ISO 3104) between the range from 180 mm<sup>2</sup>/s to 700 mm<sup>2</sup>/s; a maximum of density at 15° C. (ISO 3675) between the range of 991.0 kg/m<sup>3</sup> to 1010.0 kg/m<sup>3</sup>; a CCAI in the range of 780 to 870; and a flash point (ISO 2719) no lower than 60° C. Properties of the Feedstock HMFO connected to the formation of particulate material (PM) include: a total sediment—aged (ISO 10307-2) less than 0.10% wt. and a carbon residue—micro method (ISO 10370) less than 20.00% wt. and a aluminum plus silicon (ISO 10478) content of less than 60 mg/kg. Environmental Contaminates other than sulfur that may be present in the Feedstock HMFO over the ISO 8217 requirements may include vanadium, nickel, iron, aluminum and silicon substantially reduced by the process of the present invention. However, one of skill in the art will appreciate that the vanadium content serves as a general indicator of these other Environmental Contaminates. In one preferred embodiment the vanadium content is ISO compliant so the Feedstock HMFO has a vanadium content (ISO 14597) no greater than the range from 350 mg/kg to 450 ppm mg/kg.

As for the properties of the Activating Gas, the Activating Gas should be selected from mixtures of nitrogen, hydrogen, carbon dioxide, gaseous water, and methane. The mixture of gases within the Activating Gas should have an ideal gas partial pressure of hydrogen (pH2) greater than 80% of the total pressure of the Activating Gas mixture (P) and more preferably wherein the Activating Gas has an ideal gas partial pressure of hydrogen (pH2) greater than 90% of the total pressure of the Activating Gas mixture (P). It will be appreciated by one of skill in the art that the molar content of the Activating Gas is another criterion the Activating Gas should have a hydrogen mole fraction in the range between 80% and 100% of the total moles of Activating Gas mixture.

The Feedstock Mixture (i.e. mixture of Feedstock HMFO and Activating Gas) is brought up to the process conditions of temperature and pressure and introduced into a Reactor System, preferably a reactor vessel, so the Feedstock Mixture is then contacted under reactive conditions with one or more catalysts (8) to form a Process Mixture from the Feedstock Mixture.

The Core Process conditions are selected so the ratio of the quantity of the Activating Gas to the quantity of Feedstock HMFO is 250 scf gas/bbl of Feedstock HMFO to 10,000 scf gas/bbl of Feedstock HMFO; and preferably between 2000 scf gas/bbl of Feedstock HMFO 1 to 5000 scf gas/bbl of Feedstock HMFO more preferably between 2500 scf gas/bbl of Feedstock HMFO to 4500 scf gas/bbl of Feedstock HMFO. The process conditions are selected so the total pressure in the first vessel is between of 250 psig and 3000 psig; preferably between 1000 psig and 2500 psig, and more preferably between 1500 psig and 2200 psig. The process reactive conditions are selected so the indicated temperature within the first vessel is between of 500° F. to 900° F., preferably between 650° F. and 850° F. and more preferably between 680° F. and 800° F. The process conditions are selected so the liquid hourly space velocity within the first vessel is between 0.05 oil/hour/m<sup>3</sup> catalyst and 1.0 oil/hour/m<sup>3</sup> catalyst; preferably between 0.08 oil/hour/m<sup>3</sup> catalyst and 0.5 oil/hour/m<sup>3</sup> catalyst; and more preferably between 0.1 oil/hour/m<sup>3</sup> catalyst and 0.3 oil/hour/m<sup>3</sup> catalyst to achieve deep desulfurization with product sulfur levels below 0.1 ppmw.

One of skill in the art will appreciate that the Core Process reactive conditions are determined considering the hydraulic capacity of the unit. Exemplary hydraulic capacity for the treatment unit may be between 100 bbl of Feedstock HMFO/day and 100,000 bbl of Feedstock HMFO/day, preferably

between 1000 bbl of Feedstock HMFO/day and 60,000 bbl of Feedstock HMFO/day, more preferably between 5,000 bbl of Feedstock HMFO/day and 45,000 bbl of Feedstock HMFO/day, and even more preferably between 10,000 bbl of Feedstock HMFO/day and 30,000 bbl of Feedstock HMFO/day.

One of skill in the art will appreciate that a fixed bed reactor using a supported transition metal heterogeneous catalyst will be the technically easiest to implement and is preferred. However, alternative reactor types may be utilized including, but not limited to: ebulliated or fluidized bed reactors see US2017008160; US20170355913; U.S. Pat. Nos. 6,620,311; 5,298,151; 4,764,347 4,312,741 the contents of which are incorporated herein by reference; structured bed reactors (see U.S. Pat. Nos. 4,731,229; 5,073,236; 5,266,546; 5,431,890; 5,730,843; US2002068026; US20020038066; US20020068026; US20030012711; US20060065578; US20070209966; US20090188837; US2010063334; US2010228063; US20110214979; US20120048778; US20150166908; US20150275105; 20160074824; 20170101592 and US20170226433, the contents of which are incorporated herein by reference; three-phase bubble reactors see US20060047163; U.S. Pat. Nos. 7,960,581; 7,504,535; 4,666,588 4,345,992; 4,389,301; 3,870,623; and 2,875,150 the contents of which are incorporated herein by reference; reactive distillation bed reactors see U.S. Pat. Nos. 4,731,229; 5,073,236; 5,266,546; 5,431,890; 5,730,843; US2002068026; US 20020038066; US20020068026; US 20030012711; US20060065578; US20070209966; US20090188837; US2010063334; US2010228063; US20110214979; US20120048778; US20150166908; US20150275105; 20160074824; 20170101592 and US20170226433, the contents of which are incorporated herein by reference and the like all of which may be co-current or counter current. We also assume high flux or liquid full type reactors may be used such as those disclosed in U.S. Pat. Nos. 6,123,835; 6,428,686; 6,881,326; 7,291,257; 7,569,136 and other similar and related patents and patent applications.

40 The transition metal heterogeneous catalyst utilized comprises a porous inorganic oxide catalyst carrier and a transition metal catalytic metal. The porous inorganic oxide catalyst carrier is at least one carrier selected from the group consisting of alumina, alumina/boria carrier, a carrier containing metal-containing aluminosilicate, alumina/phosphorus carrier, alumina/alkaline earth metal compound carrier, alumina/titania carrier and alumina/zirconia carrier. The transition metal catalytic metal component of the catalyst is one or more metals selected from the group consisting of group 6, 8, 9 and 10 of the Periodic Table. In a preferred and illustrative embodiment, the transition metal heterogeneous catalyst is a porous inorganic oxide catalyst carrier and a transition metal catalyst, in which the preferred porous inorganic oxide catalyst carrier is alumina and the preferred transition metal catalyst is Ni—Mo, Co—Mo, Ni—W or Ni—Co—Mo. The process by which the transition metal heterogeneous catalyst is manufactured is known in the literature and preferably the catalysts are commercially available as hydrodemetallization catalysts, transition catalysts, desulfurization catalyst and combinations of these which might be pre-sulfided.

45 The Process Mixture (10) in this Core Process is removed from the Reactor System (8) and from being in contact with the one or more catalyst and is sent via fluid communication to a second vessel (12), preferably a gas-liquid separator or hot separators and cold separators, for separating the liquid components (14) of the Process Mixture from the bulk

## 11

gaseous components (16) of the Process Mixture. The gaseous components (16) are treated beyond the battery limits of the immediate process. Such gaseous components may include a mixture of Activating Gas components and lighter hydrocarbons (mostly methane, ethane and propane but some wild naphtha) that may have been formed as part of the by-product hydrocarbons from the process.

The Liquid Components (16) in this Core Process are sent via fluid communication to a third vessel (18), preferably a fuel oil product stripper system, for separating any residual gaseous components (20) and by-product hydrocarbon components (22) from the Product HMFO (24). The residual gaseous components (20) may be a mixture of gases selected from the group consisting of: nitrogen, hydrogen, carbon dioxide, hydrogen sulfide, gaseous water, C<sub>1</sub>-C<sub>5</sub> hydrocarbons. This residual gas is treated outside of the battery limits of the immediate process, combined with other gaseous components (16) removed from the Process Mixture (10) in the second vessel (12). The liquid by-product hydrocarbon component, which are condensable hydrocarbons formed in the process (22) may be a mixture selected from the group consisting of C<sub>4</sub>-C<sub>20</sub> hydrocarbons (wild naphtha) (naphtha—diesel) and other condensable light liquid (C<sub>3</sub>-C<sub>8</sub>) hydrocarbons that can be utilized as part of the motor fuel blending pool or sold as gasoline and diesel blending components on the open market. These liquid by-product hydrocarbons should be less than 15% wt., preferably less than 5% wt. and more preferably less than 3% wt. of the overall process mass balance.

The Product HMFO (24) resulting from the Core Process is discharged via fluid communication into storage tanks beyond the battery limits of the immediate process. The Product HMFO complies with ISO 8217 and has a maximum sulfur content (ISO 14596 or ISO 8754) between the range of 0.05 mass % to 1.0 mass % preferably a sulfur content (ISO 14596 or ISO 8754) between the range of 0.05 mass % ppm and 0.7 mass % and more preferably a sulfur content (ISO 14596 or ISO 8754) between the range of 0.1 mass % and 0.5 mass %. The vanadium content of the Product HMFO is also ISO compliant with a maximum vanadium content (ISO 14597) between the range from 350 mg/kg to 450 ppm mg/kg, preferably a vanadium content (ISO 14597) between the range of 200 mg/kg and 300 mg/kg and more preferably a vanadium content (ISO 14597) between the range of 50 mg/kg and 100 mg/kg.

The Product HMFO should have bulk physical properties that are ISO 8217 compliant. The Product HMFO should exhibit Bulk Properties of: a maximum of kinematic viscosity at 50° C. (ISO 3104) between the range from 180 mm<sup>2</sup>/s to 700 mm<sup>2</sup>/s; a maximum of density at 15° C. (ISO 3675) between the range of 991.0 kg/m<sup>3</sup> to 1010.0 kg/m<sup>3</sup>; a CCAI value in the range of 780 to 870; a flash point (ISO 2719) no lower than 60.0° C.; a total sediment—aged (ISO 10307-2) of less than 0.10 mass %; and a carbon residue—micro method (ISO 10370) lower than 20.00 mass %. The Product HMFO should have an aluminum plus silicon (ISO 10478) content of less than 60 mg/kg.

Relative the Feedstock HMFO, the Product HMFO will have a sulfur content (ISO 14596 or ISO 8754) between 1% and 20% of the maximum sulfur content of the Feedstock HMFO. That is the sulfur content of the Product HMFO will be reduced by about 80% or greater when compared to the Feedstock HMFO. Similarly, the vanadium content (ISO 14597) of the Product HMFO is between 1% and 20% of the maximum vanadium content of the Feedstock HMFO. One of skill in the art will appreciate that the above data indicates a substantial reduction in sulfur and vanadium content

## 12

indicate a process having achieved a substantial reduction in the Environmental Contaminates from the Feedstock HMFO while maintaining the desirable properties of an ISO 8217 compliant and merchantable HMFO.

As a side note, the residual gaseous component is a mixture of gases selected from the group consisting of: nitrogen, hydrogen, carbon dioxide, hydrogen sulfide, gaseous water, C<sub>1</sub>-C<sub>5</sub> hydrocarbons. An amine scrubber will effectively remove the hydrogen sulfide content which can then be processed using technologies and processes well known to one of skill in the art. In one preferable illustrative embodiment, the hydrogen sulfide is converted into elemental sulfur using the well-known Claus process. An alternative embodiment utilizes a proprietary process for conversion of the Hydrogen sulfide to hydrosulfuric acid. Either way, the sulfur is removed from entering the environment prior to combusting the HMFO in a ships engine. The cleaned gas can be vented, flared or more preferably recycled back for use as Activating Gas.

## 20 Product HMFO

The Product HMFO resulting from the disclosed illustrative process is of merchantable quality for sale and use as a heavy marine fuel oil (also known as a residual marine fuel oil or heavy bunker fuel) and exhibits the bulk physical properties required for the Product HMFO to be an ISO 8217 compliant (preferably ISO 8217 (2017)) residual marine fuel oil. The Product HMFO should exhibit the Bulk Properties of: a maximum of kinematic viscosity at 50° C. (ISO 3104) between the range from 180 mm<sup>2</sup>/s to 700 mm<sup>2</sup>/s; a density at 15° C. (ISO 3675) between the range of 991.0 kg/m<sup>3</sup> to 1010.0 kg/m<sup>3</sup>; a CCAI is in the range of 780 to 870; a flash point (ISO 2719) no lower than 60° C.; a total sediment—aged (ISO 10307-2) less than 0.10% wt.; a carbon residue—micro method (ISO 10370) less than 20.00% wt.; The product HMFO should have an aluminum plus silicon (ISO 10478) content no more than of 60 mg/kg.

The Product HMFO has a sulfur content (ISO 14596 or ISO 8754) less than 0.5 wt % and preferably less than 0.1% wt. and complies with the IMO Annex VI (revised) requirements for a low sulfur and preferably an ultra-low sulfur HMFO. That is the sulfur content of the Product HMFO has been reduced by about 80% and preferably 90% or greater when compared to the Feedstock HMFO. Similarly, the vanadium content (ISO 14597) of the Product Heavy Marine Fuel Oil is less than 20% and more preferably less than 10% of the maximum vanadium content of the Feedstock Heavy Marine Fuel Oil. One of skill in the art will appreciate that a substantial reduction in sulfur and vanadium content of the Feedstock HMFO indicates a process having achieved a substantial reduction in the Environmental Contaminates from the Feedstock HMFO; of equal importance is this has been achieved while maintaining the desirable properties of an ISO 8217 compliant HMFO.

The Product HMFO not only complies with ISO 8217 (and is merchantable as a residual marine fuel oil or bunker fuel), the Product HMFO has a maximum sulfur content (ISO 14596 or ISO 8754) between the range of 0.05% wt. to 1.0% wt. preferably a sulfur content (ISO 14596 or ISO 8754) between the range of 0.05% wt. ppm and 0.5% wt. and more preferably a sulfur content (ISO 14596 or ISO 8754) between the range of 0.1% wt. and 0.5% wt. The vanadium content of the Product HMFO is well within the maximum vanadium content (ISO 14597) required for an ISO 8217 residual marine fuel oil exhibiting a vanadium content lower than 450 ppm mg/kg, preferably a vanadium content (ISO 14597) lower than 300 mg/kg and more preferably a vanadium content (ISO 14597) less than 50 mg/kg.

One knowledgeable in the art of marine fuel blending, bunker fuel formulations and the fuel requirements for marine shipping fuels will readily appreciate that without further compositional changes or blending, the Product HMFO can be sold and used as a low sulfur MARPOL Annex VI compliant heavy (residual) marine fuel oil that is a direct substitute for the high sulfur heavy (residual) marine fuel oil or heavy bunker fuel currently in use. One illustrative embodiment is an ISO 8217 compliant low sulfur heavy marine fuel oil comprising (and preferably consisting essentially of) hydroprocessed ISO 8217 compliant high sulfur heavy marine fuel oil, wherein the sulfur levels of the hydroprocessed ISO 8217 compliant high sulfur heavy marine fuel oil is greater than 0.5% wt. and wherein the sulfur levels of the ISO 8217 compliant low sulfur heavy marine fuel oil is less than 0.5% wt. Another illustrative embodiment is an ISO 8217 compliant ultra-low sulfur heavy marine fuel oil comprising (and preferably consisting essentially of) a hydroprocessed ISO 8217 compliant high sulfur heavy marine fuel oil, wherein the sulfur levels of the hydroprocessed ISO 8217 compliant high sulfur heavy marine fuel oil is greater than 0.5% wt. and wherein the sulfur levels of the ISO 8217 compliant low sulfur heavy marine fuel oil is less than 0.1% wt.

Because of the present invention, multiple economic and logistical benefits to the bunkering and marine shipping industries can be realized. The benefits include minimal changes to the existing heavy marine fuel bunkering infrastructure (storage and transferring systems); minimal changes to shipboard systems are needed to comply with emissions requirements of MARPOL Annex VI (revised); no additional training or certifications for crew members will be needed, amongst the realizable benefits. Refiners will also realize multiple economic and logistical benefits, including: no need to alter or rebalance the refinery operations, crude sources, and product streams to meet a new market demand for low sulfur or ultralow sulfur HMFO; no additional units are needed in the refinery with additional hydrogen or sulfur capacity because the illustrative process can be conducted as a stand-alone unit; refinery operations can remain focused on those products that create the greatest value from the crude oil received (i.e. production of petrochemicals, gasoline and distillate (diesel); refiners can continue using the existing slates of crude oils without having to switch to sweeter or lighter crudes to meet the environmental requirements for HMFO products.

#### Heavy Marine Fuel Composition

One aspect of the present inventive concept is a fuel composition comprising, but preferably consisting essentially of, the Product HMFO resulting from the processes disclosed, and may optionally include Diluent Materials. The Product HMFO itself complies with ISO 8217 and meets the global IMO Annex VI requirements for maximum sulfur content (ISO 14596 or ISO 8754). If ultra-low levels of sulfur are desired, the process of the present invention achieves this and one of skill in the art of marine fuel blending will appreciate that a low sulfur or ultra-low sulfur Product HMFO can be utilized as a primary blending stock to form a global IMO Annex VI compliant low sulfur Heavy Marine Fuel Composition. Such a low sulfur Heavy Marine Fuel Composition will comprise (and preferably consist essentially of): a) the Product HMFO and b) Diluent Materials. In one embodiment, the majority of the volume of the Heavy Marine Fuel Composition is the Product HMFO with the balance of materials being Diluent Materials. Preferably, the Heavy Marine Fuel Composition is at least 75% by volume, preferably at least 80% by volume, more preferably

at least 90% by volume, and furthermore preferably at least 95% by volume Product HMFO with the balance being Diluent Materials.

Diluent Materials may be hydrocarbon or non-hydrocarbon based materials mixed into or combined with or added to, or solid particle materials suspended in, the Product HMFO. The Diluent Materials may intentionally or unintentionally alter the composition of the Product HMFO but not so the resulting mixture violates the ISO 8217 standards for residual marine fuels or fails to have a sulfur content lower than the global MARPOL standard of 0.5% wt. sulfur (ISO 14596 or ISO 8754). Examples of Diluent Materials considered hydrocarbon based materials include: Feedstock HMFO (i.e. high sulfur HMFO); distillate based fuels such as road diesel, gas oil, MGO or MDO; cutter oil (which is used in formulating residual marine fuel oils); renewable oils and fuels such as biodiesel, methanol, ethanol, and the like; synthetic hydrocarbons and oils based on gas to liquids technology such as Fischer-Tropsch derived oils, synthetic oils such as those based on polyethylene, polypropylene, dimer, trimer and poly butylene; refinery residues or other hydrocarbon oils such as atmospheric residue, vacuum residue, fluid catalytic cracker (FCC) slurry oil, FCC cycle oil, pyrolysis gasoil, cracked light gas oil (CLGO), cracked heavy gas oil (CHGO), light cycle oil (LCO), heavy cycle oil (HCO), thermally cracked residue, coker heavy distillate, bitumen, de-asphalted heavy oil, visbreaker residue, slop oils, asphaltinic oils; used or recycled motor oils; lube oil aromatic extracts and crude oils such as heavy crude oil, distressed crude oils and similar materials that might otherwise be sent to a hydrocracker or diverted into the blending pool for a prior art high sulfur heavy (residual) marine fuel oil. Examples of Diluent Materials considered non-hydrocarbon based materials include: residual water (i.e. water absorbed from the humidity in the air or water that is miscible or solubilized, sometimes as microemulsions, into the hydrocarbons of the Product HMFO), fuel additives which can include, but are not limited to detergents, viscosity modifiers, pour point depressants, lubricity modifiers, de-hazers (e.g. alkoxylated phenol formaldehyde polymers), antifoaming agents (e.g. polyether modified polysiloxanes); ignition improvers; anti rust agents (e.g. succinic acid ester derivatives); corrosion inhibitors; anti-wear additives, anti-oxidants (e.g. phenolic compounds and derivatives), coating agents and surface modifiers, metal deactivators, static dissipating agents, ionic and nonionic surfactants, stabilizers, cosmetic colorants and odorants and mixtures of these. A third group of Diluent Materials may include suspended solids or fine particulate materials that are present because of the handling, storage and transport of the Product HMFO or the Heavy Marine Fuel Composition, including but not limited to: carbon or hydrocarbon solids (e.g. coke, graphitic solids, or micro-agglomerated asphaltenes), iron rust and other oxidative corrosion solids, fine bulk metal particles, paint or surface coating particles, plastic or polymeric or elastomer or rubber particles (e.g. resulting from the degradation of gaskets, valve parts, etc. . . . ), catalyst fines, ceramic or mineral particles, sand, clay, and other earthen particles, bacteria and other biologically generated solids, and mixtures of these that may be present as suspended particles, but otherwise don't detract from the merchantable quality of the Heavy Marine Fuel Composition as an ISO 8217 compliant heavy (residual) marine fuel.

The blend of Product HMFO and Diluent Materials must be of merchantable quality as a low sulfur heavy (residual) marine fuel. That is the blend must be suitable for the intended use as heavy marine bunker fuel and generally be

fungible and compatible as a bunker fuel for ocean going ships. Preferably the Heavy Marine Fuel Composition must retain the bulk physical properties required of an ISO 8217 compliant residual marine fuel oil and a sulfur content lower than the global MARPOL standard of 0.5% wt. sulfur (ISO 14596 or ISO 8754) so that the material qualifies as MARPOL Annex VI Low Sulfur Heavy Marine Fuel Oil (LS-HMFO). The sulfur content of the Product HMFO can be lower than 0.5% wt. (i.e. below 0.1% wt sulfur (ISO 14596 or ISO 8754)) to qualify as a MARPOL Annex VI compliant Ultra-Low Sulfur Heavy Marine Fuel Oil (ULS-HMFO) and a Heavy Marine Fuel Composition likewise can be formulated to qualify as a MARPOL Annex VI compliant ULS-HMFO suitable for use as marine bunker fuel in the ECA zones. To qualify as an ISO 8217 qualified fuel, the Heavy Marine Fuel Composition of the present invention must meet those internationally accepted standards. Those include Bulk Properties of: a maximum of kinematic viscosity at 50° C. (ISO 3104) between the range from 180 mm<sup>2</sup>/s to 700 mm<sup>2</sup>/s; a density at 15° C. (ISO 3675) between the range of 991.0 kg/m<sup>3</sup> to 1010.0 kg/m<sup>3</sup>; a CCAI is in the range of 780 to 870; a flash point (ISO 2719) no lower than 60° C.; a total sediment—aged (ISO 10307-2) less than 0.10% wt.; and a carbon residue—micro method (ISO 10370) less than 20% wt. The Heavy Marine Fuel Composition must also have an aluminum plus silicon (ISO 10478) content no more than of 60 mg/kg.

#### Core Process Production Plant Description:

Turning now to a more detailed illustrative embodiment of a production plant, FIG. 2 shows a schematic for a production plant implementing the Core Process described above for reducing the environmental contaminates in a Feedstock HMFO to produce a Product HMFO. It will be appreciated by one of skill in the art will appreciate that FIG. 2 is a generalized schematic drawing, and the exact layout and configuration of a plant will depend upon factors such as location, production capacity, environmental conditions (i.e. wind load, etc.) and other factors and elements that a skilled detailed engineering firm can provide. Such variations are contemplated and within the scope of the present disclosure.

In FIG. 2, Feedstock HMFO (A) is fed from outside the battery limits (OSBL) to the Oil Feed Surge Drum (1) that receives feed from outside the battery limits (OSBL) and provides surge volume adequate to ensure smooth operation of the unit. Entrained materials are removed from the Oil Feed Surge Drum by way of a stream (1c) for treatment OSBL.

The Feedstock HMFO (A) is withdrawn from the Oil Feed Surge Drum (1) via line (1b) by the Oil Feed Pump (3) and is pressurized to a pressure required for the process. The pressurized HMFO (A') then passes through line (3a) to the Oil Feed/Product Heat Exchanger (5) where the pressurized HMFO Feed (A') is partially heated by the Product HMFO (B). The pressurized Feedstock HMFO (A') passing through line (5a) is further heated against the effluent from the Reactor System (E) in the Reactor Feed/Effluent Heat Exchanger (7).

The heated and pressurized Feedstock HMFO (A'') in line (7a) is then mixed with Activating Gas (C) provided via line (23c) at Mixing Point (X) to form a Feedstock Mixture (D). The mixing point (X) can be any well known gas/liquid mixing system or entrainment mechanism well known to one skilled in the art.

The Feedstock Mixture (D) passes through line (9A) to the Reactor Feed Furnace (9) where the Feedstock Mixture (D) is heated to the specified process temperature. The

Reactor Feed Furnace (9) may be a fired heater furnace or any other kind to type of heater as known to one of skill in the art if it will raise the temperature of the Feedstock Mixture (D) to the desired temperature for the process conditions.

The fully Heated Feedstock Mixture (D') exits the Reactor Feed Furnace (9) via line 9B and is fed into the Reactor System (11). The fully Heated Feedstock Mixture (D') enters the Reactor System (11) where environmental contaminates, such a sulfur, nitrogen, and metals are preferentially removed from the Feedstock HMFO component of the fully Heated Feedstock Mixture. The Reactor System contains a catalyst which preferentially removes the sulfur compounds in the Feedstock HMFO component by reacting them with hydrogen in the Activating Gas to form hydrogen sulfide. The Reactor System will also achieve demetallization, denitrogenation, and a certain amount of ring opening hydrogenation of the complex aromatics and asphaltenes, however minimal hydrocracking of hydrocarbons should take place.

The process conditions of hydrogen partial pressure, reaction pressure, temperature and residence time as measured liquid hourly velocity are optimized to achieve desired final product quality. A more detailed discussion of the Reactor System, the catalyst, the process conditions, and other aspects of the process are contained below in the "Reactor System Description."

The Reactor System Effluent (E) exits the Reactor System (11) via line (11a) and exchanges heat against the pressurized and partially heats the Feedstock HMFO (A') in the Reactor Feed/Effluent Exchanger (7). The partially cooled Reactor System Effluent (E') then flows via line (11c) to the Hot Separator (13).

The Hot Separator (13) separates the gaseous components of the Reactor System Effluent (F) which are directed to line (13a) from the liquid components of the Reactor System effluent (G) which are directed to line (13b). The gaseous components of the Reactor System effluent in line (13a) are cooled against air in the Hot Separator Vapor Air Cooler (15) and then flow via line (15a) to the Cold Separator (17).

The Cold Separator (17) further separates any remaining gaseous components from the liquid components in the cooled gaseous components of the Reactor System Effluent (F'). The gaseous components from the Cold Separator (F'') are directed to line (17a) and fed onto the Amine Absorber (21). The Cold Separator (17) also separates any remaining Cold Separator hydrocarbon liquids (H) in line (17b) from any Cold Separator condensed liquid water (I). The Cold Separator condensed liquid water (I) is sent OSBL via line (17c) for treatment.

The hydrocarbon liquid components of the Reactor System effluent from the Hot Separator (G) in line (13b) and the Cold Separator hydrocarbon liquids (H) in line (17b) are combined and are fed to the Oil Product Stripper System (19). The Oil Product Stripper System (19) removes any residual hydrogen and hydrogen sulfide from the Product HMFO (B) which is discharged in line (19B) to storage OSBL. We also assume a second draw (not shown) may be included to withdraw a distillate product, preferably a middle to heavy distillate. The vent stream (M) from the Oil Product Stripper in line (19A) may be sent to the fuel gas system or to the flare system that are OSBL. A more detailed discussion of the Oil Product Stripper System is contained in the "Oil Product Stripper System Description."

The gaseous components from the Cold Separator (F'') in line (17a) contain a mixture of hydrogen, hydrogen sulfide and light hydrocarbons (mostly methane and ethane). This vapor stream (17a) feeds an Amine Absorber System (21)

where it is contacted against Lean Amine (J) provided OSBL via line (21a) to the Amine Absorber System (21) to remove hydrogen sulfide from the gases making up the Activating Gas recycle stream (C'). Rich amine (K) which has absorbed hydrogen sulfide exits the bottom of the Amine Absorber System (21) and is sent OSBL via line (21b) for amine regeneration and sulfur recovery.

The Amine Absorber System overhead vapor in line (21c) is preferably recycled to the process as a Recycle Activating Gas (C') via the Recycle Compressor (23) and line (23 a) where it is mixed with the Makeup Activating Gas (C") provided OSBL by line (23b). This mixture of Recycle Activating Gas (C') and Makeup Activating Gas (C") to form the Activating Gas (C) utilized in the process via line (23c) as noted above. A Scrubbed Purge Gas stream (H) is taken from the Amine Absorber System overhead vapor line (21c) and sent via line (21d) to OSBL to prevent the buildup of light hydrocarbons or other non-condensable hydrocarbons. A more detailed discussion of the Amine Absorber System is contained in the "Amine Absorber System Description."

#### Reactor System Description:

The Core Process Reactor System (11) illustrated in FIG. 2 comprises a single reactor vessel loaded with the process catalyst and sufficient controls, valves and sensors as one of skill in the art would readily appreciate. One of skill in the art will appreciate that the reactor vessel itself must be engineered to withstand the pressures, temperatures and other conditions (i.e. presence of hydrogen and hydrogen sulfide) of the process. Using special alloys of stainless steel and other materials typical of such a unit are within the skill of one in the art and well known. As illustrated, fixed bed reactors are preferred as these are easier to operate and maintain, however other reactor types are also within the scope of the invention.

A description of the process catalyst, the selection of the process catalyst and the loading and grading of the catalyst within the reactor vessel is contained in the "Catalyst in Reactor System".

Alternative configurations for the Core Process Reactor System (11) are contemplated. In one illustrative configuration, more than one reactor vessel may be utilized in parallel as shown in FIG. 3 to replace the Core Process Reactor System (11) illustrated in FIG. 2.

In the embodiment in FIG. 3, each reactor vessel is loaded with process catalyst in a similar manner and each reactor vessel in the Reactor System is provided the heated Feed Mixture (D') via a common line (9B). The effluent from each reactor vessel in the Reactor System is recombined and forms a combined Reactor Effluent (E) for further processing as described above via line (11a). The illustrated arrangement will allow the three reactors to carry out the process effectively multiplying the hydraulic capacity of the overall Reactor System. Control valves and isolation valves may also prevent feed from entering one reactor vessel but not another reactor vessel. In this way one reactor can be by-passed and placed off-line for maintenance and reloading of catalyst while the remaining reactors continues to receive heated Feedstock Mixture (D'). It will be appreciated by one of skill in the art this arrangement of reactor vessels in parallel is not limited in number to three, but multiple additional reactor vessels can be added as shown by dashed line reactor. The only limitation to the number of parallel reactor vessels is plot spacing and the ability to provide heated Feedstock Mixture (D') to each active reactor.

A cascading series in FIG. 4 can also be substituted for the single reactor vessel Reactor System (11) in FIG. 2. The cascading reactor vessels are loaded with process catalyst

with the same or different activities toward metals, sulfur or other environmental contaminates to be removed. For example, one reactor may be loaded with a highly active demetallization catalyst, a second subsequent or downstream reactor may be loaded with a balanced demetallization/desulfurizing catalyst, and reactor downstream from the second reactor may be loaded with a highly active desulfurization catalyst. This allows for greater control and balance in process conditions (temperature, pressure, space flow velocity, etc. . . .) so it is tailored for each catalyst. In this way one can optimize the parameters in each reactor depending upon the material being fed to that specific reactor/catalyst combination and minimize the hydrocracking reactions.

An alternative implementation of the parallel reactor concept is illustrated in greater detail in FIG. 5. Heated Feed Mixture (D') is provided to the reactor System via line (9B) and is distributed amongst multiple reactor vessels (11, 12a, 12b, 12c and 12d). Flow of heated Feedstock to each reactor vessel is controlled by reactor inlet valves (60, 60a, 60b, 60c, and 60d) associated with each reactor vessel respectively. Reactor Effluent (E) from each reactor vessel is controlled by a reactor outlet valve (62, 62a, 62b, 62c and 62d) respectively. Line (9B) has multiple inflow diversion control valves (68, 68a, 68b and 68c), the function and role of which will be described below. Line (11a) connects the outlet of each reactor, and like Line (9B) has multiple outflow diversion control valves (70, 70a, 70b and 70c) the function and role of which will be described below. Also shown is a by-pass line defined by lower by-pass control valve (64, 64a, 64b, 64c) and upper by-pass control valve (66, 66a, 66b and 66c), between line (9B) and line (11a) the function and purpose of which will be described below. One of skill in the art will appreciate that control over the multiple valves and flow can be achieved using a computerized control system/distributed control system (DCS) or programmable logic controllers (PLC) programed to work with automatic motorized valve controls, position sensors, flow meters, thermocouples, etc. . . . These systems are commercially available from vendors such as Honeywell International, Schneider Electric; and ABB. Such control systems will include lock-outs and other process safety control systems to prevent opening of valves in manner either not productive or unsafe.

One of skill in the art upon careful review of the illustrated configuration will appreciate that multiple flow schemes and configurations can be achieved with the illustrated arrangement of reactor vessels, control valves and interconnected lines forming the reactor System. For example, in one configuration one can: open all of inflow diversion control valves (68, 68a, 68b and 68c); open the reactor inlet valves (60, 60a, 60b, 60c, and 60d); open the reactor outlet valves (62, 62a, 62b, 62c and 62d); open the outflow diversion control valves (70, 70a, 70b and 70c); and close lower by-pass control valve (64, 64a, 64b, 64c) and upper by-pass control valve (66, 66a, 66b and 66c), to substantially achieve a reactor configuration of five parallel reactors each receiving heated Feed Mixture (D') from line (9B) and discharging Reactor Effluent (E) into line (11a). In such a configuration, the reactors are loaded with catalyst in substantially the same manner. One of skill in the art will also appreciate that closing of an individual reactor inlet valve and corresponding reactor outlet valve (for example closing reactor inlet vale 60 and closing reactor outlet valve 62) effectively isolates the reactor vessel (11). This will allow for the isolated reactor vessel (11) to be brought off

line and serviced and or reloaded with catalyst while the remaining reactors continue to transform Feedstock HMFO into Product HMFO.

A second illustrative configuration of the control valves allows for the reactors to work in series as shown in FIG. 5 by using the by-pass lines. In such an illustrative embodiment, inflow diversion control valve (68) is closed and reactor inlet valve (60) is open. Reactor (11) is loaded with demetallization catalyst and the effluent from the reactor exits via open outlet control valve (62). Closing outflow diversion control valve (70), the opening of lower by-pass control valve (64) and upper by-pass control valve (66), the opening of reactor inlet valve (60a) and closing of inflow diversion control valve (68a) re-routes the effluent from reactor (11) to become the feed for reactor (12a). reactor (12a) may be loaded with additional demetallization catalyst, or a transition catalyst loading or a desulfurization catalyst loading. One of skill in the art will quickly realize and appreciate this configuration can be extended to the other reactors (12b, 12c and 12d) allowing for a wide range of flow configurations and flow patterns through the Reactor Section. An advantage of this illustrative embodiment of the Reactor Section is that it allows for any one reactor to be taken off-line, serviced and brought back on line without disrupting the transformation of Feedstock HMFO to Product HMFO. It will also allow a plant to adjust the configuration so that as the composition of the feedstock HMFO changes, the reactor configuration (number of stages) and catalyst types can be adjusted. For example a high metal containing Feedstock HMFO, such as a Ural residual based HMFO, may require two or three reactors (i.e. reactors 11, 12a and 12b) loaded with demetallization catalyst and working in series while reactor 12c is loaded with transition catalyst and reactor 12d is loaded with desulfurization catalyst. Many permutations and variations can be achieved by opening and closing control valves as needed and adjusting the catalyst loadings in each of the reactor vessels by one of skill in the art and only for brevity need not be described. One of skill in the art will appreciate that control over the multiple valves and flow can be achieved using a computerized control system/distributed control system (DCS) or programmable logic controllers (PLC) programmed to work with automatic motorized valve controls, position sensors, flow meters, thermocouples, etc. . . . These systems are commercially available from vendors such as Honeywell International, Schneider Electric; and ABB. Such control systems will include lock-outs and other process safety control systems to prevent opening of valves in manner either not productive or unsafe.

Another illustrative embodiment of the replacement of the single reactor vessel Reactor System 11 in FIG. 2 is a matrix of reactors composed of interconnected reactors in parallel and in series. A simple 2x2 matrix arrangement of reactors with associated control valves and piping is shown in FIG. 6, however a wide variety of matrix configurations such as 2x3; 3x3, etc. . . are contemplated and within the scope of the present invention. As depicted in FIG. 6, a 2 reactor by 2 reactor (2x2) matrix of comprises four reactor vessels (11, 12a, 14 and 14b) each with reactor inlet control valves (60, 60a, 76, and 76a) and reactor outlet control valves (62, 62a, 78 and 78a) associated with each vessel. Horizontal flow control valves (68, 68a, 70, 70a, 70b, 74, 74a, 74b, 80, 80a, and 80b) regulate the flow across the matrix from heated Feedstock (D') in line 9B to discharging Reactor Effluent (E) into line 11a. Vertical flow control valves (64, 64a, 66, 66a, 72, 72a, 72b, 72c, 82, 82a, 84, and 84b) control the flow through the matrix from line 9B to line 11a. One of skill in

the art will appreciate that control over the multiple valves and flow can be achieved using a computerized control system/distributed control system (DCS) or programmable logic controllers (PLC) programmed to work with automatic motorized valve controls, position sensors, flow meters, thermocouples, etc. . . . These systems are commercially available from vendors such as Honeywell International, Schneider Electric; and ABB. Such control systems will include lock-outs and other process safety control systems to prevent opening of valves in manner either not productive or unsafe.

One of skill in the art will quickly realize and appreciate that by opening and closing the valves and varying the catalyst loads present in each reactor, many configurations may be achieved. One such configuration would be to open valves numbered: 60, 62, 72, 76, 78, 80, 82, 84, 72a, 64, 66, 68a, 60a, 62a, 72b, 76a, 78a, and 80b, with all other valves closed so the flow for heated Feed Mixture (D') will pass through reactors 11, 14, 12a and 14a in series. Another such configuration would be to open valves numbered: 60, 62, 70, 64, 66, 68a, 60a, 62a, 72b, 76a, 78a, and 80b, with all other valves closed so the flow of heated Feed Mixture (D') will pass through reactors 11, 12a and 14a (but not 14). As with the prior example, the nature of the Feedstock HSFO and the catalyst loaded in each reactor may be optimized and adjusted to achieve the desired Product HSFO properties, however for brevity of disclosure all such variations will be apparent to one of skill in the art.

One benefit of having a multi-reactor Reactor System is that it allows for a reactor experiencing decreased activity or plugging because of coke formation can be isolated and taken off line for turn-around (i.e. deactivated, catalyst and internals replaced, etc. . . ) without the entire plant having to shut down. Another benefit as noted above is that it allows one to vary the catalyst loading in the Reactor System so the overall process can be optimized for a specific Feedstock HSFO. A further benefit is that one can design the piping, pumps, heaters/heat exchangers, etc. . . to have excess capacity so that when an increase in capacity is desired, additional reactors can be quickly brought on-line. Conversely, it allows an operator to take capacity off line, or turn down a plant output without having a concern about turn down and minimum flow through a reactor. While the above matrix Reactor System is described referring to a fixed bed or packed bed trickle flow reactor, one of skill in the art will appreciate that other reactor types may be utilized. For example, one or more reactors may be configured to be ebullated bed up flow reactors or three phase upflow bubble reactors, or counter-current reactors, or reactive distillation reactors the configuration of which will be known to one of skill in the art. It is anticipated that many other operational and logistical benefits will be realized by one of skill in the art from the Reactor Systems configurations disclosed.

#### Catalyst in Reactor System:

The reactor vessel in each Reactor System is loaded with one or more process catalysts. The exact design of the process catalyst system is a function of feedstock properties, product requirements and operating constraints and optimization of the process catalyst can be carried out by routine trial and error by one of ordinary skill in the art.

The process catalyst(s) comprise at least one metal selected from the group consisting of the metals each belonging to the groups 6, 8, 9 and 10 of the Periodic Table, and more preferably a mixed transition metal catalyst such as Ni—Mo, Co—Mo, Ni—W or Ni—Co—Mo are utilized. The metal is preferably supported on a porous inorganic oxide catalyst carrier. The porous inorganic oxide catalyst

carrier is at least one carrier selected from the group consisting of alumina, alumina/boria carrier, a carrier containing metal-containing aluminosilicate, alumina/phosphorus carrier, alumina/alkaline earth metal compound carrier, alumina/titania carrier and alumina/zirconia carrier. The preferred porous inorganic oxide catalyst carrier is alumina. The pore size and metal loadings on the carrier may be systematically varied and tested with the desired feedstock and process conditions to optimize the properties of the Product HMFO. One of skill in the art knows that demetallization using a transition metal catalyst (such a CoMo or NiMo) is favored by catalysts with a relatively large surface pore diameter and desulfurization is favored by supports having a relatively small pore diameter. Generally the surface area for the catalyst material ranges from 200-300 m<sup>2</sup>/g. The systematic adjustment of pore size and surface area, and transition metal loadings activities to preferentially form a demetallization catalyst or a desulfurization catalyst are well known and routine to one of skill in the art. Catalyst in the fixed bed reactor(s) may be dense-loaded or sock-loaded and including inert materials (such as glass or ceric balls) may be needed to ensure the desired porosity.

The catalyst selection utilized within and for loading the Reactor System may be preferential to desulfurization by designing a catalyst loading scheme that results in the Feedstock mixture first contacting a catalyst bed that with a catalyst preferential to demetallization followed downstream by a bed of catalyst with mixed activity for demetallization and desulfurization followed downstream by a catalyst bed with high desulfurization activity. In effect the first bed with high demetallization activity acts as a guard bed for the desulfurization bed.

The objective of the Reactor System is to treat the Feedstock HMFO at the severity required to meet the Product HMFO specification. Demetallization, denitrogenation and hydrocarbon hydrogenation reactions may also occur to some extent when the process conditions are optimized so the performance of the Reactor System achieves the required level of desulfurization. Hydrocracking is preferably minimized to reduce the volume of hydrocarbons formed as by-product hydrocarbons to the process. The objective of the process is to selectively remove the environmental contaminants from Feedstock HMFO and minimize the formation of unnecessary by-product hydrocarbons (C<sub>1</sub>-C<sub>8</sub> hydrocarbons).

The process conditions in each reactor vessel will depend upon the feedstock, the catalyst utilized and the desired properties of the Product HMFO. Variations in conditions are to be expected by one of ordinary skill in the art and these may be determined by pilot plant testing and systematic optimization of the process. With this in mind it has been found that the operating pressure, the indicated operating temperature, the ratio of the Activating Gas to Feedstock HMFO, the partial pressure of hydrogen in the Activating Gas and the space velocity all are important parameters to consider. The operating pressure of the Reactor System should be in the range of 250 psig and 3000 psig, preferably between 1000 psig and 2500 psig and more preferably between 1500 psig and 2200 psig. The indicated operating temperature of the Reactor System should be 500° F. to 900° F., preferably between 650° F. and 850° F. and more preferably between 680° F. and 800° F. The ratio of the quantity of the Activating Gas to the quantity of Feedstock HMFO should be in the range of 250 scf gas/bbl of Feedstock HMFO to 10,000 scf gas/bbl of Feedstock HMFO, preferably between 2000 scf gas/bbl of Feedstock HMFO to 5000 scf gas/bbl of Feedstock HMFO and more preferably

between 2500 scf gas/bbl of Feedstock HMFO to 4500 scf gas/bbl of Feedstock HMFO. The Activating Gas should be selected from mixtures of nitrogen, hydrogen, carbon dioxide, gaseous water, and methane, so Activating Gas has an ideal gas partial pressure of hydrogen (p<sub>H2</sub>) greater than 80% of the total pressure of the Activating Gas mixture (P) and preferably wherein the Activating Gas has an ideal gas partial pressure of hydrogen (p<sub>H2</sub>) greater than 90% of the total pressure of the Activating Gas mixture (P). The Activating Gas may have a hydrogen mole fraction in the range between 80% of the total moles of Activating Gas mixture and more preferably wherein the Activating Gas has a hydrogen mole fraction between 80% and 90% of the total moles of Activating Gas mixture. The liquid hourly space velocity within the Reactor System should be between 0.05 oil/hour/m<sup>3</sup> catalyst and 1.0 oil/hour/m<sup>3</sup> catalyst; preferably between 0.08 oil/hour/m<sup>3</sup> catalyst and 0.5 oil/hour/m<sup>3</sup> catalyst and more preferably between 0.1 oil/hour/m<sup>3</sup> catalyst and 0.3 oil/hour/m<sup>3</sup> catalyst to achieve deep desulfurization with product sulfur levels below 0.1 ppmw.

The hydraulic capacity rate of the Reactor System should be between 100 bbl of Feedstock HMFO/day and 100,000 bbl of Feedstock HMFO/day, preferably between 1000 bbl of Feedstock HMFO/day and 60,000 bbl of Feedstock HMFO/day, more preferably between 5,000 bbl of Feedstock HMFO/day and 45,000 bbl of Feedstock HMFO/day, and even more preferably between 10,000 bbl of Feedstock HMFO/day and 30,000 bbl of Feedstock HMFO/day. The desired hydraulic capacity may be achieved in a single reactor vessel Reactor System or in a multiple reactor vessel Reactor System as described.

#### Oil Product Stripper System Description:

The Oil Product Stripper System (19) comprises a stripper column (also known as a distillation column or exchange column) and ancillary equipment including internal elements and utilities required to remove hydrogen, hydrogen sulfide and hydrocarbons lighter than diesel from the Product HMFO. Such systems are well known to one of skill in the art, see U.S. Pat. Nos. 6,640,161; 5,709,780; 5,755,933; 4,186,159; 3,314,879; 3,844,898; 4,681,661; or U.S. Pat. No. 3,619,377 the contents of which are incorporated herein by reference, a generalized functional description is provided herein. Liquid from the Hot Separator (13) and Cold Separator (7) feed the Oil Product Stripper Column (19). Stripping of hydrogen and hydrogen sulfide and hydrocarbons lighter than diesel may be achieved via a reboiler, live steam or other stripping medium. The Oil Product Stripper System (19) may be designed with an overhead system comprising an overhead condenser, reflux drum and reflux pump or it may be designed without an overhead system. The conditions of the Oil Product Stripper may be optimized to control the bulk properties of the Product HMFO, more specifically viscosity and density. We also assume a second draw (not shown) may be included to withdraw a distillate product, preferably a middle to heavy distillate.

#### Amine Absorber System Description:

The Amine Absorber System (21) comprises a gas liquid contacting column and ancillary equipment and utilities required to remove sour gas (i.e. hydrogen sulfide) from the Cold Separator vapor feed so the resulting scrubbed gas can be recycled and used as Activating Gas. Because such systems are well known to one of skill in the art, see U.S. Pat. Nos. 4,425,317; 4,085,199; 4,080,424; 4,001,386; which are incorporated herein by reference, a generalized functional description is provided herein. Vapors from the Cold Separator (17) feed the contacting column/system (19). Lean Amine (or other suitable sour gas stripping fluids or

systems) provided from OSBL is utilized to scrub the Cold Separator vapor so hydrogen sulfide is effectively removed. The Amine Absorber System (19) may be designed with a gas drying system to remove the any water vapor entrained into the Recycle Activating Gas (C'). The absorbed hydrogen sulfide is processed using conventional means OSBL in a tail gas treating unit, such as a Claus combustion sulfur recovery unit or sulfur recovery system that generates sulfuric acid.

Distressed Fuel Oil Materials Pre-Treatment Unit:

It will be appreciated by one of skill in the art, that the conditions utilized in the Core Process have been intentionally selected to minimize cracking of hydrocarbons and remove significant levels of sulfur by taking advantage of the properties of the Feedstock HMFO. However, one of skill in the art will also appreciate there are number of Distressed Fuel Oil Materials (DFOM) that alone or in combination may be pre-treated to provide a suitable Feedstock HMFO. The economic advantages of this will be apparent; low cost Distressed Fuel Oil Materials (DFOM), (i.e. materials that do not meet the ISO 8217 standards for a residual marine fuel oil and are sold at a substantial discount) may be pre-treated and then utilized as Feedstock HMFO in the Core Process to produce high value Product HMFO. Examples of DFOM include, but are not limited to: heavy hydrocarbons such as atmospheric residue; vacuum residue; FCC slurry oil; black oil, crude oils such as heavy crude oil, distressed crude oil, slop oils, de-asphalted oil (DAO), heavy coker oil, visbreaker bottoms, bitumen tars, and the like; non-merchantable residual fuel oils contaminated with high levels of solids, water, resins, acrylic or styrene oligomers, cumene, phenols, or other materials that make the Fuel Oil non-merchantable; DFOM also include off specification or distressed marine distillate and blends of marine distillate with residual high sulfur fuel oils that are not ISO 8217 compliant. An example of such a material would be a distillate/heavy marine fuel oil blend that has a 4 or 5 rating on ASTM D4740 compatibility tests. DFOM in and of themselves are not ISO 8217 compliant materials and are not merchantable as a residual ISO 8217 compliant Heavy Marine Fuel Oil or as a substitute for Heavy Marine Fuel Oil and sold at a considerable discount to the compliant materials.

The generalized purpose for the DFOM Pre-Treatment Unit is to condition or treat the DFOM so they may be utilized as a feedstock HMFO in the Core Process. This conditioning or treatment of the DFOM may involve treatment conditions including, but not limited to: blending DFOM with distillates or heavy gas oil; blending DFOM with HMFO; blending DFOM with other DFOM's together; and then optionally the subjecting the DFOM or DFOM blended material to additional treatment conditions such as: exposure to selective absorption materials; ultrafiltration; centrifugation; microwaves; ultrasound; gravity separation; gas purging (scrubbing) with nitrogen or other inert gases; ionic liquid extraction; extraction or washing the DFOM or DFOM blended material with water (with or without surfactants present); washing or counter-current extraction with non-miscible polar fluids such as acetonitrile, ethylene glycol, diethylene glycol, 2-aminoethanol, benzyl alcohol, ethylacetacetates or other materials having a relative polarity greater than 0.6 on a scale where water has a polarity of 1.0 or a polarity index greater than about 5.5; super critical fluids such as supercritical CO<sub>2</sub> or supercritical water may also be utilized as extraction medium under conditions well known in the art; subjecting the DFOM or DFOM blended material to vacuum; subjecting the DFOM or DFOM blended material to heat sufficient to volatilize components

having a boiling point below 350° F. (177° C.) at standard pressure, preferably below 400° F. (205° C.) at standard pressure and more preferably below 500° F. (260° C.), and optionally heating to those same temperatures under vacuum. Sometimes it may be desirable to blend the DFOM with a co-solvent or co-volatilizing material to enhance the volatilization of the certain components over other components. Such co-solvents or co-volatilizing materials will have a boiling point preferably the same as or form an azeotrope with the components to be removed from the DFOM in the pre-treatment step. When the DFOM or DFOM blended material and other materials are heated this preferably will occur under conditions of controlled distillation so the volatilized materials can be selectively separated by boiling point, condensed and withdrawn so they may be reused or sent to other parts of the refinery for commercialization. The above functional description of the DFOM Pre-Treatment Unit has been sufficiently disclosed to one of skill in the art, this additional description provides information that will be helpful to one of skill in the art by providing more specific illustrative embodiments.

Blending Pre-Treatment Unit:

One illustrative embodiment of a pre-treatment process involves the blending of the DFOM with a Blending Agent. The blending of DFOM with a Blending Agent will address deficiencies such as pour point, density, viscosity, CCAI (calculated carbon aromaticity index) excessive metals content, high levels of nitrogen or high solids content. As used herein, a Blending Agent will preferably be a hydrocarbon such as gas oil, FCC slurry oil, gas oil, diesel, middle distillate or heavy distillate cuts, cutter oil, condensable hydrocarbons generated in the Core Process, heavy or middle coker oils, and mixtures of these that serve as a diluent to the DFOM. Surfactants or other supplemental blending agents may be needed to ensure a uniform and rapid blending of the DFOM with the Blending Agent, but adding surfactants is not preferred. The functional role of the Blending Agent is to adjust the properties by dilution of the DFOM so the DFOM becomes ISO 8217 compliant feedstock HMFO suitable for the Core Process. It will be appreciated by one of skill in the art that the ratio or relative proportions of DFOM to Blending Agent will be dependent not only on the nature and properties of the DFOM, but also those of the selected Blending Agent. For example a simple reduction in viscosity may be achieved by mixing DFOM with a middle or heavy distillate fraction such as cutter oil. Similarly, the density of the DFOM may be adjusted by blending the DFOM with a small portion of diesel or recycled middle or heavy distillate materials produced in the Core Process. It will be a simple matter of adjusting the ratios of materials being blended to achieve the desired properties of the Feedstock HMFO.

An example of a Blending Pre-Treatment Unit is schematically illustrated in FIG. 7. A blending vessel (100) equipped with a means for blending such as simple paddle mixer shown (102) or orifice mixers or screw type mixers may mix the DFOM (P) provided via line (104) and Blending Agent (Q) via line (106). Sometimes it will be desirable to heat the DFOM prior to blending a heat exchanger (108) may be needed to provide heat to the DFOM prior to introduction into the blending vessel (100). In certain instances heating of the blending vessel (100) may be needed and such heat will be provided via heating elements (not shown) in the blending vessel (100). These may be steam heating element or electrical heating elements or other commonly used heating elements known to one of skill in the art. During the blending process, gases or other volatile

non-residual components (F) may evolve; in such instances vent line (110) will direct those gases or other volatile non-residual components (F) for processing elsewhere in the facility. The resulting blended material removed from the blending vessel via off-take line (112) will preferably be a compliant Feedstock HMFO (A) ready to be sent to the Core Process via pump (114) and line (116). However sometimes, some post blending physical treatment may be advantageous, such a dewatering, centrifugation or filtering to remove solids such as FCC catalytic fines, or shearing in a high speed mixer. In FIG. 7, a post blending treatment of centrifugation is illustrated with the blended material being pumped to a centrifuge (118) to remove solids (not shown) prior to being sent as Feedstock HMFO (A) to the Core Process via line (120). While the above Blending Pre-Treatment Unit is illustrated as a stirred tank blending process, one of skill in the art of hydrocarbon blending will appreciate that an in-line blending unit may also replace the blending tank shown and achieve substantially the same result. Variations such as this are contemplated as within the present invention as they achieve the overall goal of blending the DFOM with a Blending Agent to provide an ISO 8217 compliant Feedstock HMFO for the Core Process.

#### Stripper Pre-Treatment Unit:

In one illustrative embodiment of the Pre-Treatment Unit in FIG. 8, a packed column stripper is utilized to process the DFOM into Feedstock HMFO for the Core Process. The stripping of the DFOM will correct deficiencies such as too low flash point (i.e. an excessive amount of high flammability hydrocarbons), high content of H<sub>2</sub>S or high content of water. The illustrative packed column stripper has stripper vessel (200) containing multiple packed beds (202) of packing material supported on porous trays of a conventional type. The packed bed may be continuous, or it may be divided into segments as shown the purpose of which will be described below. DFOM (P) will be introduced into the stripper via DFOM feed line (204) and distributor tray (206) or manifold to ensure an appropriate distribution across the stripper column. Stripping agent (S) will be introduced into the bottom of the stripper via the stripper feed line (208) and is distributed across the vessel with a distribution tray (210) or manifold to maximize the effect of the stripping agent. Because of the residual properties of the DFOM being stripped, auxiliary or interbed injection of stripper agent will likely be needed and desired. This is achieved by auxiliary stripper inlet line (212) which injects the stripping agent via distribution manifolds or trays or injectors at breaks or gaps in the packed bed. The Feedstock HMFO (A) exits the bottom of the stripper via line (214) and is routed to the Core Process. The non-residual components of the DFOM are stripped from the DFOM and exit the top of the stripper column with the stripping agent via line (216). The stripper agent and non-residual components of the DFOM are passed through a heat exchanger (218) and then sent to knockdown drum (220) so the stripper gas and more volatile materials can be separated from the more condensable components stripped from the DFOM. In certain instances, as shown in FIG. 8, it will be desirable to withdraw a portion of the condensed components from the knockdown drum via line (222), pump (224) and reflux line (226) and reflux this material back into the stripper. This reflux loop however is optional. The non-condensed vapors and stripping agent (F) are vented from the knockdown drum (220) via line (228) and processed elsewhere in the plant. The condensable liquid materials (G) are removed via line (230) and process elsewhere in the plant. In at least one preferred embodiment, a downcomer/bubble cap tray (232) is inserted into the

stripper column at an appropriate location to create a side draw stream via line (234) of heavy to medium distillate materials (G'). This may be especially helpful when the DFOM is a blend made of MGO or marine diesel with residual components of the DFOM or containing distillate or residual streams containing volatile light components.

Steam, air, inert gases, and light hydrocarbon gases can be the stripping agent (S) to separate the residual components of the DFOM from the non-residual volatile components of the DFOM. Selection of the stripping agent (S) will depend upon solubility, stability, and availability as well as ability to remove the non-residual volatile components of the DFOM. Because the stripping agents (S) will be preferably gases, operation at nearly the highest temperature and lowest pressure that will maintain the components of the DFOM desired in the Feedstock HMFO and vaporize the volatile components in the DFOM feed stream is desired.

One of skill in the art will appreciate that strippers can be trayed or packed. Packed column strippers, as shown in FIG. 8, particularly when random packing is used, are usually favored when fluid velocity is high, and when particularly low pressure drop is desired. Trayed strippers are advantageous because of ease of design and scale up. Structured packing can be used similar to trays despite possibly being the same material as dumped (random) packing. Using structured packing is a common method to increase the capacity for separation or to replace damaged trays.

Trayed strippers can have sieve, valve, or bubble cap trays while packed strippers can have either structured packing or random packing. Trays and packing are used to increase the contact area over which mass transfer can occur as mass transfer theory dictates. Packing can have varying material, surface area, flow area, and associated pressure drop. Older generation packing include ceramic Raschig rings and Berl saddles. More common packing materials are metal and plastic Pall rings, metal and plastic Zbigniew Bialecki rings, and ceramic Intalox saddles. Each packing material improves the surface area, the flow area, and/or the associated pressure drop across the packing. Also important, is the ability of the packing material to not stack on top of itself. If such stacking occurs, it drastically reduces the surface area of the material.

During operation, monitoring the pressure drop across the column can help to determine the performance of the stripper. A changed pressure drop over a significant range of time can indicate that the packing may need to be replaced or cleaned.

#### Distillation Pre-Treatment Unit:

When the DFOM material has significant non-residual volatile materials, such as diesel, MGO or lighter materials, it may be economically advantageous to subject the DFOM to a distillation process so the non-residual volatile materials can be recovered. The distillation pre-treatment of the DFOM will also address deficiencies such as flash point, high content of H<sub>2</sub>S or water. FIG. 9 illustrates such an embodiment of the Pre-Treatment Unit in which distillation takes place. The distillation column (300) will have within it multiple internal distillation elements (302) such as the downcomer/bubble cap tray illustrated. The number of downcomer trays will depend upon how many theoretical plates are needed to achieve the desire level of purity and separation desired. The number of trays shown serves to merely illustrate the concept and one of skill in the art will be able engineering in much greater detail the placement, size, number and characteristics of the distillation elements. One can utilize packed bed distillation elements supported on trays, or other similar distillation elements well known to

one of skill in the art of distillation of hydrocarbons. Trays and packing are used to increase the contact area over which mass transfer can occur as mass transfer theory dictates. Packing can have varying material, surface area, flow area, and associated pressure drop. Older generation packing include ceramic Raschig rings and Berl saddles. More common packing materials are metal and plastic Pall rings, metal and plastic Zbigniew Bialecki rings, and ceramic Intalox saddles. The DFOM (P) is fed to the Pre-Treatment Unit via line (304) onto a distribution tray (306) or fluid distribution manifold to distribute DFOM feed across the distillation column. The residual components of the DFOM will travel down the column towards the lower end of the column while the more volatile components will travel up the column towards the upper end of the column. At the lower end of the column the Feedstock HMFO (A) will exit via line (308) and sent to the Core Process for transformation into low sulfur HMFO that is ISO 8217 compliant. A reboiler loop or bottoms reflux loop (310) with recirculation pump (312) may be desirable to ensure the Feedstock HMFO exiting the lower portion of the distillation Pre-Treatment Unit are maintained within the desired window of acceptable properties. So heat may be added to the column, a heater (not shown) may optionally be added to the reboiler loop (310). In certain embodiments it may be desirable to introduce an optional stripping gas (S) via line (314) in which instances a distribution tray or manifold distributor (316) may also be needed to ensure a uniform introduction of the stripper gas into the distillation column. In the portion of the distillation column above the introduction point of the DFOM there will also be multiple distillation elements (302) shown in FIG. 9 as downcomer/bubble cap trays. A limited number are shown, but one of skill in the art will appreciate the number of downcomer trays will depend upon how many theoretical plates are needed to achieve the desire level of purity and separation desired. The number of trays shown serves to merely illustrate the concept and one of skill in the art will be able engineering in much greater detail the placement, size, number and characteristics of the distillation elements. One can utilized packed bed distillation elements supported on trays, or other similar distillation elements well known to one of skill in the art of distillation of hydrocarbons. The non-residual volatile components of the DFOM may exit the top of the distillation column via line (318). The non-residual volatile components of the DFOM are cooled in heat exchanger (320) and then sent to a knockdown drum (322) so that the condensed liquid portions can be separated from the vaporous components. One of skill in the art will appreciate that it will be desirable to utilize a portion of the condensed liquids as a reflux to the upper portion of the distillation column. In such instances, line (324) will withdraw a portion of the condensed liquids in knockdown drum (322) and return them to the distillation column via pump (325) and upper reflux line (326). The vapors (F) in the knockdown drum (322) are vented via line (328) so they will be combined and co-processed with the vapors generated in the Core Process. Similarly excess condensed liquids (G) accumulated in knockdown drum (322) can be removed via line (330) and combined and co-processed with the similar condensable hydrocarbons generated in the Core Process. One of skill in the art of distillation column design and engineering will appreciate that the distillation elements also present the opportunity to remove non-residual fractions from the distillation column. For example, middle distillate fractions (G') may be removed with off-take line (332). Other heavier non-residual fractions may also be recovered in a similar manner with

off-take lines located in the appropriate section of the distillation column. In this way the distillation Pre-Treatment Unit achieves not only the production of Feedstock HMFO for the Core Process, but also recover valuable distillate components of the DFOM such as gas oil, middle distillates, heavy distillates and the like.

One of skill in the art will appreciate that in certain embodiments it may be desirable to incorporate catalytic materials within the internal structures of the Distillation Pre-Treatment Unit. A description of suitable structured catalyst beds is below.

#### Structured Catalyst Bed

Turning now to the structured catalyst bed, similar beds have been disclosed in the prior art in reactive distillation configurations involving catalyst promoted reactions. See for example U.S. Pat. Nos. 4,731,229; 5,073,236; 5,266,546; 5,431,890; 5,730,843; USUS2002068026; US20020038066; US20020068026; US20030012711; US20060065578; US20070209966; US20090188837; US2010063334; US2010228063; US20110214979; US20120048778; US20150166908; US20150275105; 20160074824; 20170101592 and US20170226433, the contents of which are incorporated herein by reference. However these disclosures involve the product being distilled from heavier bottoms or feedstock materials. For example heavy and light naphtha streams are desulfurized with the desired light naphtha being the desired product for the gasoline pool and the heavy naphtha either recycled or sent to an FCC cracker for further upgrading. The process of the invention utilized the distillation separation process to remove undesired by-product hydrocarbons and gases produced by the catalytic reaction (i.e. ammonia and hydrogen sulfide) and the desired product is the bottoms stream is catalytically treated, but not distilled. The structured catalyst beds as described above balance the catalyst density load, the catalyst activity load and the desired liquid space velocity through the reactor so an effective separation or distillation of purified lighter products can be produced. In contrast the present process functionally combines the functioning of a reactor with a stripper column or knock down drum. A further problem solved by the structured catalyst bed is to reduce the pressure drop through the catalyst beds and provision of sufficient contact of the Distressed Fuel Oil Materials with the catalyst and mixing with an Activating Gas.

A first illustrative embodiment of the structured catalyst beds is shown in FIG. 10 and FIG. 11 in a side view. As illustrated in FIG. 10 is a catalyst retention structure (400) composed of a pair of fluid permeable corrugated metal sheets (402 and 404), wherein the pair of the fluid permeable corrugated metal sheets are aligned so the corrugations are sinusoidal, have the same wave length and amplitude, but are out of phase and defining a catalyst rich space (406) and a catalyst lean space (408). The catalyst rich space will be loaded with one or more catalyst materials and optionally inert packing materials. The catalyst lean space (408) may be left empty or it may be loaded with inert packing such as ceramic beads, inactive (non-metal containing) catalyst support, glass beads, rings, wire or plastic balls and the like. These inert packing materials may serve the role of assisting in the mixing of an Activating Gas with the DFOM, facilitate the removal or separation of gaseous by products (i.e. hydrogen sulfide or ammonia) from the process mixture or facilitate the separation of any hydrocarbon by-products.

FIG. 11 shows in side perspective a plurality of catalyst retention structures (410, 412 and 414) formed into a structured catalyst bed (416). Structural supports (418) may be

optionally incorporated into the structured catalyst bed to lend rigidity as needed. As shown the catalyst rich spaces are radially aligned so the catalyst rich spaces of one catalyst retention structure is aligned with the catalyst rich structure of the adjacent layers. In the illustrated configuration, the radial angle between adjacent layers is 0° (or 180°). One of skill in the art will appreciate that the angle of radial alignment between adjacent layers may be varied from 0° to 180°, preferably between 20° and 160° and more preferably 90° so the catalyst rich areas in one layer are perpendicular to the adjacent layers. It will be further appreciated that the alignment of a particular set of three or more layers need not be the same. A first layer may be aligned along and define the 0° axis relative to the other two layers; a second adjacent layer may be radially aligned along a 45° angle relative to the first layer; and the third layer aligned along a 90° angle relative to the first layer. This pattern of alignment may be continued until the desired number of layers is achieved. It also should be appreciated that it may be desirable to angle of the catalyst rich spaces (i.e. the plane of the catalyst retention structure), relative to the flow of DFOM and Activating Gas within the structured catalyst beds. This relative angle is referred to herein as the inclination angle. As shown in FIG. 11, the inclination angle is perpendicular (90°) to the flow of DFOM and Activating Gas through the structured catalyst beds. However, it will be appreciated that the inclination level may be varied between 0°, in which case the catalyst rich spaces are vertically aligned with the flow of DFOM and 90° in which case the catalyst rich spaces are perpendicular to the flow of DFOM. By varying both the radial alignment and the inclination angle of the catalyst rich spaces, one can achieve a wide variety and be able to optimize the flow of DFOM through the structured catalyst bed with minimal plugging/coking.

A second illustrative embodiment of the structured catalyst beds is shown in FIG. 12 and FIG. 13 in a side view. As illustrated in FIG. 12, catalyst retention structure (420) comprises a flat fluid permeable metal sheet (422) and a corrugated fluid permeable metal sheet (424) aligned to be co-planar and defining a catalyst rich space (426) and a catalyst lean space (428). As with the prior illustrative embodiment, the catalyst rich space will contain one or more catalyst materials and optionally inert packing materials and the catalyst lean space will be empty or optionally contain inert packing materials. FIG. 13 shows in side perspective a plurality of catalyst retention structures (430, 432 and 434) formed into a structured catalyst bed (436). Structural supports (438) may be optionally incorporated into the structured catalyst bed to lend rigidity as needed. As shown the catalyst rich spaces are radially aligned so the catalyst rich spaces of one catalyst retention structure is perpendicular with the catalyst rich structure of the adjacent layers. In the illustrated configuration, the radial angle between adjacent layers is 90°. The same considerations of radial alignment and inclination of the catalyst retention structures described above will apply to this embodiment. The principle benefit of the illustrated structured catalyst bed is that the manufacturing process because affixing the flat fluid permeable sheet and the corrugated fluid permeable sheet will be greatly simplified. Further as illustrated, if the corrugated sheet is constructed using 90° angle corrugations, each catalyst retention structure can withstand much greater weight loadings than if the corrugations are sinusoidal.

The loading of the catalyst structures will depend upon the particle size of the catalyst materials and the activity level of the catalyst. The structures should be loaded so the open space will be at least 10 volume % of the overall

structural volume, and preferably will be up to about 65% of the overall structural volume. Active catalyst materials should be loaded in the catalyst support structure at a level dependent upon the catalyst activity level and the desired level of treatment. For example a catalyst material highly active for desulfurization may be loaded at a lower density than a less active desulfurization catalyst material and yet still achieve the same overall balance of catalyst activity per volume. One of skill in the art will appreciate that by systematically varying the catalyst loaded per volume and the catalyst activity level one may optimize the activity level and fluid permeability levels of the structured catalyst bed. In one such example, the catalyst density is so over 50% of the open space in the catalyst rich space, which may occupy only 1/2 of the over space within the structured catalyst bed. In another example catalyst rich space is loaded (i.e. dense packed into each catalyst rich space), however the catalyst rich space may occupy only 30 volume % of the overall structured catalyst bed. It will be appreciated that the catalyst density in the catalyst rich space may vary between 30 vol % and 100 vol % of the catalyst rich space. It will be further appreciated that that catalyst rich space may occupy as little as 10 vol % of the overall structured catalyst bed or it may occupy as much as 80 vol % of the overall structured catalyst bed.

The liquid hourly space velocity within the structured catalyst beds should be between 0.05 oil/hour/m<sup>3</sup> catalyst and 10.0 oil/hour/m<sup>3</sup> catalyst; preferably between 0.08 oil/hour/m<sup>3</sup> catalyst and 5.0 oil/hour/m<sup>3</sup> catalyst and more preferably between 0.1 oil/hour/m<sup>3</sup> catalyst and 3.0 oil/hour/m<sup>3</sup> catalyst to achieve deep desulfurization using a highly active desulfurization catalyst and this will achieve a product with sulfur levels below 0.1 ppmw. However, it will be appreciated by one of skill in the art that when there is lower catalyst density, it may be desirable to adjust the space velocity to value outside of the values disclosed.

One of skill in the art will appreciate that the above described structured catalyst beds can serve as a direct substitute for dense packed beds that include inert materials, such as glass beads and the like. An important criteria is the catalyst density within the beds themselves. The structured catalyst beds can be loaded with a catalyst density comparable to that of a dense loaded bed with a mixture of catalyst and inert materials or a bed with layers of catalyst and inert materials. Determining the optimized catalyst density will be a simple matter of systematically adjusting the catalyst density (for a set of reaction conditions) in a pilot plant. A fixed density catalyst structure will be made and the reaction parameters of space velocity and temperature and bed depth will be systematically varied and optimized.

#### Reactive Distillation Pre-Treatment Unit:

As illustrated in FIG. 14, a Reactive Distillation Pre-Treatment Unit as contemplated by the present invention may comprise a reactor vessel (500) within which one or more structured beds as described above will be provided (502, 504 and 506). One of skill in the art will note that heated DFOM (P) enters the reactor vessel in the upper portion of the reactor via line (501) above the structured catalyst beds (502, 504 and 506). When elements are the same as those disclosed, the same reference number is utilized for continuity within the disclosure. Entry of the heated DFOM above the structured catalyst beds (502, 504 and 506) may be facilitated by a distribution tray or similar device not shown. It will also be noted that each of the structured catalyst beds is different in appearance, the reason for this will now be described. The upper most structured catalyst bed (502) will be preferably loaded with a low

activity demetallization catalyst and in a structure optimized for the volatilization of the light hydrocarbons and middle distillate hydrocarbons present in DFOM mixture. The middle structured catalyst bed (504) will preferably be loaded with a higher activity demetallization and optionally inert materials or even a low activity desulfurization catalyst. The lower most structured catalyst bed will be preferably loaded with inert material and low activity desulfurization catalyst. A gas sparger or distribution tray or gas injection manifold (508) is below structured catalyst tray (506). In this way, the DFOM flows from the upper portion of the reactor to the lower portion of the reactor and will be transformed into Feedstock HMFO (A) which exits the bottom of the reactor via line (509).

As shown, an Activating Gas (C'') may be provided via line (514) to both quench and create within the reactor a counter-current flow of Activating Gas within the reactor vessel. One of skill in the art will appreciate this flow may also be connected to the reactor vessel so make up Activating Gas is also injected between structured catalyst beds (506) and (504) and (504) and (502). In the upper portion of the reactor vessel, inert distillation packing beds (510 and 512) may be located. It may be desirably and optionally it is preferable for the lower most of these upper beds (510) to be a structured catalyst bed as well with catalyst for the desulfurization of the distillate materials. In such an instance a down comber tray or similar liquid diversion tray (514) is inserted so a flow of middle to heavy distillate (G') can be removed from the upper portion of the reactor via line (526). Light hydrocarbons (i.e. lighter than middle distillate) exits the top of the reactor via line (516) and passes through heat exchanger (517) to help with heat recovery. This stream is then directed to the reflux drum (518) in which liquids are collected for use as reflux materials. The reflux loop to the upper reactor is completed via reflux pump (522) and reflux line (524). That portion of the lights not utilized in the reflux are combined with similar flows (F and G) via lines (13a) and (13b) respectively.

One of skill in the art of reactive distillation reactor design will note that unlike the prior art reactive distillation processes and reactor designs, the present invention presents multiple novel and non-obvious (i.e. inventive step) features. One such aspect, as noted above, the DFOM enters the upper portion of the reactor above the structured catalytic beds. In doing so it is transformed into Feedstock HMFO (A) that exits the bottom of the reactor. One of skill in the art will appreciate that by this flow, the majority of Feedstock HMFO material (which is characterized as being residual, that is having a boil point greater than 500° F. (260° C.) at standard pressure, preferably greater than 600° F. (315° C.) at standard pressure and more preferably greater than 650° F. (343° C.)) that is the primary product of this Pre-Treatment Unit will not be volatile or distilled, but any by product gases, contaminating materials, distillate hydrocarbons or light hydrocarbons are volatilized into the upper portion of the reactor. The reactor will be hydraulically designed so the majority of the volume of the liquid components having residual properties in the DFOM will exit the lower portion of the reactor, preferably over 75% vol. of the volume of the liquid components having residual properties in the DFOM will exit the lower portion of the reactor and even more preferably over 90% vol. of the volume of the liquid components having residual properties in the DFOM will exit the lower portion of the reactor. This is in contrast with the prior art reactive distillation processes where the majority of the desired products exit the upper portion of the

reactor via distillation and the residual bottoms portions are recycled or sent to another refinery unit for further processing.

In a variation of the above illustrative embodiment, one or 5 more fixed bed reactor(s) containing, solid particle filtering media such as inactive catalyst support, inert packing materials, selective absorption materials such as sulfur absorption media, demetallization catalyst or combinations and mixtures of these may be located upstream of the Reactive 10 Distillation Pre-Treatment Unit. In one embodiment, the upstream reactors are loaded within inert packing materials and deactivated catalyst to remove solids followed by a reactor loaded within absorptive desulfurization materials. One of skill in the art will appreciate these upstream reactors 15 may allow the upstream reactors to be taken out of service and catalysts changed out without shutting down or affecting operation of the Reactive Distillation Pre-Treatment Unit or the subsequent downstream Core Process.

In another variation of the above illustrative embodiment 20 in FIG. 14, a fired reboiler can be added to the lower portion of the reactive distillation reactor. Such a configuration would take a portion of the Feedstock HMFO (A) product material from the bottom of the reactor prior to its exit via line 509, pass it through a pump and optionally a heater, and 25 reintroduce the material into the reactor above tray (508) and preferably above the lowermost structured catalyst bed (506). The purpose of the reboiler will be to add or remove heat within the reactor, and increase column traffic; because of this reboiler loop a temperature profile in the reactor will 30 be controlled and more distillate product(s) may be taken. We assume severity in the column could be increased to increase the hydrocracking activity by including zeolitic materials in the structured catalyst beds within the Distillation Pre-Treatment Unit increasing the distillate production. 35 Because of the washing effect caused by refluxing Feedstock HMFO product back into the Distillation Pre-Treatment Unit, coking and fouling of catalysts should be minimized, allowing for extending run lengths.

#### Divided Wall Pre-Treatment Unit:

40 In a further alternative embodiment, a divided wall reactor or distillation column configuration may be desired, especially when heat preservation is desired, such as when feed heater capabilities are limited or when it is economical to combine feed pre-treatment and product post-treatment in a 45 single column.

Referring now to FIG. 15 FIG. 12, there is illustrated a Pre-Treatment Unit vessel (600) comprising an upper treatment section (602), first lower treatment section (604) and second lower treatment section (606). The treatment system 50 contains a longitudinally oriented partition (608) which extends through at least a part of the length of the vessel (602) to define the partitioned first lower treatment section (604) and the second lower treatment section (606).

As illustrate, DFOM (P) is provided into upper portion of 55 the first treatment section (604) through conduit means (610). Top vapor from the first treatment section comprising gases and light and middle distillate hydrocarbons will be withdrawn from the upper portion of the first lower treatment section (602). Middle distillate hydrocarbons are condensed in the upper portion of the treatment system (602) and optionally may be removed via line (611) as medium to heavy distillate (i.e. diesel and gas oil) for use and processing outside the battery limits shown. A portion of the middle distillate hydrocarbons can be diverted and used as a reflux 60 (not shown) if desired, the volume of that reflux may be minimal. The gases and light hydrocarbons collect at the top of the treatment system and exit the vessel via line (612) for 65

later processing which may occur outside of the battery limits. As illustrated the later processing may comprise a heat exchanger (614) followed by a separator drum (616). The condensed hydrocarbon liquids can be used in part as a reflux to the treatment section via pump (618) and lines (617 & 619). Or in addition, the light hydrocarbon liquids (wild naphtha) can be withdrawn via line (620) and processed using conventional techniques outside of the battery limits shown. Any sour water accumulating in the reflux drum can be withdrawn via line (621). Vapors and lighter hydrocarbons will be removed via vent (622) and processed outside the battery limits. The bottoms portion of the first lower treatment section (604), comprising partially treated DFOM may be reboiled via the reboiler loop (623). The source of heat may be a fired heater or hot stream. Note that the reboiler loop may not be required for all applications. Side reboilers or side coolers/condensers may also be added to the divided wall pretreatment device.

The cross-hatched areas represent mass transfer elements such as dense packed transition metal catalyst beds (with or without inert materials such as glass beads); loose catalyst supported on trays, or packing. The packing, if used, may be structured catalyst beds or random packing catalyst beds with inert materials mixed with the transition metal catalyst materials.

The partition may be made of any suitable material if there is substantially no mass transfer across the partition, however there may be some heat transfer across the partition. The column cross-sectional area need not be divided equally by the partition. The partition can have any suitable shape such as a vertical dividing plate or an internal cylindrical shell configuration. In the embodiment illustrated in FIG. 15 the partition is a vertical dividing plate bisecting the reactor, however, more than one plate may form radially arranged reactor sections.

The partially treated DFOM fluid from the lower portion of the first lower treatment section (604) is pumped through conduit means (624) into the second lower treatment section (606) at a point above the partitioned section. Top vapor from the second treatment section comprising gases and light and middle distillate hydrocarbons are withdrawn from the upper portion of the second lower treatment section (604). Middle distillate hydrocarbons are condensed in the upper portion of the treatment system (602) and removed via line (611) as medium and heavy distillate hydrocarbons (G) (i.e. diesel and gas oil) for use and processing outside the battery limits shown. A bottoms portion of the second lower treatment section, comprising Feedstock HMFO (A) may be routed through reboiler loop (625). The source of heat may be a fired heater or hot stream. Note that the reboiler loop is not required for all applications. Side reboilers or condensers may also be added to the divided wall pretreatment device. A second portion of the bottoms portion from the second lower treatment section (606) is removed through line (628) for use as Feedstock HMFO (A) in the Core Process. It may be desirable for there to be injection of make up or quenching Activating Gas in to the lower portions of the vessel. This may be achieved using Activating (or Stripping) Gas feedlines (630) and (632). One of skill in the art will appreciate that the properties of the DFOM sent to the first treatment section and the partially treated DFOM may be (but need not be) substantially the same (except for the levels of environmental contaminants such as sulfur).

At the design stage, different packing or combinations of trays, structured catalyst beds, and packing can be specified on each side of the partition to alter the fraction of the DFOM which flows on each side of the partition. Other

products such as middle and heavy distillate hydrocarbons may be taken from the upper portion of the treatment system 602 preferably from above the partitioned section.

In one embodiment the dividing partition is extended to the bottom of the part of the divided column containing trays or packing, and the section of trays or packing above the partition is eliminated. Such an arrangement allows easy control of the reflux liquid on each side of the divided column with a control valve (not shown) external to the column. In the embodiments illustrated in FIG. 15 flow through the lines are controlled in part by appropriate valving as is well known to those skilled in the art and these valves are not illustrated in the drawings.

One of skill in the art will appreciate the thermal benefits to be derived from the above illustrative embodiment. For example, one can utilize the above arrangement to more efficiently process relatively small volume (i.e. 500-5000 Bbl) of DFOM that a refinery would otherwise have to clear/dispose of. The divided wall reactor allows for a single treatment vessel to function as two separate vessels and take advantage of the combined collection of the by-product gases and light hydrocarbons.

In another illustrative embodiment of a divided wall Pre-Treatment Unit is shown in FIG. 16 in which the DFOM(P) is fed via line (610) to partition section (604) at a location below the top of the partition (608) and the treated DFOM exits from the lower portion of the first lower treatment section (604) as Feedstock HMFO (A) and is pumped through conduit means (623) to the Core Process as flow (A) shown in FIG. 2. Line (624), which corresponds to flow (B) in FIG. 2 receives the Product HMFO (B) from the Core Process into the second lower treatment section (606) at a point below the top of the partition (608). The return of the Product HMFO to the Divided wall Pre-Treatment Unit 35 will allow the recovery of any remaining distillate materials from the product HMFO either as distillate product via line (611) or to recycle the distillate material in the DFOM material being processed. It also takes advantage of the residual heat in the Product HMFO and may effectively transfer heat to the DFOM or reduce reboiler heat requirements. In this way the Pre-Treatment Unit can function as both a pre-Core Process treatment unit and a post-Core Process treatment unit.

By utilizing a divided wall Pre-Treatment Unit as illustrated in FIG. 16, light materials can be fractionated from the DFOM. Removal of light materials from the DFOM may adjust the flash point of the DFOM, bringing it into ISO 8217 compliance. H<sub>2</sub>S and water may also be removed from the feed by fractionating light components from the DFOM. Distillate range material from the product HMFO can also effectively be transferred to the DFOM by boiling the treated HMFO and refluxing liquid back to the column by utilizing a divided wall Pre-Treatment Unit. The transference of distillate range material from the product HMFO to the DFOM will address deficiencies such as pour point, density, viscosity, CCAI (calculated carbon aromaticity index) excessive metals content, high levels of nitrogen or high solids content.

Because of the nature of the divided wall Pre-Treatment Unit, a different temperature profile may be maintained below the partition (608) for the DFOM (P) contained in partition section (604) and the Product HMFO (B) contained in section (606). Cutpoints of the DFOM and HMFO can be controlled independently. A distillate side draw product 60 (611) may also be taken.

For the present disclosure, it one of skill in the art will appreciate that one or more of the above described pre-

treatment processes may need to be carried out to produce a Feedstock HMFO. The selection of the pre-treatment process will by necessity depend upon the nature and characteristics of the DFOM. For example if the DFOM is a high sulfur and high metals containing vacuum residual material (such as Ural vacuum residue or a heavy Mayan vacuum residue) the simple blending with heavy gas oil or FCC slurry oil may be sufficient to reduce the viscosity and sulfur and metals content so the DFOM is transformed into a Feedstock HMFO. However, pre-treatment of incompatible blends of Marine Gas Oil and high sulfur HMFO may require heating and distillation of the DFOM. A third example of DFOM requiring pre-treatment maybe the contamination of high sulfur HMFO with phenol or cumene and styrene oligomers which may required counter-current extraction with a polar liquid followed by heating and distillation removal of the non-residual volatiles boiling below 400° F. (205° C.). The specific pre-treatment process for any given DFOM will need to be adjusted and tested via an informed iterative process of optimization to produce a Feedstock HMFO for the Core Process.

These examples will provide one skilled in the art with a more specific illustrative embodiment for conducting the process disclosed and claimed herein:

#### EXAMPLE 1

##### Overview:

The purpose of a pilot test run is to demonstrate that feedstock HMFO can be processed through a reactor loaded with commercially available catalysts at specified conditions to remove environmental contaminates, specifically sulfur and other contaminates from the HMFO to produce a product HMFO that is MARPOL compliant, that is production of a Low Sulfur Heavy Marine Fuel Oil (LS—HMFO) or Ultra-Low Sulfur Heavy Marine Fuel Oil (ULS-HMFO).

##### Pilot Unit Set Up:

The pilot unit will be set up with two 434 cm<sup>3</sup> reactors arranged in series to process the feedstock HMFO. The lead reactor will be loaded with a blend of a commercially available hydrodemetalization (HDM) catalyst and a commercially available hydro-transition (HDT) catalyst. One of skill in the art will appreciate that the HDT catalyst layer may be formed and optimized using a mixture of HDM and HDS catalysts combined with an inert material to achieve the desired intermediate/transition activity levels. The second reactor will be loaded with a blend of the commercially available hydro-transition (HDT) and a commercially available hydrodesulfurization (HDS). One can load the second reactor simply with a commercially hydrodesulfurization (HDS) catalyst. One of skill in the art will appreciate that the specific feed properties of the Feedstock HMFO may affect the proportion of HDM, HDT and HDS catalysts in the reactor system. A systematic process of testing different combinations with the same feed will yield the optimized catalyst combination for any feedstock and reaction conditions. For this example, the first reactor will be loaded with 2/3 hydrodemetalization catalyst and 1/3 hydro-transition catalyst. The second reactor will be loaded with all hydrodesulfurization catalyst. The catalysts in each reactor will be mixed with glass beads (approximately 50% by volume) to improve liquid distribution and better control reactor temperature. For this pilot test run, one should use these commercially available catalysts: HDM: Albemarle KFR 20 series or equivalent; HDT: Albemarle KFR 30 series or equivalent; HDS: Albemarle KFR 50 or KFR 70 or equivalent. Once set up of the pilot unit is complete, the

catalyst can be activated by sulfiding the catalyst using dimethyldisulfide (DMDS) in a manner well known to one of skill in the art.

##### Pilot Unit Operation:

Upon completion of the activating step, the pilot unit will be ready to receive the feedstock HMFO and Activating Gas feed. For the present example, the Activating Gas can be technical grade or better hydrogen gas. The mixed Feedstock HMFO and Activating Gas will be provided to the pilot plant at rates and operating conditions as specified: Oil Feed Rate: 108.5 ml/h (space velocity=0.25/h); Hydrogen/Oil Ratio: 570 Nm<sup>3</sup>/m<sup>3</sup> (3200 scf/bbl); Reactor Temperature: 372° C. (702° F.); Reactor Outlet Pressure: 13.8 MPa(g) (2000 psig).

One of skill in the art will know that the rates and conditions may be systematically adjusted and optimized depending upon feed properties to achieve the desired product requirements. The unit will be brought to a steady state for each condition and full samples taken so analytical tests can be completed. Material balance for each condition should be closed before moving to the next condition.

Expected impacts on the Feedstock HMFO properties are: Sulfur Content (wt %): Reduced by at least 80%; Metals Content (wt %): Reduced by at least 80%; MCR/Asphaltene Content (wt %): Reduced by at least 30%; Nitrogen Content (wt %): Reduced by at least 20%; C<sub>1</sub>-Naphtha Yield (wt %): Not over 3.0% and preferably not over 1.0%.

Process conditions in the Pilot Unit can be systematically adjusted as per Table 1 to assess the impact of process conditions and optimize the performance of the process for the specific catalyst and feedstock HMFO utilized.

TABLE 1

| Case     | Optimization of Process Conditions    |                                                                                    |                     |                           |
|----------|---------------------------------------|------------------------------------------------------------------------------------|---------------------|---------------------------|
|          | HC Feed Rate<br>(ml/h),<br>[LHSV/(h)] | Nm <sup>3</sup> H <sub>2</sub> /m <sup>3</sup> oil/<br>scf H <sub>2</sub> /bbl oil | Temp<br>(° C./° F.) | Pressure<br>(MPa(g)/psig) |
| Baseline | 108.5 [0.25]                          | 570/3200                                                                           | 372/702             | 13.8/2000                 |
| T1       | 108.5 [0.25]                          | 570/3200                                                                           | 362/684             | 13.8/2000                 |
| T2       | 108.5 [0.25]                          | 570/3200                                                                           | 382/720             | 13.8/2000                 |
| L1       | 130.2 [0.30]                          | 570/3200                                                                           | 372/702             | 13.8/2000                 |
| L2       | 86.8 [0.20]                           | 570/3200                                                                           | 372/702             | 13.8/2000                 |
| H1       | 108.5 [0.25]                          | 500/2810                                                                           | 372/702             | 13.8/2000                 |
| H2       | 108.5 [0.25]                          | 640/3590                                                                           | 372/702             | 13.8/2000                 |
| S1       | 65.1 [0.15]                           | 620/3480                                                                           | 385/725             | 15.2/2200                 |

In this way, the conditions of the pilot unit can be optimized to achieve less than 0.5% wt. sulfur product HMFO and preferably a 0.1% wt. sulfur product HMFO. Conditions for producing ULS-HMFO (i.e. 0.1% wt. sulfur product HMFO) will be: Feedstock HMFO Feed Rate: 65.1 ml/h (space velocity=0.15/h); Hydrogen/Oil Ratio: 620 Nm<sup>3</sup>/m<sup>3</sup> (3480 scf/bbl); Reactor Temperature: 385° C. (725° F.); Reactor Outlet Pressure: 15 MPa(g) (2200 psig)

Table 2 summarizes the anticipated impacts on key properties of HMFO.

TABLE 2

| Property                  | Minimum | Typical | Maximum |
|---------------------------|---------|---------|---------|
| Sulfur Conversion/Removal | 80%     | 90%     | 98%     |
| Metals Conversion/Removal | 80%     | 90%     | 100%    |
| MCR Reduction             | 30%     | 50%     | 70%     |
| Asphaltene Reduction      | 30%     | 50%     | 70%     |
| Nitrogen Conversion       | 10%     | 30%     | 70%     |

TABLE 2-continued

| Property                       | Minimum | Typical | Maximum |
|--------------------------------|---------|---------|---------|
| C1 through Naphtha Yield       | 0.5%    | 1.0%    | 4.0%    |
| Hydrogen Consumption (scf/bbl) | 500     | 750     | 1500    |

Table 3 lists analytical tests to be carried out for the characterization of the Feedstock HMFO and Product HMFO. The analytical tests include those required by ISO for the Feedstock HMFO and the product HMFO to qualify and trade in commerce as ISO compliant residual marine fuels. The additional parameters are provided so that one skilled in the art can understand and appreciate the effectiveness of the inventive process.

TABLE 3

| Analytical Tests and Testing Procedures |                                               |
|-----------------------------------------|-----------------------------------------------|
| Sulfur Content                          | ISO 8754 or ISO 14596 or ASTM D4294           |
| Density @ 15° C.                        | ISO 3675 or ISO 12185                         |
| Kinematic                               | ISO 3104                                      |
| Viscosity @ 50° C.                      |                                               |
| Pour Point, ° C.                        | ISO 3016                                      |
| Flash Point, ° C.                       | ISO 2719                                      |
| CCAI                                    | ISO 8217, ANNEX B                             |
| Ash Content                             | ISO 6245                                      |
| Total Sediment - Aged                   | ISO 10307-2                                   |
| Micro Carbon Residue, mass %            | ISO 10370                                     |
| H2S, mg/kg                              | IP 570                                        |
| Acid Number                             | ASTM D664                                     |
| Water                                   | ISO 3733                                      |
| Specific Contaminants                   | IP 501 or IP 470 (unless indicated otherwise) |
| Vanadium                                | or ISO 14597                                  |
| Sodium                                  |                                               |
| Aluminum                                | or ISO 10478                                  |
| Silicon                                 | or ISO 10478                                  |
| Calcium                                 | or IP 500                                     |
| Zinc                                    | or IP 500                                     |
| Phosphorous                             | IP 500                                        |
| Nickle                                  |                                               |
| Iron                                    |                                               |
| Distillation                            | ASTM D7169                                    |
| C:H Ratio                               | ASTM D3178                                    |
| SARA Analysis                           | ASTM D2007                                    |
| Asphaltenes, wt %                       | ASTM D6560                                    |
| Total Nitrogen                          | ASTM D5762                                    |
| Vent Gas Component Analysis             | FID Gas Chromatography or comparable          |

Table 4 contains the Feedstock HMFO analytical test results and the Product HMFO analytical test results expected from the inventive process that indicate the production of a LS HMFO. It will be noted by one of skill in the art that under the conditions, the levels of hydrocarbon cracking will be minimized to levels substantially lower than 10%, more preferably less than 5% and even more preferably less than 1% of the total mass balance.

TABLE 4

| Analytical Results                               |                |                    |
|--------------------------------------------------|----------------|--------------------|
|                                                  | Feedstock HMFO | Product HMFO       |
| Sulfur Content, mass %                           | 3.0            | 0.3                |
| Density @ 15° C., kg/m <sup>3</sup>              | 990            | 950 <sup>(1)</sup> |
| Kinematic Viscosity @ 50° C., mm <sup>2</sup> /s | 380            | 100 <sup>(1)</sup> |
| Pour Point, ° C.                                 | 20             | 10                 |
| Flash Point, ° C.                                | 110            | 100 <sup>(1)</sup> |

TABLE 4-continued

| Analytical Results           |                |              |
|------------------------------|----------------|--------------|
|                              | Feedstock HMFO | Product HMFO |
| 5 CCAI                       | 850            | 820          |
| Ash Content, mass %          | 0.1            | 0.0          |
| Total Sediment—Aged, mass %  | 0.1            | 0.0          |
| Micro Carbon Residue, mass % | 13.0           | 6.5          |
| H2S, mg/kg                   | 0              | 0            |
| 10 Acid Number, mg KO/g      | 1              | 0.5          |
| Water, vol %                 | 0.5            | 0            |
| Specific Contaminants, mg/kg |                |              |
| 15 Vanadium                  | 180            | 20           |
| Sodium                       | 30             | 1            |
| Aluminum                     | 10             | 1            |
| Silicon                      | 30             | 3            |
| Calcium                      | 15             | 1            |
| Zinc                         | 7              | 1            |
| Phosphorous                  | 2              | 0            |
| Nickle                       | 40             | 5            |
| Iron                         | 20             | 2            |
| 20 Distillation, ° C./° F.   |                |              |
| IBP                          | 160/320        | 120/248      |
| 5% wt                        | 235/455        | 225/437      |
| 10% wt                       | 290/554        | 270/518      |
| 30% wt                       | 410/770        | 370/698      |
| 25 50% wt                    | 540/1004       | 470/878      |
| 70% wt                       | 650/1202       | 580/1076     |
| 90% wt                       | 735/1355       | 660/1220     |
| FBP                          | 820/1508       | 730/1346     |
| C:H Ratio (ASTM D3178)       | 1.2            | 1.3          |
| 30 SARA Analysis             |                |              |
| Saturates                    | 16             | 22           |
| Aromatics                    | 50             | 50           |
| Resins                       | 28             | 25           |
| Asphaltenes                  | 6              | 3            |
| Asphaltenes, wt %            | 6.0            | 2.5          |
| 35 Total Nitrogen, mg/kg     | 4000           | 3000         |

Note:

<sup>(1)</sup>property will be adjusted to a higher value by post process removal of light material via distillation or stripping from product HMFO.

40 The product HMFO produced by the inventive process will reach ULS HMFO limits (i.e. 0.1% wt. sulfur product HMFO) by systematic variation of the process parameters, for example by a lower space velocity or by using a Feedstock HMFO with a lower initial sulfur content.

#### 45 EXAMPLE 2: RMG-380 HMFO

##### Pilot Unit Set Up:

50 A pilot unit was set up as noted above in Example 1 with these changes: the first reactor was loaded with: as the first (upper) layer encountered by the feedstock 70% vol Albemarle KFR 20 series hydrodemetallization catalyst and 30% vol Albemarle KFR 30 series hydro-transition catalyst as the second (lower) layer. The second reactor was loaded with 20% Albemarle KFR 30 series hydrotransition catalyst as 55 the first (upper) layer and 80% vol hydrodesulfurization catalyst as the second (lower) layer. The catalyst was activated by sulfiding the catalyst with dimethyldisulfide (DMDS) in a manner well known to one of skill in the art.

##### Pilot Unit Operation:

60 Upon completion of the activating step, the pilot unit was ready to receive the feedstock HMFO and Activating Gas feed. The Activating Gas was technical grade or better hydrogen gas. The Feedstock HMFO was a commercially available and merchantable ISO 8217 compliant HMFO, 65 except for a high sulfur content (2.9 wt %). The mixed Feedstock HMFO and Activating Gas was provided to the pilot plant at rates and conditions as specified in Table 5

below. The conditions were varied to optimize the level of sulfur in the product HMFO material.

TABLE 5

| Case     | Process Conditions                   |                                                                                    |                         |                               |                                    |
|----------|--------------------------------------|------------------------------------------------------------------------------------|-------------------------|-------------------------------|------------------------------------|
|          | HC Feed<br>Rate (ml/h),<br>[LHSV(h)] | Nm <sup>3</sup> H <sub>2</sub> /m <sup>3</sup> oil/<br>scf H <sub>2</sub> /bbl oil | Temp<br>(° C./<br>° F.) | Pressure<br>(MPa(g)/<br>psig) | Product<br>HMFO<br>Sulfur<br>% wt. |
| Baseline | 108.5 [0.25]                         | 570/3200                                                                           | 371/700                 | 13.8/2000                     | 0.24                               |
| T1       | 108.5 [0.25]                         | 570/3200                                                                           | 362/684                 | 13.8/2000                     | 0.53                               |
| T2       | 108.5 [0.25]                         | 570/3200                                                                           | 382/720                 | 13.8/2000                     | 0.15                               |
| L1       | 130.2 [0.30]                         | 570/3200                                                                           | 372/702                 | 13.8/2000                     | 0.53                               |
| S1       | 65.1 [0.15]                          | 620/3480                                                                           | 385/725                 | 15.2/2200                     | 0.10                               |
| P1       | 108.5 [0.25]                         | 570/3200                                                                           | 371/700                 | /1700                         | 0.56                               |
| T2/P1    | 108.5 [0.25]                         | 570/3200                                                                           | 382/720                 | /1700                         | 0.46                               |

Analytical data for a representative sample of the feedstock HMFO and representative samples of product HMFO are below:

TABLE 6

| Analytical Results - HMFO (RMG-380)              |            |          |          |
|--------------------------------------------------|------------|----------|----------|
|                                                  | Feedstock  | Product  | Product  |
| Sulfur Content, mass %                           | 2.9        | 0.3      | 0.1      |
| Density @ 15° C., kg/m <sup>3</sup>              | 988        | 932      | 927      |
| Kinematic Viscosity @ 50° C., mm <sup>2</sup> /s | 382        | 74       | 47       |
| Pour Point, ° C.                                 | -3         | -12      | -30      |
| Flash Point, ° C.                                | 116        | 96       | 90       |
| CCAI                                             | 850        | 812      | 814      |
| Ash Content, mass %                              | 0.05       | 0.0      | 0.0      |
| Total Sediment - Aged, mass %                    | 0.04       | 0.0      | 0.0      |
| Micro Carbon Residue, mass %                     | 11.5       | 3.3      | 4.1      |
| H2S, mg/kg                                       | 0.6        | 0        | 0        |
| Acid Number, mg KO/g                             | 0.3        | 0.1      | >0.05    |
| Water, vol %                                     | 0          | 0.0      | 0.0      |
| Specific Contaminants, mg/kg                     |            |          |          |
| Vanadium                                         | 138        | 15       | <1       |
| Sodium                                           | 25         | 5        | 2        |
| Aluminum                                         | 21         | 2        | <1       |
| Silicon                                          | 16         | 3        | 1        |
| Calcium                                          | 6          | 2        | <1       |
| Zinc                                             | 5          | <1       | <1       |
| Phosphorous                                      | <1         | 2        | 1        |
| Nickle                                           | 33         | 23       | 2        |
| Iron                                             | 24         | 8        | 1        |
| Distillation, ° C./° F.                          |            |          |          |
| IBP                                              | 178/352    | 168/334  | 161/322  |
| 5% wt                                            | 258/496    | 235/455  | 230/446  |
| 10% wt                                           | 298/569    | 270/518  | 264/507  |
| 30% wt                                           | 395/743    | 360/680  | 351/664  |
| 50% wt                                           | 517/962    | 461/862  | 439/822  |
| 70% wt                                           | 633/1172   | 572/1062 | 552/1026 |
| 90% wt                                           | >720/>1328 | 694/1281 | 679/1254 |
| FBP                                              | >720/>1328 | >720/    | >720/    |
|                                                  |            | >1328    | >1328    |
| C:H Ratio (ASTM D3178)                           | 1.2        | 1.3      | 1.3      |
| SARA Analysis                                    |            |          |          |
| Saturates                                        | 25.2       | 28.4     | 29.4     |
| Aromatics                                        | 50.2       | 61.0     | 62.7     |
| Resins                                           | 18.6       | 6.0      | 5.8      |
| Asphaltenes                                      | 6.0        | 4.6      | 2.1      |
| Asphaltenes, wt %                                | 6.0        | 4.6      | 2.1      |
| Total Nitrogen, mg/kg                            | 3300       | 1700     | 1600     |

In Table 6, both feedstock HMFO and product HMFO exhibited observed bulk properties consistent with ISO 8217 for a merchantable residual marine fuel oil, except that the

sulfur content of the product HMFO was reduced as noted above when compared to the feedstock HMFO.

One of skill in the art will appreciate that the above product HMFO produced by the inventive process has achieved not only an ISO 8217 compliant LS HMFO (i.e. 0.5% wt. sulfur) but also an ISO 8217 compliant ULS HMFO limits (i.e. 0.1% wt. sulfur) product HMFO.

#### EXAMPLE 3: RMK-500 HMFO

The feedstock to the pilot reactor utilized in example 2 above was changed to a commercially available and merchantable ISO 8217 RMK-500 compliant HMFO, except that it has high environmental contaminates (i.e. sulfur (3.3 wt %)). Other bulk characteristic of the RMK-500 feedstock high sulfur HMFO are provide below:

TABLE 7

| Analytical Results - Feedstock HMFO (RMK-500)    |      |  |
|--------------------------------------------------|------|--|
| Sulfur Content, mass %                           | 3.3  |  |
| Density @ 15° C., kg/m <sup>3</sup>              | 1006 |  |
| Kinematic Viscosity @ 50° C., mm <sup>2</sup> /s | 500  |  |

The mixed Feedstock (RMK-500) HMFO and Activating Gas was provided to the pilot plant at rates and conditions and the resulting sulfur levels achieved in the table below

TABLE 8

| Case | Process Conditions                      |                                                                                       |                         |                               |                                      |
|------|-----------------------------------------|---------------------------------------------------------------------------------------|-------------------------|-------------------------------|--------------------------------------|
|      | HC Feed<br>Rate<br>(ml/h),<br>[LHSV(h)] | Nm <sup>3</sup> H <sub>2</sub> /m <sup>3</sup> oil/<br>scf H <sub>2</sub> /bbl<br>oil | Temp<br>(° C./<br>° F.) | Pressure<br>(MPa(g)/<br>psig) | Product<br>sulfur % wt.<br>(RMK-500) |
| A    | 108.5 [0.25]                            | 640/3600                                                                              | 377/710                 | 13.8/2000                     | 0.57                                 |
| B    | 95.5 [0.22]                             | 640/3600                                                                              | 390/735                 | 13.8/2000                     | 0.41                                 |
| C    | 95.5 [0.22]                             | 640/3600                                                                              | 390/735                 | 11.7/1700                     | 0.44                                 |
| D    | 95.5 [0.22]                             | 640/3600                                                                              | 393/740                 | 10.3/1500                     | 0.61                                 |
| E    | 95.5 [0.22]                             | 640/3600                                                                              | 393/740                 | 17.2/2500                     | 0.37                                 |
| F    | 95.5 [0.22]                             | 640/3600                                                                              | 393/740                 | 8.3/1200                      | 0.70                                 |
| G    | 95.5 [0.22]                             | 640/3600                                                                              | 416/780                 | 8.3/1200                      |                                      |

The resulting product (RMK-500) HMFO exhibited observed bulk properties consistent with the feedstock (RMK-500) HMFO, except that the sulfur content was reduced as noted in the above table.

One of skill in the art will appreciate that the above product HMFO produced by the inventive process has achieved a LS HMFO (i.e. 0.5% wt. sulfur) product HMFO having bulk characteristics of an ISO 8217 compliant RMK-500 residual fuel oil. It will also be appreciated that the process can be successfully carried out under non-hydrocracking conditions (i.e. lower temperature and pressure) that substantially reduce the hydrocracking of the feedstock material. When conditions were increased to much higher pressure (Example E) a product with a lower sulfur content was achieved, however some observed there was an increase in light hydrocarbons and wild naphtha production.

It will be appreciated by those skilled in the art that changes could be made to the illustrative embodiments described above without departing from the broad inventive concepts thereof. It is understood, therefore, that the inventive concepts disclosed are not limited to the illustrative embodiments or examples disclosed, but it should cover modifications within the scope of the inventive concepts as defined by the claims.

The invention claimed is:

1. A process for production of a Product Heavy Marine Fuel Oil from Distressed Fuel Oil Materials, the process comprising: processing the Distressed Fuel Oil Materials in a pre-treatment unit under operative conditions to give a pre-treated Feedstock Heavy Marine Fuel Oil, wherein the pre-treated Feedstock Heavy Marine Fuel Oil complies with ISO 8217 except for the environmental contaminates including a sulfur content (ISO 14596 or ISO 8754) between the range of 5.0 wt % to 0.50 wt %; mixing a quantity of the pre-treated Feedstock Heavy Marine Fuel Oil with a quantity of Activating Gas mixture to give a Feedstock Mixture; contacting the Feedstock Mixture with one or more transition metal catalysts under reactive conditions to form a Process Mixture from said Feedstock Mixture; receiving said Process Mixture and separating the Product Heavy Marine Fuel Oil liquid components of the Process Mixture from the gaseous components and by-product hydrocarbon components of the Process Mixture and, discharging the Product Heavy Marine Fuel Oil.

2. The process of claim 1 wherein the Product Heavy Marine Fuel Oil complies with ISO 8217:2017 and has a sulfur content (ISO 14596 or ISO 8754) between the range of 0.05 wt % to 0.50 wt %.

3. The process of claim 1, wherein said Product Heavy Marine Fuel Oil has bulk properties of: a kinematic viscosity at 50° C. (ISO 3104) between the range from 180 mm<sup>2</sup>/s to 700 mm<sup>2</sup>/s; a density at 15° C. (ISO 3675) between the range of 991.0 kg/m<sup>3</sup> to 1010.0 kg/m<sup>3</sup>; a CCAI is in the range of 780 to 870; a flash point (ISO 2719) no lower than 60° C.; a total sediment—aged (ISO 10307-2) less, than 0.10 mass %; and a carbon residue—micro method (ISO 10.170) less than 20.00 mass %.

4. The process of claim 1, wherein the transition metal catalyst comprises: a porous inorganic oxide catalyst carrier and a transition metal catalyst, wherein the porous inorganic oxide catalyst carrier is at least one carrier selected from the group consisting of alumina, alumina/boria carrier, a carrier containing metal-containing aluminosilicate, alumina/phosphorus carrier, alumina/alkaline earth metal compound carrier, alumina/Titania carrier and alumina/zirconia carrier, and wherein the transition metal catalyst is one or more metals selected from the group consisting of group 6, 8, 9 and 10 of the Periodic Table and wherein the hydrogen has an ideal gas, partial pressure of hydrogen (p<sub>H2</sub>) greater than 80% of the total pressure of the gas mixture (P).

5. The process of claim 4, wherein the reactive conditions comprise: the ratio of the quantity of the Activating Gas mixture to the quantity of Feedstock Heavy Marine Fuel Oil is in the range of 250 scf gas/bbl of Feedstock Heavy Marine Fuel Oil to 10,000 scf gas/bbl of Feedstock Heavy Marine Fuel Oil; a the total pressure is between of 250 psig and 3000 psig; and, the indicated temperature is between of 500° F. to 900° F., and, wherein the liquid hourly space velocity is between 0.05 oil/hour/m<sup>3</sup> catalyst and 1.0 oil/hour/m<sup>3</sup> catalyst.

6. The process of claim 1, wherein the pre-treatment unit is selected from the group consisting of a distillation column, steam stripper column, and a reactive distillation column, wherein the operative conditions of the pre-treatment unit are selected so that non-residual volatile components of the Distressed Fuel Oil Materials, wherein the non-residual volatile components have a boiling temperature of less than 400° F. (205° C.), are removed via distillation from the Distressed Fuel Oil Materials to produce a distillate

stream having a boiling temperature of less than 400° F. (205° C.) and the pre-treated Feedstock Heavy Marine Fuel Oil stream.

7. The process of claim 1 wherein the pre-treatment unit is a divided wall distillation column, wherein non-residual volatile components of the Distressed Fuel Oil Materials, wherein the non-residual volatile components have a boiling temperature of less than 400° F. (205° C.) are removed via distillation from the residual components of the Distressed Fuel Oil Materials to produce a distillate stream having a boiling temperature of less than 400° F. (205° C.) and, the pre-treated Feedstock Heavy Marine Fuel Oil stream.

8. The process of claim 7, wherein the divided wall distillation column further comprises one or more structured beds, wherein the one or more structured beds comprises a plurality of catalyst retention structures, each catalyst retentions structure comprising at least two coplanar fluid permeable metal sheets, wherein at least one of the fluid permeable sheets is corrugated and wherein the two coplanar fluid permeable metal sheets define one or more catalyst rich spaces and one or more catalyst lean spaces, wherein within the catalyst rich space there is one or more catalyst materials, and optionally inert packing materials and wherein the catalyst lean spaces optionally contain an inert packing material.

9. The process of claim 6 wherein the pre-treatment unit is a reactive distillation column, wherein the reactive distillation column comprises one or more structured beds, wherein the one or more structured beds comprises a plurality of catalyst retention structures, each catalyst retentions structure comprising at least two coplanar fluid permeable metal sheets, wherein at least one of the fluid permeable sheets is corrugated and wherein the two coplanar fluid permeable metal sheets define one or more catalyst rich spaces and one or more catalyst lean spaces, wherein within the catalyst rich space there is one or more catalyst materials and optionally inert packing materials and wherein the catalyst lean spaces optionally contain an inert packing material and wherein non-residual volatile components of the Distressed Fuel Oil Materials having a boiling temperature of less than 400 (205° C.) are removed via reactive distillation from the residual components of the Distressed Fuel Oil Materials having a boiling temperature of less than 400° F. (205° C.) to produce a distillate stream and a pre-treated Feedstock Heavy Marine Fuel Oil stream.

10. A process for production of a Product Heavy Marine Fuel Oil from Distressed Fuel Oil Materials, the process comprising: selecting a Distressed Fuel Oil Material selected from the group consisting of: atmospheric residue; vacuum residue; FCC slurry, oil; black oil; FCC cycle oil; vacuum gas oil; gas oil; distillates; coker gas oil; de-asphalted heavy oil; synthetic oils; visbreaker residue; crude oils such as heavy crude oil; distressed crude oil; residual marine fuel or distillate and residual blends that have a 4 or 5 rating on ASTM D4740 compatibility tests and combinations thereof; processing the Distressed Fuel Oil Materials in a pre-treatment unit under operative conditions to give a m-treated Feedstock Heavy Marine Fuel Oil, wherein the pre-treated Feedstock Heavy Marine Fuel Oil complies with ISO 8247 except for the environmental contaminates, wherein the environmental contaminates are selected from the group consisting of: sulfur (ISO 14596 or ISO 8754); aluminum (ISO 10478); silicon (ISO 10478); nitrogen (ASTM D5762); vanadium content (ISO 14597), iron, nickel, calcium (IP 500), phosphorous (IP 500), and combinations thereof; and wherein the environmental contaminates have a cumulative concentration between the range of 5.0 wt % to 0.50 wt %;

mixing a quantity of the pre-treated Feedstock Heavy Marine Fuel Oil with a quantity of an Activating Gas mixture to give a Feedstock Mixture, wherein the Activating Gas mixture is selected from the groups consisting of: nitrogen, hydrogen, carbon dioxide, gaseous water, methane and mixtures thereof, and wherein the Activating Gas Mixture has an ideal gas partial pressure of hydrogen ( $p_{H_2}$ ) greater than 80% of the total pressure of the Activating Gas mixture (P); contacting the Feedstock Mixture with one or more transition metal catalysts under reactive conditions to form a Process Mixture from said Feedstock Mixture, wherein the Process Mixture comprises a mixture of gaseous components, by-product hydrocarbon components and a Product Heavy Marine Fuel Oil liquid component; receiving said Process Mixture in one or more separation vessels and separating the Product Heavy Marine Fuel Oil liquid component of the Process Mixture from the gaseous components and by-product hydrocarbon components of the Process Mixture and, discharging the Product Heavy Marine Fuel Oil liquid component.

11. The process of claim 10 wherein the Product Heavy Marine Fuel Oil complies with ISO 8217:2017 and has a sulfur content (ISO 14596 or ISO 8754) between the range of 0.05 wt % to 0.50 wt %.

12. The process of claim 10, wherein said Product Heavy Marine Fuel Oil has bulk properties of: a kinematic viscosity at 50° C. (ISO 3104) between the range from 180 mm<sup>2</sup>/s to 700 mm<sup>2</sup>/s; a density at 15° C. (ISO 3675) between the range of 991.0 kg/m<sup>3</sup> to 1010.0 kg/m<sup>3</sup>; a CCAI is in the range of 780 to 870; a flash point (ISO 2719) no lower than 60° C.; a total sediment—aged (ISO 10307-2) less than 0.10 mass and a carbon residue—micro method (ISO 10370) less than 20.00 mass %.

13. The process of claim 10, wherein the transition metal catalyst comprises: a porous inorganic oxide catalyst carrier and a transition metal catalyst, wherein the porous inorganic oxide catalyst carrier is at least one carrier selected from the group consisting of alumina, alumina/aria carrier, a carrier containing metal-containing aluminosilicate, alumina/phosphorus carrier, alumina/alkaline earth metal compound carrier, alumina/titania carrier and alumina/zirconia carrier, and wherein the transition metal catalyst is one or more metals selected from the group consisting of group 6, 8, 9 and 10 of the Periodic Table.

14. A process for production of a Product Heavy Marine Fuel Oil from Distressed Fuel Oil Materials, the process comprising: selecting a Distressed Fuel Oil Material selected from the group consisting of: atmospheric residue; vacuum residue; FCC slurry oil; black oil; FCC cycle oil; vacuum gas oil; gas oil; distillates; coker gas oil; de-asphalted heavy oil; synthetic oils; visbreaker residue; crude oils such as heavy crude oil; distressed crude oil; residual marine fuel or distillate and residual blends that have a 4 or 5 rating on ASTM 04740 compatibility tests and combinations thereof; processing the Distressed Fuel Oil Materials in a pre-treatment unit under operative conditions to give a pre-treated Feedstock Heavy Marine Fuel Oil, wherein the pre-treated Feedstock Heavy Marine Fuel Oil complies with ISO 8217 except for the sulfur (ISO 14596 or ISO 8754) content; wherein the sulfur content has a concentration between the range of 5.0 wt % to 0.50 wt %; mixing a quantity of the pre-treated Feedstock Heavy Marine Fuel Oil with a quantity of an Activating Gas mixture to give a Feedstock Mixture, wherein the Activating Gas, wherein the Activating Gas Mixture has an ideal gas partial pressure of hydrogen ( $p_{H_2}$ ) greater than 80% of the total pressure of the Activating Gas mixture (P); contacting the Feedstock Mix-

ture with one or more transition metal catalysts under reactive conditions to form a Process Mixture from said Feedstock Mixture, wherein said Process Mixture is a combination of heavy hydrocarbon, liquid components, condensable and non-condensable by-product hydrocarbon components, bulk gaseous components, and residual gaseous components; passing to and receiving said Process Mixture in a first separation vessel and separating and separating a mixture of the heavy hydrocarbon liquid components, the condensable by-product hydrocarbon components and the residual gaseous components of the Process Mixture from the non-condensable by-product hydrocarbon components and the hulk gaseous components of the Process Mixture, and discharging the mixture of heavy hydrocarbon liquid components, the condensable by-product hydrocarbon components and residual gaseous components of the Process Mixture from the first separating vessel via fluid communication to said second separating vessel; separating in the second separation vessel the residual gaseous components and condensable by-product hydrocarbon components from the heavy hydrocarbon liquid components of the Process Mixture, and discharging the heavy hydrocarbon liquid components from the second separating vessel forming the Product Heavy Marine Fuel Oil.

15. The process of claim 14 wherein the Product Heavy Marine Fuel Oil complies with ISO 8217:2017 and has a sulfur content (ISO 14596 or ISO 8754) between the range of 0.05 wt % to 0.50 wt %.

16. The process of claim 14, wherein said Product Heavy Marine Fuel Oil has bulk properties of: a kinematic viscosity at 50° C. (ISO 3104) between the range from 180 mm<sup>2</sup>/s to 700 mm<sup>2</sup>/s; a density at 15° C. (ISO 3675) between the range of 991.0 kg/m<sup>3</sup> to 1010.0 kg/m<sup>3</sup>; a CCAI is in the range of 780 to 870; a flash point (ISO 2719) no lower than 60° C.; a total sediment—aged (ISO 10307-2) less than 0.10 mass %; and a carbon residue—micro method (ISO 10370) less than 20.00 mass %.

17. The process of claim 14, wherein the transition metal catalyst comprises: a porous inorganic oxide catalyst carrier and a transition metal catalyst, wherein the porous inorganic oxide catalyst carrier is at least one carrier selected from the group consisting of alumina, alumina/boria carrier, a carrier containing metal-containing aluminosilicate, alumina/phosphorus carrier, alumina/alkaline earth metal compound carrier, alumina/titania carrier and alumina/zirconia carrier, and wherein the transition metal catalyst is one or more metals selected from the group consisting of group 6, 8, 9 and 10 of the Periodic Table.

18. The process of claim 14 wherein the pre-treatment unit is a reactive distillation column, wherein the reactive distillation column comprises one or more structured beds, wherein the one or more structured beds comprises a plurality of catalyst retention structures, each catalyst retentions structure comprising at least two coplanar fluid permeable metal sheets, wherein at least one of the fluid permeable sheets is corrugated and wherein the two coplanar fluid permeable metal sheets define one or more catalyst rich spaces and one or more catalyst lean spaces, wherein within the catalyst rich space there is one or more catalyst materials, wherein the catalyst materials are selected from the group consisting of hydrodemetallization catalyst, hydrotransition catalyst, hydrodesulfurization catalyst, and combinations thereof, and optionally inert packing materials and wherein the catalyst lean spaces optionally contain an inert packing material and wherein non-residual volatile components of the Distressed Fuel Oil Materials, having a boiling temperature of less than 400° F. (205° C.) are

removed via reactive distillation from the residual components of the Distressed Fuel Oil Materials having a boiling temperature of less than 400° F. (205° C.) to produce a distillate stream having a boiling temperature of less than 400° F. (205° C.) and a pre-treated Feedstock Heavy Marine 5 Fuel Oil stream.

19. The process of claim 14 wherein the pre-treatment unit is a distillation column, wherein non-residual volatile components of the Distressed Fuel Oil Materials, wherein the non-residual volatile components have a boiling temperature of less than 400° F. (205° C.) are removed via distillation from the residual components of the Distressed Fuel Oil Materials to produce a distillate stream having a boiling temperature of less than 400° F. (205° C.) and the pre-treated Feedstock Heavy Marine Fuel Oil stream. 15

\* \* \* \* \*